# EUROPEAN PATENT APPLICATION

(11) **EP 4 190 581 A1**
(43) Date of publication of application: **07.06.2023**
(21) Application number: 21848782.5
(22) Date of filing: 27.07.2021
(51) Int. Cl.: B41N 1/14, B41C 1/10, B41M 1/06, G03F 7/00, G03F 7/11, G03F 7/20

(54) **ON-PRESS-DEVELOPMENT-TYPE PLANOGRAPHIC PRINTING ORIGINAL PLATE, METHOD FOR PRODUCING PLANOGRAPHIC PRINTING PLATE, AND PLANOGRAPHIC PRINTING METHOD**

(30) Priority: 31.07.2020 JP 2020130529
(71) Applicant: FUJIFILM Corporation, Tokyo 106-8620 (JP)
(72) Inventor: KOYAMA, Ichiro, Haibara-gun, Shizuoka 421-0396 (JP); YANAGI, Shunsuke, Haibara-gun, Shizuoka 421-0396 (JP); ENOMOTO, Kazuaki, Haibara-gun, Shizuoka 421-0396 (JP); KUDO, Kotaro, Haibara-gun, Shizuoka 421-0396 (JP)
(74) Representative: HGF
(86) International application number: PCT/JP2021/027775
(87) International publication number: WO 2022/025068

(57) **Abstract**

Provided is an on-press development type lithographic printing plate precursor having a support, an image-recording layer, and an outermost layer in this order, in which the outermost layer has a sea-island structure consisting of a discontinuous phase that contains a hydrophobic polymer and a continuous phase that contains a water-soluble polymer. Also provided are a method of preparing a lithographic printing plate and a lithographic printing method in which the on-press development type lithographic printing plate precursor is used.

## Description

### BACKGROUND OF THE INVENTION

### 1. Field of the Invention

The present disclosure relates to an on-press development type lithographic printing plate precursor, a method of preparing a lithographic printing plate, and a lithographic printing method.

### 2. Description of the Related Art

Generally, a lithographic printing plate consists of a lipophilic image area that receives ink in a printing process and a hydrophilic non-image area that receives dampening water. Lithographic printing is a method exploiting the mutual repulsion of water and oil-based ink, in which the lipophilic image area and the hydrophilic non-image area of a lithographic printing plate are used as an ink-receiving portion and a dampening water-receiving portion (non-ink-receiving portion) respectively, the adhesiveness of ink is varied within the surface of the lithographic printing plate such that only the image area receives the ink, and then printing is performed by the transfer of the ink to a printing substrate such as paper.

In the related art, in order to prepare this lithographic printing plate, a lithographic printing plate precursor (PS plate) has been widely used which is obtained by providing a lipophilic photosensitive resin layer (image-recording layer) on a hydrophilic support. Generally, a lithographic printing plate is obtained by a plate making method of exposing a lithographic printing plate precursor through an original picture such as a lith film, then keeping a portion of an image-recording layer that will be an image area while removing other unnecessary portions of the image-recording layer by dissolving such portions in an alkaline developer or an organic solvent, and forming a non-image area by exposing the hydrophilic surface of a support.

In response to the intensifying interest in the global environment, an environmental issue of waste liquid generated by wet treatments such as a development treatment has gathered more attention.

Regarding the environmental issue described above, an attempt is made to simplify development or plate making or to remove treatments. As one of simple preparation methods, a method called "on-press development" is being carried out. That is, on-press development is a method of exposing a lithographic printing plate precursor, then immediately mounting the precursor on a printer without performing development of the related art, and removing an unnecessary portion of the image-recording layer at an early stage of the ordinary printing step.

In the present disclosure, a lithographic printing plate precursor that can be used for such on-press development is called "on-press development type lithographic printing plate precursor"

Examples of the lithographic printing plate precursors in the related art include those described in JP2006-264300A or WO2019/243036A.

JP2006-264300A describes a lithographic printing plate precursor having an image-recording layer and an overcoat layer in this order on a support, in which an image can be formed on the image-recording layer by supplying an oil-based ink and an aqueous component to the image-recording layer on a printer and removing a non-exposed portion, and heat-fusible fine particles are dispersed in the overcoat layer.

Furthermore, WO2019/243036A describes a negative tone lithographic printing plate precursor having a top layer.

### SUMMARY OF THE INVENTION

An object of an embodiment of the present disclosure is to provide an on-press development type lithographic printing plate precursor excellent in receptivity and on-press development residue suppressiveness.

An object of another embodiment of the present disclosure is to provide a method of preparing a lithographic printing plate and a lithographic printing method in which the on-press development type lithographic printing plate precursor is used.

Means for achieving the above objects include the following aspects.
<1> An on-press development type lithographic printing plate precursor having a support, an image-recording layer, and an outermost layer in this order, in which the outermost layer has a sea-island structure consisting of a discontinuous phase that contains a hydrophobic polymer and a continuous phase that contains a water-soluble polymer.
<2> The on-press development type lithographic printing plate precursor described in <1>, in which a contact angle of water on a surface of the outermost layer that is measured 30 seconds after the water is landed as a droplet of water-in-oil is 60° to 160°.
<3> The on-press development type lithographic printing plate precursor described in <1> or <2>, in which a contact angle of water on a surface of the outermost layer that is measured 60 seconds after the water is landed as a droplet of water-in-oil is 60° to 160°.
<4> The on-press development type lithographic printing plate precursor described in any one of <1> to <3>, in which the hydrophobic polymer is particles.
<5> The on-press development type lithographic printing plate precursor described in <4>, in which the particles are crosslinked particles.
<6> The on-press development type lithographic printing plate precursor described in <4> or <5>, in which the particles have a dispersible group.
<7> The on-press development type lithographic printing plate precursor described in <6>, in which the dispersible group includes a group represented by Formula Z.

   *-Q-W-Y Formula Z

   In Formula Z, Q represents a divalent linking group, W represents a divalent group having a hydrophilic structure or a divalent group having a hydrophobic structure, Y represents a monovalent group having a hydrophilic structure, either W or Y has a hydrophilic structure, and * represents a bonding site with another structure.
<8> The on-press development type lithographic printing plate precursor described in <6> or <7>, in which the dispersible group has a polyalkylene oxide structure.
<9> The on-press development type lithographic printing plate precursor described in any one of <1> to <8>, in which the water-soluble polymer includes polyvinyl alcohol.
<10> The on-press development type lithographic printing plate precursor described in <9>, in which a saponification degree of the polyvinyl alcohol is 65% to 100%.
<11> The on-press development type lithographic printing plate precursor described in any one of <1> to <10>, in which the image-recording layer or the outermost layer contains a fluorohydrocarbon group-containing copolymer.
<12> The on-press development type lithographic printing plate precursor described in <11>, in which the fluorohydrocarbon group-containing copolymer includes constitutional units derived from monomers represented by Formula (F1) to Formula (F3). In Formula (F1) to Formula (F3), R^{F1} each independently represent a hydrogen atom or a methyl group, L^{F} represents a single bond or a divalent linking group, Cf represents a linear or branched hydrocarbon group having 1 to 10 carbon atoms in which some or all of hydrogen atoms of the hydrocarbon group are substituted with fluorine atoms, X^{F} each independently represent an oxygen atom, a sulfur atom, or -N(R^{F3})-, R^{F2} represents a hydrogen atom or a fluorine atom, w1 to w3 each independently represent an integer of 0 to 9, w4 represents an integer of 1 to 10, w5 represents an integer of 0 to 2, and R^{F3} represents a hydrogen atom or an alkyl group having 1 to 4 carbon atoms.
<13> The on-press development type lithographic printing plate precursor described in <12>, in which the fluorohydrocarbon group-containing copolymer includes a constitutional unit derived from a monomer represented by Formula (F2) or Formula (F3).
<14> The on-press development type lithographic printing plate precursor described in any one of <11> to <13>, in which the fluorohydrocarbon group-containing copolymer includes a constitutional unit having a polyalkylene oxide structure.
<15> The on-press development type lithographic printing plate precursor described in any one of <1> to <14>, in which the outermost layer contains a preservative.
<16> The on-press development type lithographic printing plate precursor described in any one of <1> to <15>, in which the outermost layer contains a discoloring compound.
<17> The on-press development type lithographic printing plate precursor described in <16>, in which the discoloring compound includes a decomposable compound that decomposes due to exposure to infrared.
<18> The on-press development type lithographic printing plate precursor described in any one of <1> to <17>, in which the image-recording layer contains an infrared absorber, an electron-accepting polymerization initiator, an electron-donating polymerization initiator, and a polymerizable compound.
<19> The on-press development type lithographic printing plate precursor described in <18>, in which an energy level of HOMO of the infrared absorber - an energy level HOMO of the electron-donating polymerization initiator is 0.70 eV or less.
<20> The on-press development type lithographic printing plate precursor described in <18> or <19>, in which an energy level of LUMO of the electron-accepting polymerization initiator - an energy level of LUMO of the infrared absorber is 1.00 eV or less.
<21> The on-press development type lithographic printing plate precursor described in any one of <18> to <20>, in which the electron-accepting polymerization initiator is an onium salt compound.
<22> The on-press development type lithographic printing plate precursor described in any one of <18> to <20>, in which the electron-accepting polymerization initiator includes a compound represented by Formula (II). In Formula (II), X^{A} represents a halogen atom, and R^{A} represents an aryl group.
<23> The on-press development type lithographic printing plate precursor described in any one of <18> to <22>, in which the polymerizable compound includes a polymerizable compound having functionalities of 2 or less.
<24> The on-press development type lithographic printing plate precursor described in any one of <18> to <23>, in which the polymerizable compound includes a polymerizable compound having functionalities of 7 or more.
<25> The on-press development type lithographic printing plate precursor described in any one of <1> to <24>, in which the image-recording layer contains polyvinyl acetal.
<26> The on-press development type lithographic printing plate precursor described in any one of <1> to <25>, in which the support has an aluminum plate and an anodic oxide film of aluminum disposed on the aluminum plate, the anodic oxide film is at a position closer to a side of the image-recording layer than the aluminum plate and has micropores extending in a depth direction from a surface of the anodic oxide film on the side of the image-recording layer, and an average diameter of the micropores within the surface of the anodic oxide film is more than 10 nm and 100 nm or less.
<27> The on-press development type lithographic printing plate precursor described in <26>, in which the micropores are each composed of a large diameter portion that extends to a position at a depth of 10 nm to 1,000 nm from the surface of the anodic oxide film and a small diameter portion that is in communication with a bottom portion of the large diameter portion and extends to a position at a depth of 20 nm to 2,000 nm from a communicate position, an average diameter of the large diameter portion within the surface of the anodic oxide film is 15 nm to 100 nm, and an average diameter of the small diameter portion at the communicate position is 15 nm or less.
<28> A method of preparing a lithographic printing plate, including a step of exposing the on-press development type lithographic printing plate precursor described in any one of <1> to <27> in a shape of an image, and a step of supplying at least one of a printing ink or dampening water on a printer to remove the image-recording layer in a non-image area.
<29> A lithographic printing method including a step of exposing the on-press development type lithographic printing plate precursor described in any one of <1> to <27> in a shape of an image, a step of supplying at least one of a printing ink or dampening water to remove the image-recording layer in a non-image area on a printer and to prepare a lithographic printing plate, and a step of performing printing by using the obtained lithographic printing plate.

According to an embodiment of the present disclosure, it is possible to provide an on-press development type lithographic printing plate precursor excellent in receptivity and on-press development residue suppressiveness.

According to another embodiment of the present disclosure, it is possible to provide a method of preparing a lithographic printing plate and a printing method using a lithographic printing plate in which the on-press development type lithographic printing plate precursor is used.

### BRIEF DESCRIPTION OF THE DRAWINGS

Fig. 1 is a schematic cross-sectional view of an embodiment of an aluminum support suitably used in the present disclosure.
Fig. 2 is a schematic cross-sectional view of an embodiment of an aluminum support having an anodic oxide film.
Fig. 3 is a schematic view of an anodization treatment device used for an anodization treatment in a manufacturing method of an aluminum support having an anodic oxide film.

### DESCRIPTION OF THE PREFERRED EMBODIMENTS

Hereinafter, the contents of the present disclosure will be specifically described. The following configuration requirements will be described on the basis of typical embodiments of the present disclosure, but the present disclosure is not limited to such embodiments.

In the present specification, a numerical range expressed using "to" includes numerical values listed before and after "to" as the lower limit and the upper limit.

Regarding the numerical ranges described stepwise in the present disclosure, the upper limit or lower limit of a certain numerical range may be replaced with the upper limit or lower limit of another numerical range described stepwise. Furthermore, regarding the numerical ranges described in the present disclosure, the upper or lower limit of a numerical range may be replaced with values described in examples.

In addition, in the present specification, in a case where there is no description regarding whether a group (atomic group) is substituted or unsubstituted, such a group includes both a group having no substituent and a group having a substituent. For example, "alkyl group" includes not only an alkyl group having no substituent (unsubstituted alkyl group) but also an alkyl group having a substituent (substituted alkyl group).

In the present specification, "(meth)acryl" is a term used to explain a concept including both the acryl and methacryl, and "(meth)acryloyl" is a term used to explain a concept including both the acryloyl and methacryloyl.

In addition, the term "step" in the present specification means not only an independent step but also a step that cannot be clearly differentiated from other steps as long as the intended goal of the step is achieved. In the present disclosure, "% by mass" has the same definition as "% by weight", and "part by mass" has the same definition as "part by weight".

In the present disclosure, unless otherwise specified, as each component contained in a composition or each constitutional unit contained in a polymer, one kind of component or one kind of constitutional unit may be used alone, or two or more kinds of components or two or more kinds of constitutional units may be used in combination.

Furthermore, in the present disclosure, in a case where there is a plurality of substances corresponding to each component in a composition, or in a case where there is a plurality of constitutional units corresponding to each constitutional unit in a polymer, unless otherwise specified, the amount of each component in the composition or the amount of each constitutional unit in the polymer means the total amount of the plurality of corresponding substances present in the composition or the total amount of the plurality of corresponding constitutional units present in the polymer.

In the present disclosure, a combination of two or more preferred aspects is a more preferred aspect.

In addition, in the present disclosure, unless otherwise specified, each of the weight-average molecular weight (Mw) and number-average molecular weight (Mn) is a molecular weight that is detected using a gel permeation chromatography (GPC) analysis device using TSKgel GMHxL, TSKgel G4000HxL, and TSKgel G2000HxL (trade names, manufactured by Tosoh Corporation) as columns, tetrahydrofuran (THF) as a solvent, and a differential refractometer, and expressed in terms of polystyrene as a standard substance.

In the present disclosure, the term "lithographic printing plate precursor" refers not only to a lithographic printing plate precursor but also to a key plate precursor. In addition, the term "lithographic printing plate" refers not only to a lithographic printing plate prepared by performing operations such as exposure and development as necessary on a lithographic printing plate precursor but also to a key plate. The key plate precursor is not necessarily subjected to the operations such as exposure and development. The key plate refers to a lithographic printing plate precursor to be mounted on a plate cylinder that is not used, in a case where monochromatic or dichromatic printing is carried out on a part of paper during, for example, color newspaper printing.

In the present disclosure, "excellent printing durability" means that a large number of sheets can be printed using a lithographic printing plate, and printing durability exhibited in a case where a UV ink is used as a printing ink will be also described as "UV printing durability" hereinafter.

Hereinafter, the present disclosure will be specifically described.

### (On-press development type lithographic printing plate precursor)

The on-press development type lithographic printing plate precursor according to the present disclosure (also simply called "lithographic printing plate precursor") has a support, an image-recording layer, and an outermost layer in this order, in which the outermost layer has a sea-island structure consisting of a discontinuous phase that contains a hydrophobic polymer and a continuous phase that contains a water-soluble polymer.

In addition, the on-press development type lithographic printing plate precursor according to the present disclosure is preferably a negative tone lithographic printing plate precursor.

The inventors of the present invention have found that in the lithographic printing plate precursor of the related art having an outermost layer, such as the lithographic printing plate precursor described in JP2006-264300A or WO2019/243036A, the components contained in the outermost layer are fused by heat and make the surface of the image-recording layer hydrophilic, which leads to the deterioration of receptivity and the occurrence of on-press development residues derived from the outermost layer and thus makes it difficult to simultaneously achieve receptivity and on-press development residue suppressiveness.

As a result of intensive studies, the inventors of the present invention have found that adopting the above constitution makes it possible to provide an on-press development type lithographic printing plate precursor excellent in receptivity and on-press development residue suppressiveness.

The detailed mechanism that brings about the aforementioned effect is unclear, but is assumed to be as below.

Because the outermost layer has a sea-island structure consisting of a discontinuous phase that contains a hydrophobic polymer and a continuous phase that contains a water-soluble polymer, in a non-image area, the hydrophobic polymer is a discontinuous phase. Presumably, as a result, the discontinuous phase may be maintained during development, and the polymers are unlikely to go through aggregation and the like, which may make it possible to suppress the occurrence of on-press development residues in dampening water, on a water supply roller, and the like. Furthermore, in an image area, the hydrophobic polymer is a discontinuous phase. Presumably, as a result, it may be possible to inhibit the hydrophobic polymers from being fused by heat and to thoroughly remove the hydrophobic polymers, which may result in excellent receptivity.

From the viewpoint of on-press development residue suppressiveness, printing durability, and on-press developability, the contact angle of water on a surface of the outermost layer of the on-press development type lithographic printing plate precursor according to the present disclosure (a surface of the outermost layer opposite to the side of the image-recording layer) that is measured 30 seconds after the water is landed as a droplet of water-in-oil is preferably 60° to 160°, more preferably 100° to 155°, and particularly preferably 120° to 150°.

From the viewpoint of on-press development residue suppressiveness, printing durability, and on-press developability, the contact angle of water on a surface of the outermost layer of the on-press development type lithographic printing plate precursor according to the present disclosure (a surface of the outermost layer opposite to the side of the image-recording layer) that is measured 60 seconds after the water is landed as a droplet of water-in-oil is preferably 60° to 160°, more preferably 100° to 155°, and particularly preferably 120° to 150°.

In the present disclosure, the contact angle of water as a droplet of water-in-oil on the surface of the outermost layer of the on-press development type lithographic printing plate precursor is measured by the following method.

By using a contact angle meter (Model: DMC-MC3) manufactured by Kyowa Interface Science Co., Ltd., the lithographic printing plate precursor is mounted on a fixing tool and put in a glass cell filled with linseed oil to prepare a sample. At 25°C, 1 µL of pure water is added dropwise to the precursor in the linseed oil. Then, 30 seconds or 60 seconds after the pure water is added dropwise, the angle between the precursor surface and a tangent of the water droplet interface at an intersection between the landed pure water droplet and the precursor surface is measured as a contact angle. It is preferable to promptly measure the contact angle after the precursor is put in the linseed oil. The precursor left in the oil for 2 minutes or more is not suitable for the measurement. The contact angle is measured at 3 or more sites on the same precursor, and the average thereof is adopted.

Hereinafter, each layer in the lithographic printing plate precursor according to the present disclosure will be specifically described.

### <Outermost layer>

The on-press development type lithographic printing plate precursor according to the present disclosure has a support, an image-recording layer, and an outermost layer in this order, in which the outermost layer has a sea-island structure consisting of a discontinuous phase that contains a hydrophobic polymer and a continuous phase that contains a water-soluble polymer.

From the viewpoint of forming a sea-island structure, it is preferable that the hydrophobic polymer and the water-soluble polymer be incompatible with each other.

The outermost layer is preferably removable with at least one of dampening water or a printing ink, and more preferably removable with dampening water.

The outermost layer may have functions such as suppressing the reaction inhibiting image formation by blocking oxygen, preventing the damage of the image-recording layer, and preventing ablation during exposure to high-illuminance lasers.

In the outermost layer, the discontinuous phase containing the hydrophobic polymer may or may not be exposed on the surface of the outermost layer. It is preferable that at least a part of the discontinuous phase in the outermost layer be exposed on the surface of the outermost layer.

In the present disclosure, the sea-island structure is a structure in which a discontinuous phase is dispersed in a continuous phase.

In the present disclosure, the sea-island structure is confirmed by a method of cutting the precursor with a microtome or the like or bending the precursor such that the cross section is exposed, then imparting conductivity to the cross section of the outermost layer and the image-recording layer, and imaging and observing the cross section by using a scanning electron microscope (SEM).

From the viewpoint of on-press development residue suppressiveness, on-press developability, printing durability, and receptivity, the proportion of the discontinuous phase containing a hydrophobic polymer in the surface of the outermost layer is preferably 1% by area to 99% by area, more preferably 5% by area to 90% by area, and particularly preferably 60% by area to 80% by area.

In a case where M^{OA} represents the total mass of the discontinuous phase in the outermost layer and M^{OB} represents the total mass of the continuous phase in the outermost layer, from the viewpoint of on-press development residue suppressiveness, on-press developability, printing durability, and receptivity, M^{OA} and M^{OB} preferably satisfy M^{OA} < M^{OB}, and the mass ratio of the continuous phase to the discontinuous phase (M^{OB}/M^{OA}) in the outermost layer is more preferably more than 1 and 10 or less, even more preferably 1.5 to 8, and particularly preferably 2 to 6.

In addition, in a case where M^{OC} represents the total mass of the hydrophobic polymer in the outermost layer and M^{OD} represents the total mass of the water-soluble polymer in the outermost layer, from the viewpoint of on-press development residue suppressiveness, on-press developability, printing durability, and receptivity, M^{OC} and M^{OD} preferably satisfy M^{OC} < M^{OD}, and the mass ratio of the hydrophobic polymer to the water-soluble polymer (M^{OC}/M^{OD}) contained in the outermost layer is preferably more than 1 and 10 or less, even more preferably 1.5 to 8, and particularly preferably 2 to 6.

The average particle diameter of the discontinuous phase is preferably 0.01 µm to 3.0 µm, more preferably 0.03 µm to 2.0 µm, and particularly preferably 0.10 µm to 1.0 µm.

### -Water-soluble polymer-

The outermost layer has a sea-island structure having a continuous phase containing a water-soluble polymer.

In the present disclosure, a water-soluble polymer refers to a polymer that dissolves 1 g or more in 100 g of pure water at 70°C and is not precipitated even though a solution of 1 g of the polymer in 100 g of pure water at 70°C is cooled to 25°C.

Examples of the water-soluble polymer used in the outermost layer include polyvinyl alcohol, modified polyvinyl alcohol, polyvinylpyrrolidone, a water-soluble cellulose derivative, polyethylene glycol, poly(meth)acrylonitrile, and the like.

As the modified polyvinyl alcohol, acid-modified polyvinyl alcohol having a carboxy group or a sulfo group is preferably used. Specific examples thereof include modified polyvinyl alcohols described in JP2005-250216A and JP2006-259137A.

Preferred examples of the water-soluble polymer include polyvinyl alcohol. Particularly, as the water-soluble polymer to be used, polyvinyl alcohol having a saponification degree (hydrolysis degree) of 50% or more is more preferable.

The saponification degree is preferably 65% to 100%, more preferably 70% to 100%, and even more preferably 85% to 100%.

The saponification degree is measured according to the method described in JIS K 6726: 1994.

Preferred examples of the water-soluble polymer also include polyvinylpyrrolidone.

As the water-soluble polymer, it is also preferable to use polyvinyl alcohol and polyvinylpyrrolidone in combination.

One kind of water-soluble polymer may be used alone, or two or more kinds of water-soluble polymers may be used in combination.

In a case where the outermost layer contains a water-soluble polymer, the content of the water-soluble polymer with respect to the total mass of the outermost layer is preferably 1% by mass to 99% by mass, more preferably 3% by mass to 97% by mass, and even more preferably 5% by mass to 95% by mass.

### <Hydrophobic polymer>

The outermost layer has a sea-island structure having a discontinuous phase containing a hydrophobic polymer.

The hydrophobic polymer refers to a polymer that dissolves less than 1 g or does not dissolve in 100 g of pure water at 70°C.

Examples of the hydrophobic polymer include polyethylene, polystyrene, polyvinyl chloride, polyvinylidene chloride, polyalkyl (meth)acrylate ester (for example, polymethyl (meth)acrylate, polyethyl (meth)acrylate, polybutyl (meth)acrylate, and the like), a copolymer obtained by combining raw material monomers of these polymers, and the like.

The hydrophobic polymer preferably includes a polyvinylidene chloride resin.

Furthermore, the hydrophobic polymer preferably includes a styrene-acrylic copolymer.

Furthermore, as the hydrophobic polymer, among the resins having a fluorine atom that will be described later, a resin exhibiting hydrophobicity can also be suitably used.

From the viewpoint of on-press developability, the hydrophobic polymer is preferably particles, that is, hydrophobic polymer particles.

In a case where the hydrophobic polymer is in the form of particles, the hydrophobicity of the surface of the outermost layer can be further improved. For example, the hydrophobic polymer in the form of particles can form a sea-island structure including the hydrophobic polymer as an island region (that is, a discontinuous phase) on the surface of the outermost layer. The sea-island structure described above can contribute to the improvement of hydrophobicity. In the present disclosure, the shape of the hydrophobic polymer whose contour is confirmed by surface observation (that is, plane view) of the outermost layer is regarded as a particle. The shape of contour of the hydrophobic polymer confirmed by the surface observation of the outermost layer is not limited to a perfect circle, and may be, for example, an ellipse, a polygon, or an amorphous shape.

From the viewpoint of printing durability and on-press developability, the hydrophobic polymer particles are preferably crosslinked particles. The crosslinked particles are particles containing a hydrophobic polymer having a crosslinked structure, and are preferably hydrophobic polymer particles obtained by at least polymerizing a polyfunctional polymerizable compound.

From the viewpoint of printing durability, on-press development residue suppressiveness, and on-press developability, it is preferable that the hydrophobic polymer particles have a dispersible group.

As the dispersible group, a hydrophilic group is preferable, and a group represented by Formula Z is more preferable.

*-Q-W-Y Formula Z

In Formula Z, Q represents a divalent linking group, W represents a divalent group having a hydrophilic structure or a divalent group having a hydrophobic structure, Y represents a monovalent group having a hydrophilic structure or a monovalent group having a hydrophobic structure, either W or Y has a hydrophilic structure, and * represents a bonding site with another structure.

From the viewpoint of UV printing durability and on-press developability, the dispersible group is preferably a hydrophilic group.

The hydrophilic group is not particularly limited as long as it has a hydrophilic structure, and examples thereof include an acid group such as a carboxy group, a hydroxy group, an amino group, a cyano group, a polyalkylene oxide structure, and the like.

Among these, from the viewpoint of on-press developability and UV printing durability, a polyalkylene oxide structure is preferable, and a polyethylene oxide structure, a polypropylene oxide structure, or a polyethylene/propylene oxide structure is more preferable.

Furthermore, from the viewpoint of on-press developability and suppressing the occurrence of development residues during on-press development, the polyalkylene oxide structure preferably has a polypropylene oxide structure, and more preferably has a polyethylene oxide structure and a polypropylene oxide structure.

Furthermore, from the viewpoint of printing durability, receptivity, and on-press developability, the hydrophobic polymer particles preferably include polymer particles having a group represented by Formula Z.

Q in Formula Z is preferably a divalent linking group having 1 to 20 carbon atoms (number of carbon atoms), and more preferably a divalent linking group having 1 to 10 carbon atoms.

Furthermore, Q in Formula Z is preferably an alkylene group, an arylene group, an ester bond, an amide bond, or a group formed by combining two or more of these, and more preferably a phenylene group, an ester bond, or an amide bond.

The divalent group having a hydrophilic structure represented by W in Formula Z is preferably a polyalkyleneoxy group or a group in which -CH₂CH₂NR^{W}- is bonded to one terminal of a polyalkyleneoxy group. R^{W} represents a hydrogen atom or an alkyl group.

The divalent group having a hydrophobic structure represented by W in Formula Z is preferably -R^{WA}-, -O-R^{WA}-O-, -R^{W}N-R^{WA}-NR^{W}-, -OC(=O)-R^{WA}-O-, or -OC(=O)-R^{WA}-O-. R^{WA} each independently represent a linear, branched, or cyclic alkylene group having 6 to 120 carbon atoms, a haloalkylene group having 6 to 120 carbon atoms, an arylene group having 6 to 120 carbon atoms, an alkarylene group having 7 to 120 carbon atoms (divalent group formed by removing one hydrogen atom from an alkylaryl group), or an aralkylene group having 7 to 120 carbon atoms.

The monovalent group having a hydrophilic structure represented by Y in Formula Z is preferably -OH, -C(=O)OH, a polyalkyleneoxy group having a hydrogen atom or an alkyl group on a terminal, or a group in which -CH₂CH₂N(R^{W})- is bonded to one terminal of a polyalkyleneoxy group having a hydrogen atom or an alkyl group on the other terminal.

The monovalent group having a hydrophobic structure represented by Y in Formula Z is preferably a linear, branched, or cyclic alkyl group having 6 to 120 carbon atoms, a haloalkyl group having 6 to 120 carbon atoms, an aryl group having 6 to 120 carbon atoms, an alkaryl group having 7 to 120 carbon atoms (alkylaryl group), an aralkyl group having 7 to 120 carbon atoms, -OR^{WB}, -C(=O)OR^{WB}, or -OC(=O)R^{WB}. R^{WB} represents an alkyl group having 6 to 20 carbon atoms.

From the viewpoint of printing durability, receptivity, and on-press developability, in the hydrophobic polymer particles having a group represented by Formula Z, W is more preferably a divalent group having a hydrophilic structure, Q is more preferably a phenylene group, an ester bond, or an amide bond, W is more preferably a polyalkyleneoxy group, and Y is more preferably a polyalkyleneoxy group having a hydrogen atom or an alkyl group on a terminal.

The average particle diameter of the hydrophobic polymer particles is preferably 0.01 µm to 3.0 µm, more preferably 0.03 µm to 2.0 µm, and particularly preferably 0.10 µm to 1.0 µm.

In the present disclosure, the average primary particle diameter of the hydrophobic polymer particles is measured using a light scattering method or by capturing an electron micrograph of the particles, measuring the particle diameter of a total of 5,000 particles in the photograph, and calculating the average thereof. For non-spherical particles, the value of particle diameter of spherical particles having the same area as the area of the particles on the photograph is adopted as the particle diameter.

Note that unless otherwise specified, the average particle diameter in the present disclosure means a volume average particle diameter.

One kind of hydrophobic polymer may be used alone, or two or more kinds of hydrophobic polymers may be used in combination.

In a case where the outermost layer contains a hydrophobic polymer, the content of the hydrophobic polymer with respect to the total mass of the outermost layer is preferably 1% by mass to 80% by mass, and more preferably 5% by mass to 50% by mass.

### -Other components-

The outermost layer may contain other components such as a discoloring compound, an acid generator, a preservative, a resin having a fluorine atom, a surfactant, an oil sensitizing agent, and an infrared absorber, in addition to the water-soluble polymer and hydrophobic polymer described above.

Hereinafter, those other components will be described.

### «Discoloring compound»

Furthermore, the outermost layer preferably contains a discoloring compound.

In the present disclosure, "discoloring compound" refers to a compound which undergoes change in absorption in the visible light region (wavelength: 400 nm or more and less than 750 nm) due to the exposure to infrared. That is, in the present disclosure, "discoloring" means that the absorption in the visible light region (that is, wavelength: 400 nm or more and less than 750 nm) changes due to the exposure to infrared.

Specifically, examples of the discoloring compound in the present disclosure include (1) compound that absorbs more light in the visible light region due to the exposure to infrared than before the exposure to infrared, (2) compound that is made capable of absorbing light in the visible light region due to the exposure to infrared, and (3) compound that is made incapable of absorbing light in the visible light region due to the exposure to infrared.

The infrared in the present disclosure is a ray having a wavelength of 750 nm to 1 mm, and preferably a ray having a wavelength of 750 nm to 1,400 nm.

The discoloring compound preferably includes a compound that develops color due to the exposure to infrared.

Furthermore, the discoloring compound preferably includes a decomposable compound that decomposes due to the exposure to infrared, and particularly preferably includes a decomposable compound that decomposes by either or both of heat and electron migration due to the exposure to infrared.

More specifically, the discoloring compound in the present disclosure is preferably a compound that decomposes due to the exposure to infrared (more preferably, decomposes by either or both of heat or electron migration due to the exposure to infrared) and absorbs more light in the visible light region than before the exposure to infrared or is made capable of absorbing light of shorter wavelengths and thus capable of absorbing light in the visible light region.

"Decomposes by electron migration" mentioned herein means that electrons excited to the lowest unoccupied molecular orbital (LUMO) from the highest occupied molecular orbital (HOMO) of the discoloring compound by exposure to infrared move to electron accepting groups (groups having potential close to LUMO) in a molecule by means of intramolecular electron migration and thus result in decomposition.

Hereinafter, as an example of the discoloring compound, a decomposable compound will be described.

There are no limitations on the decomposable compound as long as it absorbs at least a part of light in the infrared wavelength region (that is, a wavelength region of 750 nm to 1 mm, preferably a wavelength region of 750 nm to 1,400 nm) and decomposes. The decomposable compound is preferably a compound having maximum absorption in a wavelength region of 750 nm to 1,400 nm.

More specifically, the decomposable compound is preferably a compound that decomposes due to the exposure to infrared and generates a compound having maximum absorption wavelength in a wavelength region of 500 nm to 600 nm.

From the viewpoint of improving visibility of exposed portions, the decomposable compound is preferably a cyanine dye having a group that decomposes by exposure to infrared (specifically, R¹ in Formula 1-1 to Formula 1-7).

From the viewpoint of improving visibility of exposed portions, the decomposable compound is more preferably a compound represented by Formula 1-1.

In Formula 1-1, R¹ represents a group that is represented by any of Formula 2-1 to Formula 4-1, R¹¹ to R¹⁸ each independently represent a hydrogen atom, a halogen atom, -R^{a}, -OR^{b}, -SR^{c}, or -NR^{d}R^{e}, R^{a} to R^{e} each independently represent a hydrocarbon group, A₁, A₂, and a plurality of R¹¹ to R¹⁸ may be linked to each other to form a monocyclic or polycyclic ring, A₁ and A₂ each independently represent an oxygen atom, a sulfur atom, or a nitrogen atom, n₁₁ and n₁₂ each independently represent an integer of 0 to 5, the sum of n₁₁ and n₁₂ is 2 or more, n₁₃ and n₁₄ each independently represent 0 or 1, L represents an oxygen atom, a sulfur atom, or -NR¹⁰-, R¹⁰ represents a hydrogen atom, an alkyl group, or an aryl group, and Za represents a counterion that neutralizes charge.

In Formula 2-1 to Formula 4-1, R²⁰, R³⁰, R⁴¹, and R⁴² each independently represent an alkyl group or an aryl group, Zb represents a counterion that neutralizes charge, a wavy line represents a bonding site with a group represented by L in Formula 1-1.

In a case where the compound represented by Formula 1-1 is exposed to infrared, the R¹-L bond is cleaved, L turns into =O, =S, or =NR¹⁰, and the compound is discolored.

In Formula 1-1, R¹ represents a group represented by any of Formula 2-1 to Formula 4-1.

Hereinafter, each of the group represented by Formula 2-1, the group represented by Formula 3-1, and the group represented by Formula 4-1 will be described.

In Formula 2-1, R²⁰ represents an alkyl group or an aryl group, and the portion of the wavy line represents a bonding site with the group represented by L in Formula 1-1.

As the alkyl group represented by R²⁰, an alkyl group having 1 to 30 carbon atoms is preferable, an alkyl group having 1 to 15 carbon atoms is more preferable, and an alkyl group having 1 to 10 carbon atoms is even more preferable.

The alkyl group may be linear or branched, or may have a ring structure.

The aryl group represented by R²⁰ is preferably an aryl group having 6 to 30 carbon atoms, more preferably an aryl group having 6 to 20 carbon atoms, and even more preferably an aryl group having 6 to 12 carbon atoms.

From the viewpoint of visibility, R²⁰ is preferably an alkyl group.

From the viewpoint of decomposition properties and visibility, the alkyl group represented by R²⁰ is preferably a secondary alkyl group or a tertiary alkyl group, and preferably a tertiary alkyl group.

Furthermore, from the viewpoint of decomposition properties and visibility, the alkyl group represented by R²⁰ is preferably an alkyl group having 1 to 8 carbon atoms, more preferably a branched alkyl group having 3 to 10 carbon atoms, even more preferably a branched alkyl group having 3 to 6 carbon atoms, particularly preferably an isopropyl group or a tert-butyl group, and most preferably a tert-butyl group.

Specific examples of the group represented by Formula 2-1 will be shown below. However, the present disclosure is not limited thereto. In the following structural formulas, ● represents a bonding site with the group represented by L in Formula 1-1.

In Formula 3-1, R³⁰ represents an alkyl group or an aryl group, and the portion of the wavy line represents a bonding site with the group represented by L in Formula 1-1.

The alkyl group and aryl group represented by R³⁰ are the same as the alkyl group and aryl group represented by R²⁰ in Formula 2-1, and the preferred aspects thereof are also the same.

From the viewpoint of decomposition properties and visibility, the alkyl group represented by R³⁰ is preferably a secondary alkyl group or a tertiary alkyl group, and preferably a tertiary alkyl group.

Furthermore, from the viewpoint of decomposition properties and visibility, the alkyl group represented by R³⁰ is preferably an alkyl group having 1 to 8 carbon atoms, more preferably a branched alkyl group having 3 to 10 carbon atoms, even more preferably a branched alkyl group having 3 to 6 carbon atoms, particularly preferably an isopropyl group or a tert-butyl group, and most preferably a tert-butyl group.

In addition, from the viewpoint of decomposition properties and visibility, the alkyl group represented by R³⁰ is preferably a substituted alkyl group, more preferably a fluoro-substituted alkyl group, even more preferably a perfluoroalkyl group, and particularly preferably a trifluoromethyl group.

From the viewpoint of decomposition properties and visibility, the aryl group represented by R³⁰ is preferably a substituted aryl group. Examples of the substituent include an alkyl group (preferably an alkyl group having 1 to 4 carbon atoms), an alkoxy group (preferably an alkoxy group having 1 to 4 carbon atoms), and the like.

Specific examples of the group represented by Formula 3-1 will be shown below. However, the present disclosure is not limited thereto. In the following structural formulas, ● represents a bonding site with the group represented by L in Formula 1-1.

In Formula 4-1, R⁴¹ and R⁴² each independently represent an alkyl group or an aryl group, Zb represents a counterion that neutralizes charge, and the portion of the wavy line represents a bonding site with the group represented by L in Formula 1-1.

The alkyl group and aryl group represented by R⁴¹ or R⁴² are the same as the alkyl group and aryl group represented by R²⁰ in Formula 2-1, and preferred aspects thereof are also the same.

From the viewpoint of decomposition properties and visibility, R⁴¹ is preferably an alkyl group.

From the viewpoint of decomposition properties and visibility, R⁴² is preferably an alkyl group.

From the viewpoint of decomposition properties and visibility, the alkyl group represented by R⁴¹ is preferably an alkyl group having 1 to 8 carbon atoms, more preferably an alkyl group having 1 to 4 carbon atoms, and particularly preferably a methyl group.

From the viewpoint of decomposition properties and visibility, the alkyl group represented by R⁴² is preferably a secondary alkyl group or a tertiary alkyl group, and preferably a tertiary alkyl group.

Furthermore, from the viewpoint of decomposition properties and visibility, the alkyl group represented by R⁴² is preferably an alkyl group having 1 to 8 carbon atoms, more preferably a branched alkyl group having 3 to 10 carbon atoms, even more preferably a branched alkyl group having 3 to 6 carbon atoms, particularly preferably an isopropyl group or a tert-butyl group, and most preferably a tert-butyl group.

Zb in Formula 4-1 may be a counterion that neutralizes charge, and may be included in Za in Formula 1-1 in the entirety of the compound.

Zb is preferably a sulfonate ion, a carboxylate ion, a tetrafluoroborate ion, a hexafluorophosphate ion, a p-toluenesulfonate ion, or a perchlorate ion, and more preferably a tetrafluoroborate ion.

Specific examples of the group represented by Formula 4-1 will be shown below. However, the present disclosure is not limited thereto. In the following structural formulas, ● represents a bonding site with the group represented by L in Formula 1-1.

L in Formula 1-1 is preferably an oxygen atom or -NR¹⁰-, and particularly preferably an oxygen atom.

Furthermore, R¹⁰ in -NR¹⁰- is preferably an alkyl group. The alkyl group represented by R¹⁰ is preferably an alkyl group having 1 to 10 carbon atoms. The alkyl group represented by R¹⁰ may be linear or branched, or may have a ring structure.

Among the alkyl groups, a methyl group or a cyclohexyl group is preferable.

In a case where R¹⁰ in -NR¹⁰- represents an aryl group, the aryl group is preferably an aryl group having 6 to 30 carbon atoms, more preferably an aryl group having 6 to 20 carbon atoms, and even more preferably an aryl group having 6 to 12 carbon atoms. These aryl groups may have a substituent.

In Formula 1-1, R¹¹ to R¹⁸ preferably each independently represent a hydrogen atom, -R^{a}, -OR^{b}, -SR^{c}, or -NR^{d}R^{e}.

The hydrocarbon group represented by R^{a} to R^{e} is preferably a hydrocarbon group having 1 to 30 carbon atoms, more preferably a hydrocarbon group having 1 to 15 carbon atoms, and even more preferably a hydrocarbon group having 1 to 10 carbon atoms.

The hydrocarbon group may be linear or branched or may have a ring structure.

As the hydrocarbon group, an alkyl group is particularly preferable.

The aforementioned alkyl group is preferably an alkyl group having 1 to 30 carbon atoms, more preferably an alkyl group having 1 to 15 carbon atoms, and even more preferably an alkyl group having 1 to 10 carbon atoms.

The alkyl group may be linear or branched, or may have a ring structure.

Specific examples of the alkyl group include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a hexadecyl group, an octadecyl group, an eicosyl group, an isopropyl group, an isobutyl group, an s-butyl group, a tert-butyl group, an isopentyl group, a neopentyl group, a 1-methylbutyl group, an isohexyl group, a 2-ethylhexyl group, a 2-methylhexyl group, a cyclohexyl group, a cyclopentyl group, and a 2-norbornyl group.

Among these alkyl groups, a methyl group, an ethyl group, a propyl group, or a butyl group is preferable.

The above alkyl group may have a substituent.

Examples of the substituent include an alkoxy group, an aryloxy group, an amino group, an alkylthio group, arylthio group, a halogen atom, a carboxy group, a carboxylate group, a sulfo group, a sulfonate group, an alkyloxycarbonyl group, an aryloxycarbonyl group, groups obtained by combining these, and the like.

R¹¹ to R¹⁴ in Formula 1-1 preferably each independently represent a hydrogen atom or -R^{a} (that is, a hydrocarbon group), more preferably each independently represent a hydrogen atom or an alkyl group, and even more preferably each independently represent a hydrogen atom except in the cases described below.

Particularly, each of R¹¹ and R¹³ bonded to the carbon atom that is bonded to the carbon atom to which L is bonded is preferably an alkyl group. It is more preferable that R¹¹ and R¹³ be linked to each other to form a ring. The ring to be formed in this way may be a monocyclic or polycyclic ring. Specifically, examples of the ring to be formed include a monocyclic ring such as a cyclopentene ring, a cyclopentadiene ring, a cyclohexene ring, or a cyclohexadiene ring, and a polycyclic ring such as an indene ring or an indole ring.

Furthermore, it is preferable that R¹² bonded to the carbon atom to which A₁⁺ is bonded be linked to R¹⁵ or R¹⁶ (preferably R¹⁶) to form a ring, and R¹⁴ bonded to the carbon atom to which A₂ is bonded be linked to R¹⁷ or R¹⁸ (preferably R¹⁸) to form a ring.

In Formula 1-1, n₁₃ is preferably 1, and R¹⁶ is preferably -R^{a} (that is, a hydrocarbon group).

Furthermore, it is preferable that R¹⁶ be linked to R¹² bonded to the carbon atom to which A₁⁺ is bonded, so as to form a ring. As the ring to be formed, an indolium ring, a pyrylium ring, a thiopyrylium ring, a benzoxazoline ring, or a benzimidazoline ring is preferable, and an indolium ring is more preferable from the viewpoint of improving visibility of exposed portions. These rings may further have a substituent.

In Formula 1-1, n₁₄ is preferably 1, and R¹⁸ is preferably -R^{a} (that is, a hydrocarbon group).

Furthermore, it is preferable that R¹⁸ be linked to R¹⁴ bonded to the carbon atom to which A₂ is bonded, so as to form a ring. As the ring to be formed, an indole ring, a pyran ring, a thiopyran ring, a benzoxazole ring, or a benzimidazole ring is preferable, and an indole ring is more preferable from the viewpoint of improving visibility of exposed portions. These rings may further have a substituent.

It is preferable that R¹⁶ and R¹⁸ in Formula 1-1 be the same group. In a case where R¹⁶ and R¹⁸ each form a ring, it is preferable that the formed rings have the same structure except for A₁⁺ and A₂.

It is preferable that R¹⁵ and R¹⁷ in Formula 1-1 be the same group. Furthermore, R¹⁵ and R¹⁷ are preferably -R^{a} (that is, a hydrocarbon group), more preferably an alkyl group, and even more preferably a substituted alkyl group.

From the viewpoint of improving water solubility, R¹⁵ and R¹⁷ in the compound represented by Formula 1-1 are preferably a substituted alkyl group.

Examples of the substituted alkyl group represented by R¹⁵ or R¹⁷ include a group represented by any of Formula (a1) to Formula (a4).

In Formula (a1) to Formula (a4), R^{W0} represents an alkylene group having 2 to 6 carbon atoms, W represents a single bond or an oxygen atom, and n_{W1} represents an integer of 1 to 45, R^{W1} represents an alkyl group having 1 to 12 carbon atoms or -C(=O)-R^{W5}, R^{W5} represents an alkyl group having 1 to 12 carbon atoms, R^{W2} to R^{W4} each independently represent a single bond or an alkylene group having 1 to 12 carbon atoms, and M represents a hydrogen atom, a sodium atom, a potassium atom, or an onium group.

Specific examples of the alkylene group represented by R^{W0} in Formula (a1) include an ethylene group, a n-propylene group, an isopropylene group, a n-butylene group, an isobutylene group, a n-pentylene group, an isopentylene group, a n-hexyl group, an isohexyl group, and the like. Among these, an ethylene group, a n-propylene group, an isopropylene group, or a n-butylene group is preferable, and a n-propylene group is particularly preferable.

n_{W1} is preferably 1 to 10, more preferably 1 to 5, and particularly preferably 1 to 3.

Specific examples of the alkyl group represented by R^{W1} include a methyl group, an ethyl group, a n-propyl group, an isopropyl group, a n-butyl group, an isobutyl group, a tert-butyl group, a n-pentyl group, an isopentyl group, a neopentyl group, a n-hexyl group, a n-octyl group, a n-dodecyl group, and the like. Among these, a methyl group, an ethyl group, a n-propyl group, an isopropyl group, a n-butyl group, or a tert-butyl group is preferable, a methyl group or an ethyl group is more preferable, and a methyl group is particularly preferable.

The alkyl group represented by R^{W5} is the same as the alkyl group represented by R^{W1}. Preferred aspects of the alkyl group represented by R^{W5} are the same as preferred aspects of the alkyl group represented by R^{W1}.

Specific examples of the group represented by Formula (a1) will be shown below. However, the present disclosure is not limited thereto. In the following structural formulas, Me represents a methyl group, Et represents an ethyl group, and * represents a bonding site.

Specific examples of the alkylene group represented by R^{W2} to R^{W4} in Formula (a2) to Formula (a4) include a methylene group, an ethylene group, a n-propylene group, an isopropylene group, a n-butylene group, an isobutylene group, a n-pentylene group, an isopentylene group, a n-hexyl group, an isohexyl group, a n-octylene group, a n-dodecylene group, and the like. Among these, an ethylene group, a n-propylene group, an isopropylene group, or a n-butylene group is preferable, and an ethylene group or a n-propylene group is particularly preferable.

In Formula (a3), two Ms may be the same as or different from each other.

Examples of the onium group represented by M in Formula (a2) to Formula (a4) include an ammonium group, an iodonium group, a phosphonium group, a sulfonium group, and the like.

All of CO₂M in Formula (a2), PO₃M₂ in Formula (a2), and SO₃M in Formula (a4) may have an anion structure from which M is dissociated. The countercation of the anion structure may be A₁⁺ or a cation that can be contained in R¹-L in Formula 1-1.

Among the groups represented by Formula (a1) to Formula (a4), the group represented by Formula (a1), Formula (a2), or Formula (a4) is preferable.

n₁₁ and n₁₂ in Formula 1-1 are preferably the same as each other, and preferably both represent an integer of 1 to 5, more preferably both represent an integer of 1 to 3, even more preferably both represent 1 or 2, and particularly preferably both represent 2.

A₁ and A₂ in Formula 1-1 each independently represent an oxygen atom, a sulfur atom, or a nitrogen atom. Among these, a nitrogen atom is preferable.

A₁ and A₂ in Formula 1-1 are preferably the same atoms.

Za in Formula 1-1 represents a counterion that neutralizes charge.

In a case where all of R¹¹ to R¹⁸ and R¹-L are groups having a neutral charge, Za is a monovalent counteranion. Here, R¹¹ to R¹⁸ and R¹-L may have an anion structure or a cation structure. For example, in a case where two or more among R¹¹ to R¹⁸ and R¹-L have an anion structure, Za can also be a countercation.

In a case where the cyanine dye represented by Formula 1-1 has such a structure that the overall charge of the compound is neutral except for Za, Za is unnecessary.

In a case where Za is a counteranion, examples thereof include a sulfonate ion, a carboxylate ion, a tetrafluoroborate ion, a hexafluorophosphate ion, a p-toluenesulfonate ion, a perchlorate ion, and the like. Among these, a tetrafluoroborate ion is preferable.

In a case where Za is a countercation, examples thereof include an alkali metal ion, an alkaline earth metal ion, an ammonium ion, a pyridinium ion, a sulfonium ion, and the like. Among these, a sodium ion, a potassium ion, an ammonium ion, a pyridinium ion, or a sulfonium ion is preferable, and a sodium ion, a potassium ion, or an ammonium ion is more preferable.

From the viewpoint of improving visibility of exposed portions, the decomposable compound is more preferably a compound represented by Formula 1-2 (that is, a cyanine dye).

In Formula 1-2, R¹ represents a group that is represented by any of Formula 2-1 to Formula 4-1, R¹⁹ to R²² each independently represent a hydrogen atom, a halogen atom, -R^{a}, -OR^{b}, -CN, -SR^{c}, or -NR^{d}R^{e}, R²³ and R²⁴ each independently represent a hydrogen atom or -R^{a}, R^{a} to R^{e} each independently represent a hydrocarbon group, R¹⁹ and R²⁰, R²¹ and R²², or R²³ and R²⁴ may be linked to each other to form a monocyclic or polycyclic ring, L represents an oxygen atom, a sulfur atom, or -NR¹⁰-, R¹⁰ represents a hydrogen atom, an alkyl group, or an aryl group, R^{d1} to R^{d4}, W¹, and W² each independently represent an alkyl group which may have a substituent, and Za represents a counterion that neutralizes charge.

R¹ in Formula 1-2 has the same definition as R¹ in Formula 1-1, and preferred aspects thereof are also the same.

In Formula 1-2, R¹⁹ to R²² preferably each independently represent a hydrogen atom, a halogen atom, -R^{a}, -OR^{b}, or -CN.

More specifically, R¹⁹ and R²¹ are preferably a hydrogen atom or -R^{a}.

Furthermore, R²⁰ and R²² are preferably a hydrogen atom, -R^{a}, -OR^{b}, or -CN.

-R^{a} represented by R¹⁹ to R²² is preferably an alkyl group or an alkenyl group.

In a case where all of R¹⁹ to R²² are -R^{a}, it is preferable that R¹⁹ and R²⁰ and R²¹ and R²² be linked to each other to form a monocyclic or polycyclic ring.

Examples of the ring formed of R¹⁹ and R²⁰ or R²¹ and R²² linked to each other include a benzene ring, a naphthalene ring, and the like.

R²³ and R²⁴ in Formula 1-2 are preferably linked to each other to form a monocyclic or polycyclic ring.

The ring formed of R²³ and R²⁴ linked to each other may be a monocyclic or polycyclic ring. Specifically, examples of the ring to be formed include a monocyclic ring such as a cyclopentene ring, a cyclopentadiene ring, a cyclohexene ring, or a cyclohexadiene ring, and a polycyclic ring such as an indene ring.

R^{d1} to R^{d4} in Formula 1-2 are preferably an unsubstituted alkyl group. Furthermore, all of R^{d1} to R^{d4} are preferably the same group.

Examples of the unsubstituted alkyl group include unsubstituted alkyl groups having 1 to 4 carbon atoms. Among these, a methyl group is preferable.

From the viewpoint of improving water solubility of the compound represented by Formula 1-2, W¹ and W² in Formula 1-2 preferably each independently represent a substituted alkyl group.

Examples of the substituted alkyl group represented by W¹ and W² include a group represented by any of Formula (a1) to Formula (a4) in Formula 1-1, and preferred aspects thereof are also the same.

From the viewpoint of on-press developability, W¹ and W² preferably each independently represent an alkyl group having a substituent. The alkyl group preferably has at least -OCH₂CH₂-, a sulfo group, a salt of a sulfo group, a carboxy group, or a salt of a carboxy group, as the substituent.

Za represents a counterion that neutralizes charge in the molecule.

In a case where all of R¹⁹ to R²², R²³ and R²⁴, R^{d1} to R^{d4}, W¹, W², and R¹-L are groups having a neutral charge, Za is a monovalent counteranion. Here, R¹⁹ to R²², R²³ and R²⁴, R^{d1} to R^{d4}, W¹, W², and R¹-L may have an anion structure or a cation structure. For example, in a case where two or more among R¹⁹ to R²², R²³ and R²⁴, R^{d1} to R^{d4}, W¹, W², and R¹-L have an anion structure, Za can be a countercation.

In a case where the compound represented by Formula 1-2 has such a structure that the overall charge of the compound is neutral except for Za, Za is unnecessary.

Examples of the case where Za is a counteranion are the same as such examples of Za in Formula 1-1, and preferred aspects thereof are also the same. Furthermore, examples of the case where Za is a countercation are the same as such examples of Za in Formula 1-1, and preferred aspects thereof are also the same.

From the viewpoint of decomposition properties and visibility, the cyanine dye as a decomposable compound is even more preferably a compound represented by any of Formula 1-3 to Formula 1-7.

Particularly, from the viewpoint of decomposition properties and visibility, the cyanine dye is preferably a compound represented by any of Formula 1-3, Formula 1-5, and Formula 1-6.

In Formula 1-3 to Formula 1-7, R¹ represents a group that is represented by any of Formula 2-1 to Formula 4-1, R¹⁹ to R²² each independently represent a hydrogen atom, a halogen atom, -R^{a}, -OR^{b}, -CN, -SR^{c}, or -NR^{d}R^{e}, R²⁵ and R²⁶ each independently represent a hydrogen atom, a halogen atom, or -R^{a}, R^{a} to R^{e} each independently represent a hydrocarbon group, R¹⁹ and R²⁰, R²¹ and R²², or R²⁵ and R²⁶ may be linked to each other to form a monocyclic or polycyclic ring, L represents an oxygen atom, a sulfur atom, or -NR¹⁰-, R¹⁰ represents a hydrogen atom, an alkyl group, or an aryl group, R^{d1} to R^{d4}, W¹, and W² each independently represent an alkyl group which may have a substituent, and Za represents a counterion that neutralizes charge.

R¹, R¹⁹ to R²², R^{d1} to R^{d4}, W¹, W², and L in Formula 1-3 to Formula 1-7 have the same definitions as R¹, R¹⁹ to R²², R^{d1} to R^{d4}, W¹, W², and L in Formula 1-2, and preferred aspects thereof are also the same.

R²⁵ and R²⁶ in Formula 1-7 preferably each independently represent a hydrogen atom or an alkyl group, more preferably each independently represent an alkyl group, and particularly preferably each independently represent a methyl group.

Specific examples of the cyanine dye as a decomposable compound will be shown below. However, the present disclosure is not limited thereto.

Furthermore, as the cyanine dye which is a decomposable compound, the infrared absorbing compound described in WO2019/219560A can be suitably used.

The discoloring compound may include an acid color developing agent.

As the acid color developing agent, it is possible to use the compounds described above as acid color developing agents in the image-recording layer, and preferred aspects thereof are also the same.

One kind of discoloring compound may be used alone, or two or more kinds of components may be combined and used as the discoloring compound.

As the discoloring compound, the decomposable compound described above and the acid generator that will be described later may be used in combination.

From the viewpoint of visibility, the content of the discoloring compound in the outermost layer with respect to the total mass of the outermost layer is preferably 0.10% by mass to 50% by mass, more preferably 0.50% by mass to 30% by mass, and even more preferably 1.0% by mass to 20% by mass.

From the viewpoint of visibility, M^{X}/M^{Y} which is a ratio of a content M^{X} of the discoloring compound in the outermost layer to a content M^{Y} of the infrared absorber in the image-recording layer is preferably 0.1 or more, more preferably 0.2 or more, and particularly preferably 0.3 or more and 3.0 or less.

### <<Acid generator>>

In a case where an acid color developing agent is used as a discoloring compound, the outermost layer preferably contains an acid generator.

"Acid generator" in the present disclosure is a compound that generates an acid by light or heat. Specifically, the acid generator refers to a compound that generates an acid by being decomposed by exposure to infrared.

The acid to be generated is preferably a strong acid having a pKa of 2 or less, such as sulfonic acid or hydrochloric acid. The acid generated from the acid generator enables the acid color developing agent to discolor.

Specifically, as the acid generator, from the viewpoint of sensitivity and stability, an onium salt compound is preferable.

Specific examples of onium salts suitable as the acid generator include the compounds described in paragraphs "0121" to "0124" of WO2016/047392A.

Particularly, sulfonate, carboxylate, BPh₄⁻, BF₄⁻, PF₆⁻, ClO₄⁻ of triarylsulfonium or diaryliodonium, and the like are preferable. Ph represents a phenyl group.

One kind of acid generator may be used alone, or two or more kinds of acid generators may be used in combination.

In a case where the outermost layer contains an acid generator, the content of the acid generator with respect to the total mass of the outermost layer is preferably 0.5% by mass to 30% by mass, and more preferably 1% by mass to 20% by mass.

### <<Preservative>>

From the viewpoint of temporal stability, it is preferable that the outermost layer contain a preservative.

In the present disclosure, a preservative refers to a component having a function of preventing the occurrence and growth of microorganisms, particularly bacteria and fungi (for example, mold).

As the preservative, a known preservative can be used. For example, any of inorganic and organic preservatives may be used. Examples of the inorganic preservatives include compounds containing heavy metal ions, silver ions, and the like. Examples of the organic preservatives include a quaternary ammonium salt (for example, tetrabutylammonium chloride, cetylpyridinium chloride, benzyltrimethylammonium chloride, or the like), a phenol derivative (for example, phenol, cresol, butylphenol, xylenol, bisphenol, or the like), a phenoxyether derivative (for example, phenoxyethanol or the like), a heterocyclic compound (for example, benzotriazole, PROXEL, 1,2-benzisothiazolin-3-one, and the like), alkanediols (for example, pentylene glycol (1,2-pentanediol), isopentyl diol (for example, 3-methyl-1,3-butanediol), hexanediol (for example, 1,2-hexanediol or the like), caprylyl glycol (for example, 1,2-octanediol) or the like), acid amides, carbamic acid, carbamates, amidine guanidines, pyridines (for example, sodium pyridinethion-1-oxide and the like), diazines, triazines, pyrrole imidazoles, oxazole oxazines, thiazole·thiadiazines, thioureas, thiosemicarbazides, dithiocarbamates, sulfides, sulfoxides, sulfones, sulfamides, antibiotics (penicillin, tetracycline, and the like), sodium dehydroacetate, sodium benzoate, p-hydroxybenzoic acid ethyl esters, and salts of these.

One kind of preservative may be used alone, or two or more kinds of preservatives may be used in combination.

In a case where the outermost layer contains a preservative, the content of the preservative with respect to the total mass of the outermost layer is preferably 0.0001% by mass to 10% by mass, more preferably 0.0005% by mass to 2.0% by mass, and particularly preferably 0.001% by mass to 0.5% by mass.

The outermost layer may contain known additives such as an oil sensitizing agent, an inorganic lamellar compound, and a surfactant, in addition to the components described above.

In addition, it is preferable that the outermost layer contain a resin having a fluorine atom, which will be described later.

Furthermore, it is preferable that the image-recording layer or the outermost layer contain a fluorohydrocarbon group-containing copolymer which will be described later. It is particularly preferable that the outermost layer contain a fluorohydrocarbon group-containing copolymer which will be described later.

The preferred aspect of the resin having a fluorine atom used in the outermost layer is the same as the preferred aspect of the resin having a fluorine atom used in the image-recording layer.

The outermost layer is formed by coating by a known method and drying.

The coating amount of the outermost layer (solid content) is preferably 0.01 g/m² to 10 g/m², more preferably 0.02 g/m² to 3 g/m², and particularly preferably 0.05 g/m² to 2.0 g/m².

The film thickness of the outermost layer is preferably 0.1 µm to 5.0 µm, and more preferably 0.3 µm to 4.0 µm.

The film thickness of the outermost layer is preferably 0.1 times to 5.0 times the film thickness of the image-recording layer that will be described later, and more preferably 0.2 times to 3.0 times the film thickness of the image-recording layer that will be described later.

The outermost layer may contain known additives such as a plasticizer for imparting flexibility, a surfactant for improving coating properties, and inorganic particles for controlling surface sliding properties.

### <Image-recording layer>

The lithographic printing plate precursor according to the present disclosure has a support, an image-recording layer, and an outermost layer in this order.

The image-recording layer used in the present disclosure is preferably a negative tone image-recording layer and more preferably a water-soluble or water-dispersible negative tone image-recording layer.

In the lithographic printing plate precursor according to the present disclosure, from the viewpoint of on-press developability, a non-exposed portion of the image-recording layer is preferably removable by at least any of dampening water or printing ink.

The image-recording layer preferably contains an infrared absorber, a polymerization initiator, and a polymerizable compound, and more preferably contains an infrared absorber, an electron-accepting polymerization initiator, an electron-donating polymerization initiator, and a polymerizable compound.

Hereinafter, each of the components to be incorporated into the image-recording layer will be specifically described.

### [Infrared absorber]

It is preferable that the image-recording layer in the present disclosure contain an infrared absorber.

The infrared absorber is not particularly limited, and examples thereof include pigments and dyes.

As the dye that is used as the infrared absorber, it is possible to use commercially available dyes and known dyes described in publications, for example, "Dye Handbooks" (edited by the Society of Synthetic Organic Chemistry, Japan, 1970). Specific examples thereof include dyes such as an azo dye, a metal complex azo dye, a pyrazolone azo dye, a naphthoquinone dye, an anthraquinone dye, a phthalocyanine dye, a carbonium dye, a quinoneimine dye, a methine dye, a cyanine dye, a squarylium colorant, a pyrylium salt, and a metal thiolate complex.

Among these dyes, for example, a cyanine dye, a squarylium colorant, a pyrylium salt, a nickel thiolate complex, and an indolenine cyanine dye are preferable, and a cyanine dye or an indolenine cyanine dye is more preferable. Among these, a cyanine dye is particularly preferable.

The aforementioned infrared absorber is preferably a cationic polymethine colorant having an oxygen atom, a nitrogen atom, or a halogen atom at the meso-position. Preferred examples of the cationic polymethine colorant include a cyanine dye, a pyrylium colorant, a thiopyrylium colorant, an azulenium colorant, and the like. From the viewpoint of ease of availability, solubility in a solvent during an introduction reaction, and the like, a cyanine dye is preferable.

Specific examples of the cyanine dye include the compounds described in paragraphs "0017" to "0019" of JP2001-133969A and the compounds described in paragraphs "0016" to "0021" of JP2002-023360A and paragraphs "0012" to "0037" of JP2002-040638A. As the cyanine dye, for example, the compounds described in paragraphs "0034" to "0041" of JP2002-278057A and paragraphs "0080" to "0086" of JP2008-195018A are preferable, and the compounds described in paragraphs "0035" to "0043" of JP2007-90850A and the compounds described in paragraphs "0105" to "0113" of JP2012-206495A are particularly preferable.

Furthermore, the compounds described in paragraphs "0008" and "0009" of JP1993-5005A (JP-H5-5005A) and paragraphs "0022" to "0025" of JP2001-222101A can also be preferably used. As pigments, the compounds described in paragraphs "0072" and" 0076" of JP2008-195018A are preferable.

The infrared absorber preferably includes a compound represented by Formula 1.

In Formula 1, R₁ and R₂ each independently represent a hydrogen atom or an alkyl group, R₁ and R₂ may be linked to each other to form a ring, R₃ to R₆ each independently represent a hydrogen atom or an alkyl group, R₇ and R₈ each independently represent an alkyl group or an aryl group, Y₁ and Y₂ each independently represent an oxygen atom, a sulfur atom, -NR₀-, or a dialkylmethylene group, R₀ represents a hydrogen atom, an alkyl group, or an aryl group, Ar₁ and Ar₂ each independently represent a group forming a benzene ring or a naphthalene ring which may have a group represented by Formula 2 that will be described later, A₁ represents -NR₉R₁₀, -X₁-L₁, or a group represented by Formula 2 that will be described later, R₉ and R₁₀ each independently represent an alkyl group, an aryl group, an alkoxycarbonyl group, or an arylsulfonyl group, X₁ represents an oxygen atom or a sulfur atom, L₁ represents a hydrocarbon group, a heteroaryl group, or a group that undergoes bond cleavage from X₁ by heat or exposure to infrared, Za represents a counterion that neutralizes charge, and at least one of Ar₁ or Ar₂ has a group represented by Formula 2.

-X Formula 2

In Formula 2, X represents a halogen atom, -C(=O)-X₂-R₁₁, -C(=O)-NR₁₂R₁₃, -O-C(=O)-R₁₄, -CN, -SO₂NR₁₅R₁₆, or a perfluoroalkyl group, X₂ represents a single bond or an oxygen atom, R₁₁ and R₁₄ each independently represent an alkyl group or an aryl group, and R₁₂, R₁₃, R₁₅, and R₁₆ each independently represent a hydrogen atom, an alkyl group, or an aryl group.

Ar₁ and Ar₂ each independently represent a group forming a benzene ring or a naphthalene ring. The benzene ring and the naphthalene ring may have a substituent other than -X. Examples of the substituent include an alkyl group, an alkoxy group, an aryloxy group, an amino group, an alkylthio group, an arylthio group, a carboxy group, a carboxylate group, a sulfo group, a sulfonate group, groups obtained by combining these, and the like. Among these, an alkyl group is preferable.

In Formula 1, at least one of Ar₁ or Ar₂ has a group represented by Formula 2. From the viewpoint of printing durability, visibility, and temporal storage stability of a coating liquid used for forming the image-recording layer (temporal stability), it is preferable that both of Ar₁ and Ar₂ have a group represented by Formula 2.

X in Formula 2 represents a halogen atom, -C(=O)-X₂-R₁₁, -C(=O)-NR₁₂R₁₃, -O-C(=O)-R₁₄, -CN, -SO₂NR₁₅R₁₆, or a perfluoroalkyl group. From the viewpoint of printing durability, visibility, and temporal stability, X is preferably a halogen atom, -C(=O)-X₂-R₁₁, -C(=O)-NR₁₂R₁₃, -O-C(=O)-R₁₄, CN, or -SO₂NR₁₅R₁₆, preferably a halogen atom, -C(=O)-O-R₁₁, -C(=O)-NR₁₂R₁₃, or -O-C(=O)-R₁₄, even more preferably a halogen atom, -C(=O)-O-R₁₁ or -O-C(=O)-R₁₄, still more preferable a fluorine atom, a chlorine atom, a bromine atom, or -C(=O)OR₁₇, and particularly preferably a chlorine atom or a bromine atom.

X substituting Ar₁, X substituting Ar₂, and X of A₁ may be the same group or different groups. From the viewpoint of printing durability, visibility, and temporal stability, it is preferable that X substituting Ar₁ and X substituting Ar₂ be the same group.

X₂ represents a single bond or an oxygen atom, and is preferably an oxygen atom.

R¹¹ and R¹⁴ each independently represent an alkyl group or an aryl group, preferably each independently represent an alkyl group having 1 to 12 carbon atoms or an aryl group having 6 to 12 carbon atoms, and more preferably each independently represent an alkyl group having 1 to 12 carbon atoms.

R₁₂, R₁₃, R₁₅, and R₁₆ each independently represent a hydrogen atom, an alkyl group, or an aryl group, preferably each independently represent a hydrogen atom, an alkyl group having 1 to 12 carbon atoms, or an aryl group having 6 to 12 carbon atoms, more preferably each independently represent a hydrogen atom or an alkyl group having 1 to 12 carbon atoms, and even more preferably each independently represent an alkyl group having 1 to 12 carbon atoms.

R₁₇ represents an alkyl group or an aryl group, preferably represents an alkyl group having 1 to 12 carbon atoms or an aryl group having 6 to 12 carbon atoms, and more preferably represents an alkyl group having 1 to 12 carbon atoms.

A₁ represents -NR₉R₁₀, -X₁-L₁, or -X. From the viewpoint of printing durability, visibility, and temporal stability, A₁ is preferably -NR₉R₁₀ or -X₁-L₁, and more preferably -NR₁₈R₁₉ or -S-R₂₀.

Furthermore, from the viewpoint of UV printing durability, A₁ is preferably -X, more preferably a halogen atom, even more preferably a chlorine atom or a bromine atom, and particularly preferably a chlorine atom.

R₉ and R₁₀ each independently represent an alkyl group, an aryl group, an alkoxycarbonyl group, or an arylsulfonyl group, preferably each independently represent an alkyl group having 1 to 12 carbon atoms or an aryl group having 6 to 12 carbon atoms, and more preferably each independently represent an alkyl group having 1 to 12 carbon atoms.

X₁ represents an oxygen atom or a sulfur atom. In a case where L₁ is a hydrocarbon group or a heteroaryl group, X₁ is preferably a sulfur atom. L₁ is preferably a group that undergoes bond cleavage from X₁ by heat or exposure to infrared.

L₁ represents a hydrocarbon group, a heteroaryl group, or a group that undergoes bond cleavage from X₁ by heat or exposure to infrared. From the viewpoint of printing durability, L₁ is preferably a hydrocarbon group or a heteroaryl group, more preferably an aryl group or a heteroaryl group, and even more preferably a heteroaryl group.

Furthermore, from the viewpoint of visibility and suppressing fading over time, L₁ is preferably a group that undergoes bond cleavage from X₁ by heat or exposure to infrared.

The group that undergoes bond cleavage from X₁ by heat or exposure to infrared will be described later.

R₁₈ and R₁₉ each independently represent an aryl group, preferably each independently represent an aryl group having 6 to 20 carbon atoms, and more preferably each independently represent a phenyl group.

R₂₀ represents a hydrocarbon group or a heteroaryl group, preferably represents an aryl group or a heteroaryl group, and more preferably represents a heteroaryl group.

Preferred examples of the heteroaryl group represented by L₁ and R₂₀ include the following groups.

The alkyl group represented by R₁ to R₁₀ and R₀ is preferably an alkyl group having 1 to 30 carbon atoms, more preferably an alkyl group having 1 to 15 carbon atoms, and even more preferably an alkyl group having 1 to 10 carbon atoms. The alkyl group may be linear or branched, or may have a ring structure.

Specific examples of the alkyl group include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a hexadecyl group, an octadecyl group, an eicosyl group, an isopropyl group, an isobutyl group, an s-butyl group, a t-butyl group, an isopentyl group, a neopentyl group, a 1-methylbutyl group, an isohexyl group, a 2-ethylhexyl group, a 2-methylhexyl group, a cyclohexyl group, a cyclopentyl group, and a 2-norbornyl group.

Among these alkyl groups, a methyl group, an ethyl group, a propyl group, or a butyl group is particularly preferable.

The above alkyl group may have a substituent. Examples of the substituent include an alkoxy group, an aryloxy group, an amino group, an alkylthio group, an arylthio group, a halogen atom, a carboxy group, a carboxylate group, a sulfo group, a sulfonate group, an alkyloxycarbonyl group, an aryloxycarbonyl group, and groups obtained by combining these, and the like.

The aryl group represented by R₉, R₁₀, R₁₈, R₁₉, and R₀ is preferably an aryl group having 6 to 30 carbon atoms, more preferably an aryl group having 6 to 20 carbon atoms, and even more preferably an aryl group having 6 to 12 carbon atoms.

The aryl group may further have a substituent. Examples of the substituent include an alkyl group, an alkoxy group, an aryloxy group, an amino group, an alkylthio group, an arylthio group, a halogen atom, a carboxy group, a carboxylate group, a sulfo group, a sulfonate group, an alkyloxycarbonyl group, an aryloxycarbonyl group, and groups obtained by combining these, and the like.

Specific examples of the aryl group include a phenyl group, a naphthyl group, a p-tolyl group, a p-chlorophenyl group, a p-fluorophenyl group, a p-methoxyphenyl group, a p-dimethylaminophenyl group, a p-methylthiophenyl group, a p-phenylthiophenyl group, and the like.

Among these aryl groups, a phenyl group, a p-methoxyphenyl group, a p-dimethylaminophenyl group, or a naphthyl group is preferable.

It is preferable that R₁ and R₂ be linked to each other to form a ring.

In a case where R₁ and R₂ are linked to each other to form a ring, the ring is preferably a 5- or a 6-membered ring and more preferably a 6-membered ring. Furthermore, the ring formed of R₁ and R₂ linked to each other is preferably a hydrocarbon ring which may have an ethylenically unsaturated bond.

Y₁ and Y₂ each independently represent an oxygen atom, a sulfur atom, -NR₀-, or a dialkylmethylene group. Among these, -NR₀- or a dialkylmethylene group is preferable, and a dialkylmethylene group is more preferable.

R₀ represents a hydrogen atom, an alkyl group, or an aryl group. R₀ is preferably an alkyl group.

It is preferable that R₇ and R₈ be the same group.

R₇ and R₈ preferably each independently represent a linear alkyl group or an alkyl group having a sulfonate group on a terminal, and more preferably each independently represent a methyl group, an ethyl group, or a butyl group having a sulfonate group on a terminal.

The countercation of the aforementioned sulfonate group may be a cation on a nitrogen atom in Formula 1 or may be an alkali metal cation or an alkaline earth metal cation.

From the viewpoint of improving water solubility of the compound represented by Formula 1, R₇ and R₈ preferably each independently represent an alkyl group having an anion structure, more preferably each independently represent an alkyl group having a carboxylate group or a sulfonate group, and even more preferably each independently represent an alkyl group having a sulfonate group on a terminal.

From the viewpoint of increasing the maximum absorption wavelength of the compound represented by Formula 1 and from the viewpoint of visibility and printing durability of the lithographic printing plate, R₇ and R₈ preferably each independently represent an alkyl group having an aromatic ring, more preferably each independently represent an alkyl group having an aromatic ring on a terminal, and particularly preferably each independently represent a 2-phenylethyl group, a 2-naphthalenylethyl group, or a 2-(9-anthracenyl)ethyl group.

R₃ to R₆ each independently represent a hydrogen atom or an alkyl group, and preferably each independently represent a hydrogen atom.

From the viewpoint of visibility and UV printing durability, the compound represented by Formula 1 preferably has one or more halogen atoms, more preferably has one or more halogen atoms in at least one group selected from the group consisting of A₁, Ar₁, and Ar₂, and particularly preferably has one or more halogen atoms in each of A₁, Ar₁, and Ar₂.

Furthermore, from the viewpoint of visibility and UV printing durability, the compound represented by Formula 1 more preferably has two or more halogen atoms, even more preferably has three or more halogen atoms, and particularly preferably has three or more and six or less halogen atoms.

Preferred examples of the aforementioned halogen atoms include a chlorine atom and a bromine atom.

From the viewpoint of temporal stability, GLV suitability, and UV printing durability, the compound represented by Formula 1 preferably has halogen atoms in at least one of Ar₁ or Ar₂, more preferably has chlorine atoms or bromine atoms in at least one of Ar₁ or Ar₂, even more preferably has bromine atoms in at least one of Ar₁ or Ar₂, and particularly preferably has bromine atoms in both of Ar₁ and Ar₂.

Za represents a counterion that neutralizes charge. In a case where Za represents anionic species, examples thereof include a sulfonate ion, a carboxylate ion, a tetrafluoroborate ion, a hexafluorophosphate ion, a perchlorate ion, a sulfonamide anion, a sulfonimide anion, and the like. In a case where Za represents cationic species, an alkali metal ion, an alkaline earth metal ion, an ammonium ion, a pyridinium ion, or a sulfonium ion is preferable, a sodium ion, a potassium ion, an ammonium ion, a pyridinium ion, or a sulfonium ion is more preferable, a sodium ion, a potassium ion, or an ammonium ion is even more preferable, and a sodium ion, a potassium ion, or a trialkylammonium ion is particularly preferable.

As Za, among the above, from the viewpoint of printing durability and visibility, an organic anion having a carbon atom is preferable, a sulfonate ion, a carboxylate ion, a sulfonamide anion, or a sulfonimide anion is more preferable, a sulfonamide anion or a sulfonimide anion is even more preferable, and a sulfonimide anion is particularly preferable.

R₁ to R₈, R₀, A₁, Ar₁, Ar₂, Y₁, and Y₂ may have an anion structure or a cation structure. In a case where all of R₁ to R₈, R₀, A₁, Ar₁, Ar₂, Y₁, and Y₂ represent a group having neutral charge, Za represents a monovalent counteranion. However, for example, in a case where two or more among R₁ to R₈, R₀, A₁, Ar₁, Ar₂, Y₁, and Y₂ have an anion structure, Za can be a countercation.

In Formula 1, in a case where portions other than Za have neutral charge, Formula 1 may not have Za.

As the sulfonamide anion, an aryl sulfonamide anion is preferable.

As the sulfonimide anion, a bisaryl sulfonimide anion is preferable.

Specific examples of the sulfonamide anion or the sulfonimide anion will be shown below, but the present disclosure is not limited thereto. In the following specific examples, Ph represents a phenyl group, Me represents a methyl group, and Et represents an ethyl group.

From the viewpoint of visibility, the group that undergoes bond cleavage from X₁ by heat or exposure to infrared is preferably a group represented by any of Formulas (1-1) to (1-7), and more preferably a group represented by any of Formulas (1-1) to (1-3).

In Formulas (1-1) to (1-7), ● represents a bonding site with X₁ in Formula 1, R¹⁰ each independently represent a hydrogen atom, an alkyl group, an alkenyl group, an aryl group, -OR¹⁴, -NR¹⁵R¹⁶, or -SR¹⁷, R¹¹ each independently represent a hydrogen atom, an alkyl group, or an aryl group, R¹² represents an aryl group, -OR¹⁴, -NR¹⁵R¹⁶, -SR¹⁷, -C(=O)R¹⁸, -OC(=O)R¹⁸, or a halogen atom, R¹³ represents an aryl group, an alkenyl group, an alkoxy group, or an onium group, R¹⁴ to R¹⁷ each independently represent a hydrogen atom, an alkyl group, or an aryl group, R¹⁸ each independently represent an alkyl group, an aryl group, -OR¹⁴, -NR¹⁵R¹⁶, or -SR¹⁷, and Z¹ represents a counterion that neutralizes charge.

In a case where R¹⁰, R¹¹, and R¹⁴ to R¹⁸ each represent an alkyl group, preferred aspects of the alkyl group are the same as preferred aspects of the alkyl group represented by R² to R⁹ and R⁰.

The number of carbon atoms in the alkenyl group represented by R¹⁰ and R¹³ is preferably 1 to 30, more preferably 1 to 15, and even more preferably 1 to 10.

In a case where R¹⁰ to R¹⁸ each represent an aryl group, preferred aspects of the aryl group are the same as preferred aspects of the aryl group represented by R⁰.

From the viewpoint of visibility, R¹⁰ in Formula (1-1) is preferably an alkyl group, an alkenyl group, an aryl group, -OR¹⁴, -NR¹⁵R¹⁶, or -SR¹⁷, more preferably an alkyl group, -OR¹⁴, -NR¹⁵R¹⁶, or -SR¹⁷, even more preferably an alkyl group or -OR¹⁴, and particularly preferably -OR¹⁴.

In a case where R¹⁰ in Formula (1-1) is an alkyl group, the alkyl group is preferably an alkyl group having an arylthio group or an alkyloxycarbonyl group at the α-position.

In a case where R¹⁰ in Formula (1-1) represents -OR¹⁴, R¹⁴ is preferably an alkyl group, more preferably an alkyl group having 1 to 8 carbon atoms, even more preferably an isopropyl group or a t-butyl group, and particularly preferably a t-butyl group.

From the viewpoint of visibility, R¹¹ in Formula (1-2) is preferably a hydrogen atom.

Furthermore, from the viewpoint of visibility, R¹² in Formula (1-2) is preferably -C(=O)OR¹⁴, -OC(=O)OR¹⁴, or a halogen atom, and more preferably -C(=O)OR¹⁴ or -OC(=O)OR¹⁴. In a case where R¹² in Formula (1-2) is -C(=O)OR¹⁴ or -OC(=O)OR¹⁴, R¹⁴ is preferably an alkyl group.

From the viewpoint of visibility, R¹¹ in Formula (1-3) preferably each independently represent a hydrogen atom or an alkyl group. It is more preferable that at least one of R¹¹'s in Formula (1-3) be an alkyl group.

The alkyl group represented by R¹¹ is preferably an alkyl group having 1 to 10 carbon atoms, and more preferably an alkyl group having 3 to 10 carbon atoms.

Furthermore, the alkyl group represented by R¹¹ is preferably an alkyl group having a branch or a cycloalkyl group, more preferably a secondary or tertiary alkyl group or a cycloalkyl group, and even more preferably an isopropyl group, a cyclopentyl group, a cyclohexyl group, or a t-butyl group.

From the viewpoint of visibility, R¹³ in Formula (1-3) is preferably an aryl group, an alkoxy group, or an onium group, more preferably a p-dimethylaminophenyl group or a pyridinium group, and even more preferably a pyridinium group.

Examples of the onium group represented by R¹³ include a pyridinium group, an ammonium group, a sulfonium group, and the like. The onium group may have a substituent. Examples of the substituent include an alkyl group, an alkoxy group, an aryloxy group, an amino group, an alkylthio group, an arylthio group, a halogen atom, a carboxy group, a sulfo group, an alkyloxycarbonyl group, an aryloxycarbonyl group, groups obtained by combining these, and the like. Among these, an alkyl group, an aryl group, and groups obtained by combining these are preferable.

Among these, a pyridinium group is preferable, a N-alkyl-3-pyridinium group, a N-benzyl-3-pyridinium group, a N-(alkoxypolyalkyleneoxyalkyl)-3-pyridinium group, a N-alkoxycarbonylmethyl-3-pyridinium group, a N-alkyl-4-pyridinium group, a N-benzyl-4-pyridinium group, a N-(alkoxypolyalkyleneoxyalkyl)-4-pyridinium group, a N-alkoxycarbonylmethyl-4-pyridinium group, or a N-alkyl-3,5-dimethyl-4-pyridinium group is more preferable, a N-alkyl-3-pyridinium group or a N-alkyl-4-pyridinium group is even more preferable, a N-methyl-3-pyridinium group, a N-octyl-3-pyridinium group, a N-methyl-4-pyridinium group, or a N-octyl-4-pyridinium group is particularly preferable, and a N-octyl-3-pyridinium group or a N-octyl-4-pyridinium group is most preferable.

In a case where R¹³ is a pyridinium group, examples of the counteranion include a sulfonate ion, a carboxylate ion, a tetrafluoroborate ion, a hexafluorophosphate ion, a p-toluenesulfonate ion, a perchlorate ion, and the like. Among these, a p-toluenesulfonate ion or a hexafluorophosphate ion is preferable.

From the viewpoint of visibility, R¹⁰ in Formula (1-4) is preferably an alkyl group or an aryl group. It is more preferable that one of two R¹⁰'s be an alkyl group and the other be an aryl group.

From the viewpoint of visibility, R¹⁰ in Formula (1-5) is preferably an alkyl group or an aryl group, more preferably an aryl group, and even more preferably a p-methylphenyl group.

From the viewpoint of visibility, R¹⁰ in Formula (1-6) preferably each independently represent an alkyl group or an aryl group, and more preferably each independently represent a methyl group or a phenyl group.

From the viewpoint of visibility, Z¹ in Formula (1-7) may be a counterion that neutralizes charge, and may be included in Za in the entirety of the compound.

Z¹ is preferably a sulfonate ion, a carboxylate ion, a tetrafluoroborate ion, a hexafluorophosphate ion, a p-toluenesulfonate ion, or a perchlorate ion, and more preferably a p-toluenesulfonate ion or a hexafluorophosphate ion.

The group that undergoes bond cleavage from X₁ by heat or exposure to infrared is particularly preferably a group represented by Formula (1-8).

In Formula (1-8), ● represents a bonding site with X₁ in Formula 1, R¹⁹ and R²⁰ each independently represent an alkyl group, and Za' represents a counterion that neutralizes charge.

In Formula (1-8), the bonding position of a pyridinium ring and a hydrocarbon group having R²⁰ is preferably the 3-position or 4-position of the pyridinium ring, and more preferably the 4-position of the pyridinium ring.

The alkyl group represented by R¹⁹ and R²⁰ may be linear or branched, or may have a ring structure.

Furthermore, the above alkyl group may have a substituent, and preferred examples of the substituent include an alkoxy group and a terminal alkoxypolyalkyleneoxy group.

R¹⁹ is preferably an alkyl group having 1 to 12 carbon atoms, more preferably a linear alkyl group having 1 to 12 carbon atoms, even more preferably a linear alkyl group having 1 to 8 carbon atoms, and particularly preferably a methyl group or a n-octyl group.

R²⁰ is preferably an alkyl group having 1 to 8 carbon atoms, more preferably a branched alkyl group having 3 to 8 carbon atoms, even more preferably an isopropyl group or a t-butyl group, and particularly preferably an isopropyl group.

Za' may be a counterion that neutralizes charge, and may be included in Za in the entirety of the compound.

Za' is preferably a sulfonate ion, a carboxylate ion, a tetrafluoroborate ion, a hexafluorophosphate ion, a p-toluenesulfonate ion, or a perchlorate ion, and more preferably a p-toluenesulfonate ion or a hexafluorophosphate ion.

Preferred specific examples of the compound represented by Formula 1 below include mother nucleus structures A-1 to A-54, counteranions B-1 to B-10, and countercations C-1 to C-3. However, the present disclosure is not limited to these. Specific examples of the compound represented by Formula 1 include compounds that are obtained by combining one of the mother nucleus structures A-1 to A-9, A-11 to A-20, and A-22 to A-54 and one of the counteranions B-1 to B-10 and compounds that are obtained by combining one of the mother nucleus structures A-10 and A-21 and one of the countercations C-1 to C-3.

As the compound represented by Formula 1, the following compounds can also be suitably used. TsO⁻ represents a tosylate anion.

The method of preparing the compound represented by Formula 1 is not particularly limited. The compound represented by Formula 1 can be prepared with reference to known methods of preparing a cyanine dye. In addition, the method described in WO2016/027886A can also be suitably used.

From the viewpoint of printing durability and visibility, the energy level of the highest occupied molecular orbital (HOMO) of the infrared absorber is preferably -5.250 eV or less, more preferably -5.30 eV or less, even more preferably -5.80 eV or more and -5.35 eV or less, and particularly preferably -5.65 eV or more and -5.40 eV or less.

In the present disclosure, the energy of molecular orbital (MO) such as highest occupied molecular orbital (HOMO) and the lowest unoccupied molecular orbital (LUMO) is calculated by the following methods.

First, free counterions in the compound as a calculation object are excluded from the calculation object. For example, for a cationic one electron-accepting polymerization initiator and a cationic infrared absorber, counteranions are excluded from the calculation object, and for an anionic one electron-donating polymerization initiator, countercations are excluded from the calculation object. "Free" mentioned herein means that the compound as an object and the counterions thereof are not covalently linked to each other.

The structural optimization is carried out by DFT (B3LYP/6-31G(d)) using quantum chemical calculation software Gaussian 16.

The MO energy is calculated by DFT (B3LYP/6-31+G(d,p)/PCM (solvent = methanol)) with quantum chemical calculation software Gaussian16 by using the optimum structure obtained by the structural optimization. For an iodine-containing compound, the MO energy is calculated under the condition of DFT (B3LYP/DGDZVP/PCM (solvent = methanol)).

The optimum structure mentioned herein means a structure in which the total energy obtained by DFT calculation is the most stable. The most stable structure is found by repeating the structural optimization as necessary.

By the following formula, the MO energy Ebare (unit: hartree) obtained by the above MO energy calculation is converted into Escaled (unit: eV) used as the values of HOMO and LUMO in the present disclosure. $Escaled = 0.823168 \times 27.2114 \times Ebare - 1.07634$ $Escaled = 0.820139 \times 27.2114 \times Ebare - 1.086039$

27.2114 is simply a coefficient for converting hartree into eV, and 0.823168 and -1.07634 used for calculating HOMO and 0.820139 and -1.086039 used for calculating LUMO are adjustment coefficients. These are determined such that the calculated values of HOMO and LUMO of the compound as a calculation object match the measured values.

One kind of infrared absorber may be used alone, or two or more kinds of infrared absorbers may be used in combination.

In addition, as the infrared absorber, a pigment and a dye may be used in combination.

The content of the infrared absorber with respect to the total mass of the image-recording layer is preferably 0.1% by mass to 10.0% by mass, and more preferably 0.5% by mass to 5.0% by mass.

### [Polymerization initiator]

It is preferable that the image-recording layer in the lithographic printing plate precursor according to the present disclosure contain a polymerization initiator.

The polymerization initiator preferably includes an electron-accepting polymerization initiator, and more preferably includes an electron-accepting polymerization initiator and an electron-donating polymerization initiator.

### «Electron-donating polymerization initiator (polymerization aid)»

It is preferable that the image-recording layer in the present disclosure contain an electron-donating polymerization initiator (also called "polymerization aid") as a polymerization initiator.

The electron-donating polymerization initiator is a compound which donates one electron by intermolecular electron migration to an orbit of an infrared absorber that has lost one electron in a case where electrons of the infrared absorber are excited or perform intramolecular migration by exposure to infrared, and thus generates polymerization initiation species such as radicals.

The electron-donating polymerization initiator is preferably an electron-donating radical polymerization initiator.

From the viewpoint of printing durability, the image-recording layer preferably contains a borate compound.

From the viewpoint of printing durability and visibility, the borate compound is preferably a tetraaryl borate compound or a monoalkyl triaryl borate compound, and more preferably a tetraaryl borate compound.

From the viewpoint of printing durability and visibility, the borate compound is preferably a tetraaryl borate compound having one or more electron-donating groups, and more preferably a tetraaryl borate compound having one electron-donating group in each aryl group.

From the viewpoint of printing durability and visibility, the aforementioned electron-donating group is preferably an alkyl group or an alkoxy group, and more preferably an alkoxy group.

A countercation that the borate compound has is not particularly limited, but is preferably an alkali metal ion or a tetraalkyl ammonium ion and more preferably a sodium ion, a potassium ion, or a tetrabutylammonium ion.

The countercation that the borate compound has may also be a cationic polymethine colorant in the infrared absorber described in the present specification. For example, the aforementioned borate compound may be used as the countercation of the cyanine dye.

Specifically, preferred examples of the borate compound include sodium tetraphenyl borate.

Specifically, as the electron-donating polymerization initiator, for example, the following B-1 to B-9 are preferable. It goes without saying that the present disclosure is not limited thereto. In the following chemical formulas, Ph represents a phenyl group, and Bu represents a n-butyl group.

From the viewpoint of improving sensitivity, the energy level of the highest occupied molecular orbital (HOMO) of the electron-donating polymerization initiator is preferably -6.00 eV or more, more preferably -5.95 eV or more, even more preferably -5.93 eV or more, and particularly preferably more than -5.90 eV

The upper limit of the energy level of HOMO is preferably -5.00 eV or less, and more preferably -5.40 eV or less.

Only one kind of electron-donating polymerization initiator may be used alone, or more kinds of electron-donating polymerization initiators may be used in combination.

From the viewpoint of sensitivity and printing durability, the content of the electron-donating polymerization initiator with respect to the total mass of the image-recording layer is preferably 0.01% by mass to 30% by mass, more preferably 0.05% by mass to 25% by mass, and even more preferably 0.1% by mass to 20% by mass.

From the viewpoint of UV printing durability, the content of the electron-donating polymerization initiator in the image-recording layer is preferably higher than the content of the infrared absorber, more preferably 1.1 to 5 times the content of the infrared absorber, and particularly preferably 1.5 to 3 times the content of the infrared absorber.

In the present disclosure, the polymerization initiator may be a compound in the form of conjugate salt of an electron-donating polymerization initiator and an electron-accepting polymerization initiator.

For example, in the present disclosure, the polymerization initiator is preferably a compound in the form of a conjugate salt of an anion in the electron-donating polymerization initiator and a cation in the electron-accepting polymerization initiator, more preferably a compound in the form of a conjugate salt of an onium cation and a borate anion, even more preferably a compound in the form of a conjugate salt of an iodonium cation or sulfonium cation and a borate anion, and particularly preferably a compound in the form of a conjugate salt of a diaryliodonium cation or a triarylsulfonium cation and a tetraarylborate anion.

Preferred aspects of the anion in the electron-donating polymerization initiator and the cation in the electron-accepting polymerization initiator are the same as the preferred aspects of the anion in the aforementioned electron-donating polymerization initiator and the cation in the aforementioned electron-accepting polymerization initiator.

In a case where the image-recording layer contains an anion as an electron-donating polymerization initiator and a cation as an electron-accepting polymerization initiator (that is, in a case where the image-recording layer contains a compound in the form of a conjugate salt described above), the image-recording layer is regarded as containing an electron-accepting polymerization initiator and an electron-donating polymerization initiator.

The compound in the form of a conjugate salt of an electron-donating polymerization initiator and an electron-accepting polymerization initiator may be used as an electron-donating polymerization initiator or an electron-accepting polymerization initiator.

The compound in the form of a conjugate salt of an electron-donating polymerization initiator and an electron-accepting polymerization initiator may be used in combination with the aforementioned electron-donating polymerization initiator or used in combination with the aforementioned electron-accepting polymerization initiator.

### «Relationship between infrared absorber and electron-donating polymerization initiator»

In the image-recording layer of the present disclosure, from the viewpoint of sensitivity improvement and printing durability, the energy level of HOMO of the infrared absorber - the energy level of HOMO of the electron-donating polymerization initiator is preferably 0.70 eV or less, more preferably 0.60 eV or less, even more preferably 0.55 eV or less, and particularly preferably 0.50 eV to -0.10 eV

The negative sign means that the energy level of HOMO of the electron-donating polymerization initiator is higher than the energy level of HOMO of the infrared absorber.

### «Electron-accepting polymerization initiator»

It is preferable that the image-recording layer in the present disclosure contain an electron-accepting polymerization initiator as a polymerization initiator.

The electron-accepting polymerization initiator is a compound which accepts an electron by intermolecular electron migration in a case where electrons of an infrared absorber are excited by exposure to infrared, and generates a polymerization initiation species such as radicals.

The electron-accepting polymerization initiator is a compound that generates a polymerization initiation species such as a radical or a cation by either or both of light energy and heat energy, and can be appropriately selected from known thermal polymerization initiators, compounds having a bond that requires low bond dissociation energy, photopolymerization initiators, and the like.

The electron-accepting polymerization initiator is preferably a radical polymerization initiator and more preferably an onium salt compound.

In addition, as the electron-accepting polymerization initiator, an infrared-sensitive polymerization initiator is preferable.

From the viewpoint of sensitivity improvement and UV printing durability, the electron-accepting polymerization initiator is preferably an iodonium salt compound or a compound having an alkyl halide group, and more preferably a compound having an alkyl halide group.

In addition, from the viewpoint of sensitivity improvement and UV printing durability, the compound having an alkyl halide group is preferably a compound having a perhalogenoalkylsulfonyl group, more preferably a compound having a trihalogenomethylsulfonyl group, and particularly preferably a compound having a tribromomethylsulfonyl group.

Among the above electron-accepting polymerization initiators, from the viewpoint of curing properties, an oxime ester compound and an onium salt compound are preferable. Particularly, from the viewpoint of printing durability, an iodonium salt compound, a sulfonium salt compound, or an azinium salt compound is preferable, an iodonium salt compound or a sulfonium salt compound is more preferable, and an iodonium salt compound is particularly preferable.

Specific examples of these compounds will be shown below, but the present disclosure is not limited thereto.

As the iodonium salt compound, for example, a diaryliodonium salt compound is preferable. Particularly, a diphenyl iodonium salt compound substituted with an electron-donating group such as an alkyl group or an alkoxyl group is more preferable. Furthermore, an asymmetric diphenyl iodonium salt compound is preferable. Specific examples thereof include diphenyliodonium=hexafluorophosphate, 4-methoxyphenyl-4-(2-methylpropyl)phenyliodonium=hexafluorophosphate, 4-(2-methylpropyl)phenyl-p-tolyliodonium=hexafluorophosphate, 4-hexyloxyphenyl-2,4,6-trimethoxyphenyl iodonium=hexafluorophosphate, 4-hexyloxyphenyl-2,4-diethoxyphenyl iodonium=tetrafluoroborate, 4-octyloxyphenyl-2,4,6-trimethoxyphenyl iodonium=1-perfluorobutane sulfonate, 4-octyloxyphenyl-2,4,6-trimethoxyphenyliodonium=hexafluorophosphate, and bis(4-t-butylphenyl)iodonium=hexafluorophosphate.

Examples of counteranions of the iodonium salt compound and the sulfonium salt compound include a sulfonate anion, a carboxylate anion, a tetrafluoroborate anion, a hexafluorophosphate anion, a p-toluene sulfonate anion, a tosylate anion, a sulfonamide anion, and a sulfonimide anion.

Among the above, a sulfonamide anion or a sulfonimide anion is preferable, and a sulfonimide anion is more preferable.

As the sulfonamide anion, an aryl sulfonamide anion is preferable.

As the sulfonimide anion, a bisaryl sulfonimide anion is preferable.

Specific examples of the sulfonamide anion and the sulfonimide anion include those described in WO2019/013268A.

From the viewpoint of temporal visibility after exposure, developability, and UV printing durability of the lithographic printing plate to be obtained, the aforementioned electron-accepting polymerization initiator preferably includes a compound represented by Formula (II) or Formula (III), and particularly preferably includes a compound represented by Formula (II).

In Formula (II) and Formula (III), X^{A} represents a halogen atom, and R^{A}, R^{A1}, and R^{A2} each independently represent a monovalent hydrocarbon group having 1 to 20 carbon atoms.

R^{A} in Formula (II) is preferably an aryl group.

Examples of X^{A} in Formula (II) and Formula (III) include a fluorine atom, a chlorine atom, a bromine atom, and an iodine atom. Among these, a chlorine atom or a bromine atom is preferable because these have excellent sensitivity, and a bromine atom is particularly preferable.

R^{A}, R^{A1}, and R^{A2} in Formula (II) and Formula (III) preferably each independently represent an aryl group. Particularly, from the viewpoint of excellent balance between sensitivity and storage stability, R^{A}, R^{A1}, and R^{A2} more preferably each independently represent an aryl group substituted with an amide group.

The aforementioned electron-accepting polymerization initiator particularly preferably includes a compound represented by Formula (IV).

In Formula (IV), X^{A} represents a halogen atom, R^{A3} and R^{A4} each independently represent a hydrogen atom or a monovalent hydrocarbon group having 1 to 20 carbon atoms, and pA and qA each independently represent an integer of 1 to 5. Here, pA + qA = 2 to 6.

Specific examples of the electron-accepting polymerization initiator include compounds represented by the following formulas. However, the present disclosure is not limited thereto. In the following compounds, Et represents an ethyl group, ⁿPr represents a n-propyl group, "C₄H₉ represents a n-butyl group, cHex represents a cyclohexyl group, ⁿC₅H₁₁ represents a n-pentyl group, ^{t}C₅H₁₁ represents a t-pentyl group, Ph represents a phenyl group, ⁿC₈H₁₇ represents a n-octyl group, ^{t}Bu represents a t-butyl group, ⁿBu represents a n-butyl group, and ⁿC₁₂H₂₅ represents a n-decyl group.

From the viewpoint of improving sensitivity, the lowest unoccupied molecular orbital (LUMO) of the electron-accepting polymerization initiator is preferably -3.00 eV or less, and more preferably -3.02 eV or less.

The lower limit of LUMO is preferably -3.80 eV or more, and more preferably -3.50 eV or more.

One kind of electron-accepting polymerization initiator may be used alone, or two or more kinds of electron-accepting polymerization initiators may be used in combination.

The content of the electron-accepting polymerization initiator with respect to the total mass of the image-recording layer is preferably 0.1% by mass to 50% by mass, more preferably 0.5% by mass to 30% by mass, and particularly preferably 0.8% by mass to 20% by mass.

### «Relationship between electron-accepting polymerization initiator and infrared absorber»

In the image-recording layer of the present disclosure, from the viewpoint of sensitivity improvement and printing durability, the energy level of LUMO of the electron-accepting polymerization initiator - the energy level of LUMO of the infrared absorber is preferably 0.45 eV or more, more preferably 0.58 eV or more, and particularly preferably 0.62 eV or more. Furthermore, the energy level of LUMO of the electron-accepting polymerization initiator - the energy level of LUMO of the infrared absorber is preferably 1.00 eV or less, more preferably 0.95 eV or less, and particularly preferably 0.70 eV or less.

The negative sign means that the energy level of LUMO of the infrared absorber is higher than the energy level of LUMO of the electron-accepting polymerization initiator.

### [Polymerizable compound]

It is preferable that the image-recording layer in the present disclosure contain a polymerizable compound.

In the present disclosure, a polymerizable compound refers to a compound having a polymerizable group.

The polymerizable group is not particularly limited and may be a known polymerizable group. As the polymerizable group, an ethylenically unsaturated group is preferable. The polymerizable group may be a radically polymerizable group or a cationically polymerizable group. The polymerizable group is preferably a radically polymerizable group.

Examples of the radically polymerizable group include a (meth)acryloyl group, an allyl group, a vinylphenyl group, a vinyl group, and the like. From the viewpoint of reactivity, a (meth)acryloyl group is preferable.

The molecular weight of the polymerizable compound (weight-average molecular weight in a case where the polymerizable compound has molecular weight distribution) is preferably 50 or more and less than 2,500.

The polymerizable compound used in the present disclosure may be, for example, a radically polymerizable compound or a cationically polymerizable compound. As the polymerizable compound, an addition polymerizable compound having at least one ethylenically unsaturated bond (ethylenically unsaturated compound) is preferable.

The ethylenically unsaturated compound is preferably a compound having at least one ethylenically unsaturated bond on a terminal, and more preferably a compound having two or more ethylenically unsaturated bonds on a terminal. The chemical form of the polymerizable compound is, for example, a monomer, a prepolymer which is in other words a dimer, a trimer, or an oligomer, a mixture of these, or the like.

Particularly, from the viewpoint of UV printing durability, the aforementioned polymerizable compound preferably includes a polymerizable compound having functionalities of 3 or more, more preferably includes a polymerizable compound having functionalities of 7 or more, and even more preferably includes a polymerizable compound having functionalities of 10 or more. Particularly, from the viewpoint of UV printing durability of the lithographic printing plate to be obtained, the aforementioned polymerizable compound preferably includes an ethylenically unsaturated compound having functionalities of 3 or more (preferably having functionalities of 7 or more and more preferably having functionalities of 10 or more), and more preferably includes a (meth)acrylate compound having functionalities of 3 or more (preferably having functionalities of 7 or more and more preferably having functionalities of 10 or more).

From the viewpoint of on-press developability and contamination suppressiveness, the aforementioned polymerizable compound preferably includes a polymerizable compound having functionalities of 2 or less, more preferably includes a difunctional polymerizable compound, and particularly preferably includes a difunctional (meth)acrylate compound.

From the viewpoint of printing durability, on-press developability, and contamination suppressiveness, the content of the polymerizable compound having functionalities of 2 or less (preferably a difunctional polymerizable compound) with respect to the total mass of polymerizable compounds in the image-recording layer is preferably 5% by mass to 100% by mass, more preferably 10% by mass to 100% by mass, and even more preferably 50% to 100% by mass.

### «Oligomer»

As the polymerizable compound to be incorporated into the image-recording layer, a polymerizable compound which is an oligomer (hereinafter, also simply called "oligomer") is preferable.

In the present disclosure, an oligomer represents a polymerizable compound which has a molecular weight (weight-average molecular weight in a case where the compound has molecular weight distribution) of 600 or more and 10,000 or less and at least one polymerizable group.

From the viewpoint of excellent chemical resistance and excellent UV printing durability, the molecular weight of the oligomer is preferably 1,000 or more and 5,000 or less.

Furthermore, from the viewpoint of improving UV printing durability, the number of polymerizable groups in one molecule of the oligomer is preferably 2 or more, more preferably 3 or more, even more preferably 6 or more, and particularly preferably 10 or more.

The upper limit of polymerizable groups in the oligomer is not particularly limited. The number of polymerizable groups is preferably 20 or less.

From the viewpoint of UV printing durability and on-press developability, an oligomer having 7 or more polymerizable groups and a molecular weight of 1,000 or more and 10,000 or less is preferable, and an oligomer having 7 or more and 20 or less polymerizable groups and a molecular weight of 1,000 or more and 5,000 or less is more preferable.

The oligomer may contain a polymer component which is likely to be generated in the process of manufacturing the oligomer.

From the viewpoint of UV printing durability, visibility, and on-press developability, the oligomer preferably has at least one kind of compound selected from the group consisting of a compound having a urethane bond, a compound having an ester bond, and a compound having an epoxy residue, and preferably has a compound having a urethane bond.

In the present disclosure, an epoxy residue refers to a structure formed of an epoxy group. For example, the epoxy residue means a structure similar to a structure established by the reaction between an acid group (carboxylic acid group or the like) and an epoxy group.

As the compound having a urethane bond, which is an example of the oligomer, for example, a compound having at least a group represented by Formula (Ac-1) or Formula (Ac-2) is preferable, and a compound having at least a group represented by Formula (Ac-1) is more preferable.

In Formula (Ac-1) and Formula (Ac-2), L¹ to L⁴ each independently represent a divalent hydrocarbon group having 2 to 20 carbon atoms, and the portion of the wavy line represents a bonding position with other structures.

L¹ to L⁴ preferably each independently represent an alkylene group having 2 to 20 carbon atoms, more preferably each independently represent an alkylene group having 2 to 10 carbon atoms, and even more preferably each independently represent an alkylene group having 4 to 8 carbon atoms. The alkylene group may have a branched structure or a ring structure. The alkylene group is preferably a linear alkylene group.

The portion of the wavy line in Formula (Ac-1) or Formula (Ac-2) is preferably each independently directly bonded to the portion of the wavy line in a group represented by Formula (Ae-1) or Formula (Ae-2).

In Formula (Ae-1) and Formula (Ae-2), R each independently represent an acryloyloxy group or a methacryloyloxy group, and the portion of the wavy line represents a bonding position with the portion of the wavy line in Formula (Ac-1) and Formula (Ac-2).

As the compound having a urethane bond, a compound may also be used which is prepared by obtaining polyurethane by a reaction between a polyisocyanate compound and a polyol compound and introducing a polymerizable group into the polyurethane by a polymer reaction.

For example, the compound having a urethane bond may be obtained by reacting a polyol compound having an acid group with a polyisocyanate compound to obtain a polyurethane oligomer and reacting this polyurethane oligomer with a compound having an epoxy group and a polymerizable group.

The number of polymerizable groups in the compound having an ester bond, which is an example of oligomer, is preferably 3 or more, and more preferably 6 or more.

As the compound having an epoxy residue, which is an example of oligomer, a compound containing a hydroxy group is preferable.

The number of polymerizable groups in the compound having an epoxy residue is preferably 2 to 6, and more preferably 2 or 3.

The compound having an epoxy residue can be obtained, for example, by reacting a compound having an epoxy group with an acrylic acid.

Specific examples of oligomers will be shown in the following tables, but the oligomer used in the present disclosure is not limited thereto.

As the oligomer, commercially available products may also be used. Examples thereof include UA510H, UA-306H, UA-306I, and UA-306T (manufactured by KYOEISHA CHEMICAL Co., LTD.), UV-1700B, UV-6300B, and UV7620EA (manufactured by NIHON GOSEI KAKO Co., Ltd.), U-15HA (manufactured by SHIN-NAKAMURA CHEMICAL Co., LTD.), EBECRYL450, EBECRYL657, EBECRYL885, EBECRYL800, EBECRYL3416, and EBECRYL860 (manufactured by DAICEL-ALLNEX LTD.), and the like. However, the oligomer is not limited to these.

From the viewpoint of improving chemical resistance and UV printing durability and further suppressing the occurrence of residues during on-press development, the content of the oligomer with respect to the total mass of polymerizable compounds in the image-recording layer is preferably 30% by mass to 100% by mass, more preferably 50% by mass to 100% by mass, and even more preferably 80% by mass to 100% by mass.

### «Low-molecular-weight polymerizable compound»

The polymerizable compound may further include a polymerizable compound other than the oligomer described above.

From the viewpoint of chemical resistance, the polymerizable compound other than the oligomer is preferably a low-molecular-weight polymerizable compound. The low-molecular-weight polymerizable compound may take a chemical form such as a monomer, a dimer, a trimer, or a mixture of these.

From the viewpoint of chemical resistance, the low-molecular-weight polymerizable compound is preferably at least a polymerizable compound selected from the group consisting of a polymerizable compound having three or more ethylenically unsaturated groups and a polymerizable compound having an isocyanuric ring structure.

In the present disclosure, a low-molecular-weight polymerizable compound refers to a polymerizable compound having a molecular weight (weight-average molecular weight in a case where the compound has molecular weight distribution) of 50 or more and less than 600.

From the viewpoint of excellent chemical resistance, excellent UV printing durability, and excellently suppressing the occurrence of residues during on-press development, the molecular weight of the low-molecular-weight polymerizable compound is preferably 100 or more and less than 600, more preferably 300 or more and less than 600, and even more preferably 400 or more and less than 600.

In a case where the polymerizable compound includes a low-molecular-weight polymerizable compound as the polymerizable compound other than an oligomer (total amount in a case where the polymerizable compound includes two or more kinds of low-molecular-weight polymerizable compounds), from the viewpoint of chemical resistance and UV printing durability and suppressing the occurrence of residues during on-press development, the ratio of the oligomer to the low-molecular-weight polymerizable compound (oligomer/low-molecular-weight polymerizable compound) is preferably 10/1 to 1/10, more preferably 10/1 to 3/7, and even more preferably 10/1 to 7/3, based on mass.

As the low-molecular-weight polymerizable compound, the polymerizable compounds described in paragraphs "0082" to "0086" of WO2019/013268A can also be suitably used.

### -Specific compound B2-

The low-molecular-weight polymerizable compound may include a compound having one or two ethylenically unsaturated groups (hereinafter, also called specific compound B2).

The polymerizable group in the specific compound B2 may be, for example, a cationically polymerizable group or a radically polymerizable group. From the viewpoint of reactivity, the polymerizable group is preferably a radically polymerizable group.

The polymerizable group is not particularly limited. From the viewpoint of reactivity and printing durability, the polymerizable group is preferably an ethylenically unsaturated group, more preferably at least one kind of group selected from the group consisting of a vinylphenyl group (styryl group), a vinyl ester group, a vinyl ether group, an allyl group, a (meth)acryloxy group, and a (meth)acrylamide group, even more preferably at least one kind of group selected from the group consisting of a vinylphenyl group (styryl group), a (meth)acryloxy group, and a (meth)acrylamide group, and particularly preferably a (meth)acryloxy group.

Furthermore, from the viewpoint of inhibiting the deterioration of on-press developability, the specific compound B2 is preferably a compound having two ethylenically unsaturated bonding groups (that is, a difunctional polymerizable compound).

From the viewpoint of on-press developability and printing durability, the specific compound B2 is preferably a methacrylate compound, that is, a compound having a methacryloxy group.

From the viewpoint of on-press developability, the specific compound B2 preferably has an alkyleneoxy structure or a urethane bond.

The molecular weight of the specific compound B2 (weight-average molecular weight in a case where the compound has molecular weight distribution) is preferably 50 or more and less than 1,000, more preferably 200 to 900, and even more preferably 250 to 800.

Specific examples of the specific compound B2 will be shown below. However, the specific compound B2 used in the present disclosure is not limited thereto. In Compound (2), for example, n + m = 10.

As the specific compound B2, the following commercially available products may be used. However, the specific compound B2 used in the present disclosure is not limited thereto.

Specific examples of the specific compound B2 include ethoxylated bisphenol A dimethacrylate such as BPE-80N (the above compound (1)), BPE-100, BPE-200, and BPE-500 manufactured by SHIN-NAKAMURA CHEMICAL CO., LTD., and CN104 (the above compound (1)) manufactured by Sartomer Company Inc.

Specific examples of the specific compound B2 include ethoxylated bisphenol A diacrylates such as A-BPE-10 (the above compound (2)) and A-BPE-4 manufactured by SHIN-NAKAMURA CHEMICAL CO., LTD.

Furthermore, specific examples of the specific compound B2 include difunctional methacrylate such as FST 510 manufactured by AZ Electronics.

The aforementioned "FST 510" is a product of a reaction between 1 mol of 2,2,4-trimethylhexamethylene diisocyanate and 2 mol of hydroxyethyl methacrylate, which is an 82% by mass methyl ethyl ketone solution of the above compound (3).

From the viewpoint of on-press developability and printing durability, the content of the specific compound B2 with respect to the total mass of the image-recording layer is preferably 1% by mass to 60% by mass, more preferably 5% by mass to 55% by mass, and even more preferably 5% by mass to 50% by mass.

In a case where the specific compound B2 is used, the content of the specific compound B2 with respect to the total mass of the polymerizable compounds in the image-recording layer is preferably 10% by mass to 100% by mass, more preferably 50% by mass to 100% by mass, and even more preferably 80% by mass to 100% by mass.

The details of how to use the polymerizable compound, such as the structure of the compound, whether the compound is used alone or used in combination with other compounds, and the amount of the compound to be added, can be randomly set.

Particularly, from the viewpoint of UV printing durability, the image-recording layer preferably contains two or more kinds of polymerizable compounds.

The content of the polymerizable compound (total content of polymerizable compounds in a case where the image-recording layer contains two or more kinds of polymerizable compounds) with respect to the total mass of the image-recording layer is preferably 5% by mass to 75% by mass, more preferably 10% by mass to 70% by mass, and even more preferably 15% by mass to 60% by mass.

### [Particles]

From the viewpoint of developability and UV printing durability, it is preferable that the image-recording layer in the present disclosure contain particles. The particles may be inorganic particles or organic particles.

Particularly, the image-recording layer preferably contains organic particles as particles, and more preferably contains resin particles as particles.

Known inorganic particles can be used as inorganic particles, and metal oxide particles such as silica particles and titania particles can be suitably used.

### <<Resin particles>>

Examples of the resin particles include particles containing an addition polymerization-type resin (that is, addition polymerization-type resin particles), particles containing a polyaddition-type resin (that is, polyaddition-type resin particles), particles containing a polycondensation-type resin (that is, polycondensation-type resin particles), and the like. Among these, addition polymerization-type resin particles or polyaddition-type resin particles are preferable.

From the viewpoint of enabling heat fusion, the resin particles may also be particles containing a thermoplastic resin (that is, thermoplastic resin particles).

The resin particles may be in the form of microcapsules, a microgel (that is, crosslinked resin particles), or the like.

The resin particles are preferably selected from the group consisting of thermoplastic resin particles, thermal reactive resin particles, resin particles having a polymerizable group, microcapsules encapsulating a hydrophobic compound, and a microgel (crosslinked resin particles). Among these, resin particles having a polymerizable group are preferable.

In a particularly preferred embodiment, the resin particles have at least one ethylenically unsaturated group. The presence of such resin particles brings about effects of improving the printing durability of an exposed portion and improving the on-press developability of a non-exposed portion.

As the thermoplastic resin particles, the thermoplastic resin particles described in Research Disclosure No. 33303 published in January 1992, JP1997-123387A (JP-H9-123387A), JP1997-131850A (JP-H9-131850A), JP1997-171249A (JP-H9-171249A), JP1997-171250A (JP-H9-171250A), EP931647B, and the like are preferable.

Specific examples of resins constituting the thermoplastic resin particles include homopolymers or copolymers of monomers of ethylene, styrene, vinyl chloride, methyl acrylate, ethyl acrylate, methyl methacrylate, ethyl methacrylate, vinylidene chloride, acrylonitrile, vinylcarbazole, acrylates or methacrylates having polyalkylene structures, and the like and mixtures of these.

From the viewpoint of ink receptivity and UV printing durability, the thermoplastic resin particles preferably contain a resin that has a constitutional unit formed of an aromatic vinyl compound and a nitrile group-containing constitutional unit.

The aforementioned aromatic vinyl compound may have a structure composed of an aromatic ring and a vinyl group bonded thereto. Examples of the compound include a styrene compound, a vinylnaphthalene compound, and the like. Among these, a styrene compound is preferable, and styrene is more preferable.

Examples of the styrene compound include styrene, p-methylstyrene, p-methoxystyrene, β-methylstyrene, p-methyl-β-methylstyrene, α-methylstyrene, p-methoxy-β-methylstyrene, and the like. Among these, for example, styrene is preferable.

From the viewpoint of ink receptivity, the content of the constitutional unit formed of an aromatic vinyl compound is preferably higher than the content of the nitrile group-containing constitutional unit that will be described later. The content of the constitutional unit formed of an aromatic vinyl compound with respect to the total mass of the thermoplastic resin is more preferably 15% by mass to 85% by mass, and even more preferably 30% by mass to 70% by mass.

The nitrile group-containing constitutional unit is preferably introduced using a monomer having a nitrile group.

Examples of the monomer having a nitrile group include an acrylonitrile compound. As the monomer having a nitrile group, for example, (meth)acrylonitrile is suitable.

As the nitrile group-containing constitutional unit, a constitutional unit formed of (meth)acrylonitrile is preferable.

From the viewpoint of ink receptivity, the content of the nitrile group-containing constitutional unit is preferably lower than the content of the aforementioned constitutional unit formed of an aromatic vinyl compound. The content of the nitrile group-containing constitutional unit with respect to the total mass of the resin is more preferably 55% by mass to 90% by mass, and even more preferably 60% by mass to 85% by mass.

In a case where the resin contained in the thermoplastic resin particles has the constitutional unit formed of an aromatic vinyl compound and the nitrile group-containing constitutional unit, the content ratio between the constitutional unit formed of an aromatic vinyl compound and the nitrile group-containing constitutional unit (constitutional unit formed of aromatic vinyl compound:nitrile group-containing constitutional unit) is preferably 5:5 to 9: 1, and more preferably 6:4 to 8:2, based on mass.

From the viewpoint of UV printing durability and chemical resistance, the resin contained in the thermoplastic resin particles preferably further has a constitutional unit formed of a N-vinyl heterocyclic compound.

Examples of the N-vinyl heterocyclic compound include N-vinylpyrrolidone, N-vinylcarbazole, N-vinylpyrrole, N-vinylphenothiazine, N-vinylsuccinic acid imide, N-vinylphthalimide, N-vinylcaprolactam, and N-vinylimidazole. Among these, N-vinylpyrrolidone is preferable.

The content of the constitutional unit formed of a N-vinyl heterocyclic compound with respect to the total mass of the thermoplastic resin is preferably 5% by mass to 50% by mass, and more preferably 10% by mass to 40% by mass.

The resin contained in the thermoplastic resin particles may contain an acidic group-containing constitutional unit. From the viewpoint of on-press developability and ink receptivity, it is preferable that the resin do not contain an acidic group-containing constitutional unit.

Specifically, in the thermoplastic resin, the content of the acidic group-containing constitutional unit is preferably 20% by mass or less, more preferably 10% by mass or less, and even more preferably 5% by mass or less. The lower limit of the content is not particularly limited, and may be 0% by mass.

The acid value of the thermoplastic resin is preferably 160 mg KOH/g or less, more preferably 80 mg KOH/g or less, and even more preferably 40 mg KOH/g or less. The lower limit of the acid value is not particularly limited, and may be 0 mg KOH/g.

In the present disclosure, the acid value is determined by the measurement method based on JIS K0070: 1992.

From the viewpoint of ink receptivity, the resin contained in the thermoplastic resin particles may contain a hydrophobic group-containing constitutional unit.

Examples of the hydrophobic group include an alkyl group, an aryl group, an aralkyl group, and the like.

As the hydrophobic group-containing constitutional unit, a constitutional unit formed of an alkyl (meth)acrylate compound, an aryl (meth)acrylate compound, or an aralkyl (meth)acrylate compound is preferable, and a constitutional unit formed of an alkyl (meth)acrylate compound is more preferable.

In the resin contained in the thermoplastic resin particles, the content of the hydrophobic group-containing constitutional unit with respect to the total mass of the resin is preferably 5% by mass to 50% by mass, and more preferably 10% by mass to 30% by mass.

From the viewpoint of UV printing durability and on-press developability, the thermoplastic resin contained in the thermoplastic resin particles preferably has a hydrophilic group.

The hydrophilic group is not particularly limited as long as it has a hydrophilic structure, and examples thereof include an acid group such as a carboxy group, a hydroxy group, an amino group, a nitrile group, a polyalkylene oxide structure, and the like.

From the viewpoint of UV printing durability and on-press developability, the hydrophilic group is preferably a group having a polyalkylene oxide structure, a group having a polyester structure, or a sulfonic acid group, more preferably a group having a polyalkylene oxide structure or a sulfonic acid group, and even more preferably a group having a polyalkylene oxide structure.

From the viewpoint of on-press developability, the polyalkylene oxide structure is preferably a polyethylene oxide structure, a polypropylene oxide structure, or a poly(ethylene oxide/propylene oxide) structure.

From the viewpoint of on-press developability, among the above hydrophilic groups, groups having a polypropylene oxide structure as a polyalkylene oxide structure are preferable, and groups having a polyethylene oxide structure and a polypropylene oxide structure are more preferable.

From the viewpoint of on-press developability, the number of alkylene oxide structures in the polyalkylene oxide structure is preferably 2 or more, more preferably 5 or more, even more preferably 5 to 200, and particularly preferably 8 to 150.

From the viewpoint of on-press developability, as the aforementioned hydrophilic group, a group represented by Formula Z, which will be described later, is preferable.

Among the hydrophilic groups that the thermoplastic resin has, a group represented by Formula PO is preferable.

In Formula PO, L^{P} each independently represent an alkylene group, R^{P} represents a hydrogen atom or an alkyl group, and n represents an integer of 1 to 100.

In Formula PO, L^{P} preferably each independently represent an ethylene group, a 1-methylethylene group, or a 2-methylethylene group, and more preferably each independently represent an ethylene group.

In Formula PO, R^{P} is preferably a hydrogen atom or an alkyl group having 1 to 18 carbon atoms, more preferably a hydrogen atom or an alkyl group having 1 to 10 carbon atoms, even more preferably a hydrogen atom or an alkyl group having 1 to 4 carbon atoms, and particularly preferably a hydrogen atom or a methyl group.

In Formula PO, n is preferably an integer of 1 to 10, and more preferably an integer of 1 to 4.

The content of the hydrophilic group-containing constitutional unit with respect to the total mass of the resin is preferably 5% by mass to 60% by mass, and more preferably 10% by mass to 30% by mass.

The resin contained in the thermoplastic resin particles may further contain other constitutional units. The resin can contain, as those other constitutional units, constitutional units other than the constitutional units described above without particular limitations. Examples thereof include constitutional units formed of an acrylamide compound, a vinyl ether compound, and the like.

In the resin contained in the thermoplastic resin particles, the content of other constitutional units with respect to the total mass of the resin is preferably 5% by mass to 50% by mass, and more preferably 10% by mass to 30% by mass.

Examples of the thermal reactive resin particles include resin particles having a thermal reactive group. The thermal reactive resin particles form a hydrophobic region through crosslinking by a thermal reaction and the accompanying change in functional groups.

The thermal reactive group in the resin particles having a thermal reactive group may be a functional group that causes any reaction as long as chemical bonds are formed. The thermal reactive group is preferably a polymerizable group. Preferred examples of the polymerizable group include an ethylenically unsaturated group that causes a radical polymerization reaction (for example, an acryloyl group, a methacryloyl group, a vinyl group, an allyl group, and the like), a cationically polymerizable group (for example, a vinyl group, a vinyloxy group, an epoxy group, an oxetanyl group, and the like), an isocyanato group or a blocked isocyanato group that causes an addition reaction, an epoxy group, a vinyloxy group, an active hydrogen atom-containing functional group that is a reaction partner thereof (for example, an amino group, a hydroxy group, a carboxy group, and the like), a carboxy group that causes a condensation reaction, a hydroxy group or an amino group that is a reaction partner of the carboxy group, an acid anhydride that causes a ring-opening addition reaction, an amino group or a hydroxy group which is a reaction partner of the acid anhydride, and the like.

The resin having a thermal reactive group may be an addition polymerization-type resin, a polyaddition-type resin, or a polycondensation-type resin or may be a thermoplastic resin.

As the microcapsules, for example, microcapsules are preferable which encapsulate at least some of the constituent components (preferably a hydrophobic compound) of the image-recording layer as described in JP2001-277740A and JP2001-277742A. In a preferred aspect of the image-recording layer containing microcapsules as resin particles, the image-recording layer is composed of microcapsules that encapsulate a hydrophobic component (that is, a hydrophobic compound) among the constituent components of the image-recording layer and a hydrophilic component (that is, a hydrophilic compound) that is on the outside of the microcapsules.

The microgel (crosslinked resin particles) can contain some of the constituent components of the image-recording layer, in at least one of the surface or the interior of the microgel. From the viewpoint of sensitivity of the lithographic printing plate precursor to be obtained and printing durability of the lithographic printing plate to be obtained, a reactive microgel having a polymerizable group on the surface thereof is particularly preferable.

In order to obtain microcapsules containing a constituent component of the image-recording layer, known synthesis methods can be used.

The microgel (crosslinked resin particles) can contain some of the constituent components of the image-recording layer, in at least one of the surface or the interior of the microgel. From the viewpoint of sensitivity of the lithographic printing plate precursor to be obtained and printing durability of the lithographic printing plate to be obtained, a reactive microgel having a polymerizable group on the surface thereof is particularly preferable.

In order to obtain a microgel containing a constituent component of the image-recording layer, known synthesis methods can be used.

As the resin particles, from the viewpoint of printing durability, antifouling properties, and storage stability of the lithographic printing plate to be obtained, polyaddition-type resin particles are preferable which are obtained by a reaction between a polyvalent isocyanate compound that is an adduct of a polyhydric phenol compound having two or more hydroxy groups in a molecule and isophorone diisocyanate and a compound having active hydrogen.

As the polyhydric phenol compound, a compound having a plurality of benzene rings having a phenolic hydroxyl group is preferable.

As the compound having active hydrogen, a polyol compound or a polyamine compound is preferable, a polyol compound is more preferable, and at least one kind of compound selected from the group consisting of propylene glycol, glycerin, and trimethylolpropane is even more preferable. As the aforementioned active hydrogen compound, water can also be used. In a case where water is used, the amine generated by the reaction between an isocyanato group and water can form a urea bond to form particles.

Preferred examples of the resin particles obtained by the reaction between a polyvalent isocyanate compound that is an adduct of a polyhydric phenol compound having two or more hydroxy groups in a molecule and isophorone diisocyanate and a compound having active hydrogen include the resin particles described in paragraphs "0230" to "0234" of WO2018043259A.

As the resin particles, from the viewpoint of printing durability and solvent resistance of the lithographic printing plate to be obtained, addition polymerization-type resin particles are preferable which have a hydrophobic main chain and include both i) constitutional unit having a nitrile group directly bonded to the hydrophobic main chain and ii) constitutional unit having a pendant group including a hydrophilic polyalkylene oxide segment. Specifically, the particles described in paragraph "0156" of JP2019-64269A are preferable.

It is preferable that the resin particles in the present disclosure have a group represented by Formula Z as a hydrophilic group.

*-Q-W-Y Formula Z

In Formula Z, Q represents a divalent linking group, W represents a divalent group having a hydrophilic structure or a divalent group having a hydrophobic structure, Y represents a monovalent group having a hydrophilic structure or a monovalent group having a hydrophobic structure, either W or Y has a hydrophilic structure, and * represents a bonding site with another structure.

Furthermore, it is preferable that any of the hydrophilic structures included in Formula Z include a polyalkylene oxide structure.

Preferred aspects of Q, W, and Y in Formula Z are the same as the preferred aspects of Q, W, and Y in Formula Z described above for the outermost layer.

The group represented by Formula Z may function as a dispersible group for improving the dispersibility of the resin particles.

From the viewpoint of printing durability and on-press developability, the resin particles in the present disclosure preferably have a polymerizable group (preferably an ethylenically unsaturated group). Particularly, the resin particles more preferably include resin particles having a polymerizable group on the surface thereof. In a case where the resin particles having a polymerizable group are used, printing durability (preferably UV printing durability) is improved.

From the viewpoint of printing durability, it is preferable that the resin particles in the present disclosure be resin particles having a hydrophilic group and a polymerizable group.

The polymerizable group may be a cationically polymerizable group or a radically polymerizable group. From the viewpoint of reactivity, the polymerizable group is preferably a radically polymerizable group.

The aforementioned polymerizable group is not particularly limited as long as it is a polymerizable group. From the viewpoint of reactivity, an ethylenically unsaturated group is preferable, a vinylphenyl group (styryl group), a (meth)acryloxy group, or a (meth)acrylamide group is more preferable, and a (meth)acryloxy group is particularly preferable.

In addition, it is preferable that the resin constituting the resin particles having a polymerizable group have a polymerizable group-containing constitutional unit.

The polymerizable group may be introduced into the surface of the resin particles by a polymer reaction.

Furthermore, from the viewpoint of printing durability, receptivity, on-press developability, and suppression of the occurrence of development residues during on-press development, the resin particles preferably contain a polyaddition-type resin having a urea bond, more preferably contain a polyaddition-type resin having a structure obtained by reacting at least an isocyanate compound represented by Formula (Iso) with water, and particularly preferably contain a polyaddition-type resin that has a structure obtained by reacting at least an isocyanate compound represented by Formula (Iso) with water and has a polyethylene oxide structure and a polypropylene oxide structure as polyoxyalkylene structures. Furthermore, the particles containing the polyaddition-type resin having a urea bond are preferably a microgel.

In Formula (Iso), n represents an integer of 0 to 10.

An example of the reaction between the isocyanate compound represented by Formula (Iso) and water is the reaction shown below. In the following example, a 4,4-isomer in which n = 0 is used.

As shown below, in a case where the isocyanate compound represented by Formula (Iso) is reacted with water, the isocyanate group is partially hydrolyzed by water and generates an amino group. The generated amino group reacts with the isocyanate group and generates a urea bond, and a dimer is consequently formed. Furthermore, the following reaction is repeated to form a polyaddition-type resin having a urea bond.

In the following reaction, by adding a compound (compound having active hydrogen) such as an alcohol compound or an amine compound reactive with an isocyanate group, it is possible to introduce the structure of an alcohol compound, an amine compound, or the like to the polyaddition-type resin having a urea bond.

Preferred examples of the compound having active hydrogen include the aforementioned compound having active hydrogen.

The polyaddition-type resin having a urea bond preferably has an ethylenically unsaturated group, and more preferably has a group represented by Formula (PETA).

In Formula (PETA), the portion of the wavy line represents a bonding position with other structures.

### <<Synthesis of resin particles>>

The synthesis method of the resin particles is not particularly limited, and may be a method that makes it possible to synthesize particles with various resins described above. Examples of the synthesis method of the resin particles include known synthesis methods of resin particles, such as an emulsion polymerization method, a suspension polymerization method, a dispersion polymerization method, a soap-free polymerization method, and a microemulsion polymerization method.

In addition, for the synthesis of the resin particles, a known microcapsule synthesis method, a known microgel (crosslinked resin particle) synthesis method, and the like may be used.

### <<Average particle diameter of particles »

The average particle diameter of the particles is preferably 0.01 µm to 3.0 µm, more preferably 0.03 µm to 2.0 µm, and even more preferably 0.10 µm to 1.0 µm. In a case where the average particle diameter is in this range, excellent resolution and temporal stability are obtained.

The average particle diameter of the particles is measured using a light scattering method or by capturing an electron micrograph of the particles, measuring the particle diameter of a total of 5,000 particles in the photograph, and calculating the average thereof. For non-spherical particles, the equivalent circle diameter of the particles in a photograph is adopted.

Note that unless otherwise specified, the average particle diameter of the particles in the present disclosure means a volume average particle diameter.

As the particles (preferably resin particles), only one kind of particles may be used, or two or more kinds of particles may be used in combination.

From the viewpoint of developability and printing durability, the content of the particles (preferably resin particles) with respect to the total mass of the image-recording layer is preferably 5% by mass to 90% by mass, more preferably 10% by mass to 90% by mass, even more preferably 20% by mass to 90% by mass, and particularly preferably 50% by mass to 90% by mass.

### [Other components]

The image-recording layer in the present disclosure may contain other components in addition to the components described above.

Examples of those other components include a binder polymer, a color developing agent, a chain transfer agent, a low-molecular-weight hydrophilic compound, an oil sensitizing agent, other additives, and the like.

Examples of those other components include a colorant, a bakeout agent, a polymerization inhibitor, a higher fatty acid derivative, a plasticizer, inorganic particles, and a low-molecular-weight hydrophilic compound disclosed in paragraphs "0181" to "0190" of JP2009-255434A, and the like.

Examples of other compounds also include a hydrophilic precursor (fine particles capable of converting the image-recording layer into a hydrophobic image-recording layer in a case where heat is applied thereto), a low-molecular-weight hydrophilic compound, an oil sensitizing agent (for example, a phosphonium compound, a nitrogen-containing low-molecular-weight compound, or an ammonium group-containing polymer), and a chain transfer agent disclosed in paragraphs "0191" to "0217" of JP2012-187907A.

### -Binder polymer-

As necessary, the image-recording layer may contain a binder polymer.

The binder polymer refers to a polymer other than resin particles, that is, a polymer that is not in the form of particles.

In addition, the binder polymer excludes an ammonium salt-containing polymer in an oil sensitizing agent and a polymer used as a surfactant.

As the binder polymer, known binder polymers (for example, a (meth) acrylic resin, polyvinyl acetal, a polyurethane resin, and the like) used for the image-recording layer of a lithographic printing plate precursor can be suitably used.

As an example, a binder polymer that is used for an on-press development type lithographic printing plate precursor (hereinafter, also called binder polymer for on-press development) will be specifically described.

As the binder polymer for on-press development, a binder polymer having an alkylene oxide chain is preferable. The binder polymer having an alkylene oxide chain may have a poly(alkylene oxide) moiety in a main chain or side chain. In addition, the binder polymer may be a graft polymer having poly(alkylene oxide) in a side chain or a block copolymer of a block composed of a poly(alkylene oxide)-containing repeating unit and a block composed of an (alkylene oxide)-free repeating unit.

As a binder polymer having a poly(alkylene oxide) moiety in the main chain, a polyurethane resin is preferable.

In a case where the binder polymer has a poly(alkylene oxide) moiety in the side chain, examples of polymers as the main chain include a (meth)acrylic resin, a polyvinyl acetal resin, a polyurethane resin, a polyurea resin, a polyimide resin, a polyamide resin, an epoxy resin, a polystyrene resin, a novolac-type phenol resin, a polyester resin, synthetic rubber, and natural rubber. Among these, a (meth)acrylic resin is particularly preferable.

In addition, as the binder polymer, for example, a polymer compound is also preferable which has a polyfunctional thiol having functionalities of 6 or more and 10 or less as a nucleus and a polymer chain that is bonded to the nucleus by a sulfide bond and has a polymerizable group (hereinafter, this compound will be also called star-shaped polymer compound).

As the star-shaped polymer compound, for example, the compounds described in JP2012-148555A can be preferably used.

Examples of the star-shaped polymer compound include the compound described in JP2008-195018A that has a polymerizable group such as an ethylenically unsaturated bond for improving the film hardness of an image area in a main chain or side chain and preferably in a side chain. The polymerizable group of the star-shaped polymer compound forms crosslinks between the molecules of the star-shaped polymer compound, which facilitates curing.

As the polymerizable group, an ethylenically unsaturated group such as a (meth)acryloyl group, a vinyl group, an allyl group, or a vinyl phenyl group (styryl group), an epoxy group, or the like is preferable, a (meth)acryloyl group, a vinyl group, or a vinyl phenyl group (styryl group) is more preferable from the viewpoint of polymerization reactivity, and a (meth)acryloyl group is particularly preferable. These groups can be introduced into the polymer by a polymer reaction or copolymerization. Specifically, for example, it is possible to use a reaction between a polymer having a carboxy group in a side chain and glycidyl methacrylate or a reaction between a polymer having an epoxy group and an ethylenically unsaturated group-containing carboxylic acid such as methacrylic acid.

The molecular weight of the binder polymer that is a polystyrene-equivalent weight-average molecular weight (Mw) determined by GPC is preferably 2,000 or more, more preferably 5,000 or more, and even more preferably 10,000 to 300,000.

As the binder polymer, as necessary, a water-soluble polymer, such as polyacrylic acid, polyvinyl alcohol, or polyvinyl acetal described in JP2008-195018A, can be used in combination. In addition, a lipophilic polymer and a hydrophilic polymer can be used in combination.

Particularly, from the viewpoint of on-press developability, the image-recording layer preferably contains polyvinyl acetal. Suitable examples of the polyvinyl acetal include polyvinyl butyral and the like.

Polyvinyl acetal is a resin obtained by acetalizing hydroxy groups of polyvinyl alcohol with an aldehyde.

Particularly, polyvinyl butyral is preferable which is obtained by acetalizing (that is, butyralizing) hydroxy groups of polyvinyl alcohol with butyraldehyde.

The polyvinyl acetal preferably has a constitutional unit represented by (a) which is obtained by acetalizing hydroxy groups of polyvinyl alcohol with an aldehyde.

R represents a residue of aldehyde used for acetalization.

Examples of R include a hydrogen atom, an alkyl group, and an ethylenically unsaturated group which will be described later.

The content of the constitutional unit represented by (a) (hereinafter, also described as the amount of ethylene groups in the main chain contained in the constitutional unit represented by (a), which is also called degree of acetalization) with respect to the total content of constitutional units of the polyvinyl acetal (that is, total amount of ethylene groups in the main chain) is preferably 50 mol% to 90 mol%, more preferably 55 mol% to 85 mol%, and even more preferably 55 mol% to 80 mol%.

The degree of acetalization is a value obtained by dividing the amount of ethylene groups to which acetal groups are bonded (that is, the amount of ethylene groups in the main chain contained in the constitutional unit represented by (a)) by the total amount of ethylene groups in the main chain and expressing the thus obtained molar fraction as a percentage.

The same shall be applied to the content of each constitutional unit of polyvinyl acetal which will be described later.

From the viewpoint of improving printing durability, the polyvinyl acetal preferably has an ethylenically unsaturated group.

The ethylenically unsaturated group that the polyvinyl acetal has is not particularly limited. From the viewpoint of reactivity, on-press developability, and printing durability, the ethylenically unsaturated group is more preferably at least one kind of group selected from the group consisting of a vinyl phenyl group (styryl group), a vinyl ester group, a vinyl ether group, an allyl group, a (meth)acryloxy group, and a (meth)acrylamide group. Among these, a vinyl group, an allyl group, a (meth)acryloxy group, and the like are preferable.

From the viewpoint of improving printing durability, the polyvinyl acetal preferably has an ethylenically unsaturated group-containing constitutional unit.

The ethylenically unsaturated group-containing constitutional unit may be the aforementioned constitutional unit having an acetal ring or a constitutional unit other than the constitutional unit having an acetal ring.

Particularly, from the viewpoint of increasing crosslink density during exposure, the polyvinyl acetal is preferably a compound in which an ethylenically unsaturated group is introduced into an acetal ring. That is, it is preferable that the constitutional unit represented by (a) have an ethylenically unsaturated group as R.

In a case where the ethylenically unsaturated group-containing constitutional unit is a constitutional unit other than the constitutional unit having an acetal ring, for example, the ethylenically unsaturated group-containing constitutional unit may be an acrylate group-containing constitutional unit, specifically, a constitutional unit represented by (d).

In a case where the ethylenically unsaturated group-containing constitutional unit is a constitutional unit other than the constitutional unit having an acetal ring, the content of the ethylenically unsaturated group-containing constitutional unit (also called amount of acrylate groups) with respect to the total content of constitutional units of the polyvinyl acetal is preferably 1 mol% to 15 mol%, and more preferably 1 mol% to 10 mol%.

From the viewpoint of on-press developability, the polyvinyl acetal preferably further has a hydroxy group-containing constitutional unit. That is, the polyvinyl acetal preferably contains a constitutional unit derived from vinyl alcohol.

Examples of the hydroxy group-containing constitutional unit include a constitutional unit represented by (b).

From the viewpoint of on-press developability, the content of the constitutional unit represented by (b) (also called amount of hydroxyl groups) with respect to the total content of constitutional units of the polyvinyl acetal is preferably 5 mol% to 50 mol%, more preferably 10 mol% to 40 mol%, and even more preferably 20 mol% to 40 mol%.

The polyvinyl acetal may further have other constitutional units.

Examples of those other constitutional units include an acetyl group-containing constitutional unit, specifically, a constitutional unit represented by (c).

The content of the constitutional unit represented by (c) (also called amount of acetyl groups) with respect to the total content of constitutional units of the polyvinyl acetal is preferably 0.5 mol% to 10 mol%, more preferably 0.5 mol% to 8 mol%, and even more preferably 1 mol% to 3 mol%.

The degree of acetalization, the amount of acrylate groups, the amount of hydroxyl groups, and the amount of acetyl groups can be determined as follows.

That is, by ¹H NMR spectroscopy, the content expressed as mol% is calculated from the ratio of peak surface area of protons of a methyl or methylene moiety of acetal, a methyl moiety of an acrylate group, and a methyl moiety of a hydroxyl group and an acetyl group.

The weight-average molecular weight of the polyvinyl acetal is preferably 18,000 to 150,000.

The solubility parameter (also called SP value) of the polyvinyl acetal is preferably 17.5 MPa^{1/2} to 20.0 MPa^{1/2}, and more preferably 18.0 MPa^{1/2} to 19.5 MPa^{1/2}.

In the present disclosure, as "solubility parameter (unit: (MPa)^{1/2})", the Hansen solubility parameters are used.

The Hansen solubility parameters are obtained by dividing the solubility parameters introduced by Hildebrand into three components, a dispersion element δd, a polarity element δp, and a hydrogen bond element δh, and expressing the parameters in a three-dimensional space. In the present disclosure, the solubility parameters (hereinafter, also called SP value) are expressed as δ (unit: (MPa)^{1/2}), and a value calculated by the following equation is used. $δ {\left(MPa\right)}^{1 / 2} = {\left({δd}^{2}+{δp}^{2}+{δh}^{2}\right)}^{1 / 2}$

The dispersion element δd, the polarity element δp, and the hydrogen bond element δh of various substances have been found by Hansen and his successors, and are described in detail in the Polymer Handbook (fourth edition), VII-698 to 711. The values of Hansen solubility parameters are also specifically described in the document "Hansen Solubility Parameters; A Users Handbook (CRC Press, 2007)" written by Charles M. Hansen.

In the present disclosure, as the Hansen solubility parameters in a partial structure of a compound, it is also possible to use the values estimated from the chemical structure by using the computer software "Hansen Solubility Parameters in Practice (HSPiP ver.4.1.07)".

Furthermore, in the present disclosure, in a case where a compound is an addition polymerization-type polymer, a polycondensation-type polymer, or the like, the SP value of the compound is expressed as the total SP value obtained by multiplying the SP values of monomer units by molar fractions. Furthermore, in a case where a compound is a low-molecular-weight compound having no monomer unit, the SP value is expressed as the total SP value of the compound.

In the present disclosure, the SP value of a polymer may be calculated from the molecular structure of the polymer by the Hoy method described in Polymer Handbook (fourth edition).

Specific examples of the aforementioned polyvinyl acetal are shown in [P-1 to P-3]. However, the polyvinyl acetal used in the present disclosure is not limited thereto.

In the following structures, "l" is 50 mol% to 90 mol%, "m" is 0.5 mol% to 10% by mass, "n" is 5 mol% to 50 mol%, and "o" is 1 mol% to 15 mol%.

As the aforementioned polyvinyl acetal, commercially available products can be used.

Examples of the commercially available products of the polyvinyl acetal include an S-LEC series manufactured by SEKISUI CHEMICAL CO., LTD. (specifically, S-LEC BX-L, BX-1, BX-5, BL-7Z, BM-1, BM-5, BH-6, BH-3, and the like).

The image-recording layer in the present disclosure preferably contains a resin having a fluorine atom, more preferably contains a fluorohydrocarbon group-containing copolymer, and particularly preferably contains a fluoroaliphatic hydrocarbon group-containing copolymer.

In a case where the resin having a fluorine atom, particularly, the fluorohydrocarbon group-containing copolymer is used, it is possible to inhibit surface abnormalities resulting from foaming during the formation of the image-recording layer and to improve the condition of the coating surface, and the formed image-recording layer has higher ink receptivity.

In addition, the image-recording layer containing the fluorohydrocarbon group-containing copolymer has high gradation and is highly sensitive, for example, to laser light. Therefore, the obtained lithographic printing plate exhibits excellent fogging properties by scattered light, reflected light, and the like and has excellent printing durability.

The fluorohydrocarbon group-containing copolymer preferably has a constitutional unit formed of a compound represented by any of Formula (F1) to Formula (F3), and more preferably has a constitutional unit formed of a compound represented by Formula (F2) or Formula (F3)

In Formula (F 1) to Formula (F3), R^{F1} each independently represent a hydrogen atom or a methyl group, L^{F} represents a single bond or a divalent linking group, Cf represents a linear or branched hydrocarbon group having 1 to 10 carbon atoms in which some or all of hydrogen atoms of the hydrocarbon group are substituted with fluorine atoms, R^{F2} represents a hydrogen atom or a fluorine atom, X^{F} each independently represent an oxygen atom, a sulfur atom, or -N(R^{F3})-, w1 to w3 each independently represent an integer of 0 to 9, w4 represents an integer of 1 to 10, w5 represents an integer of 0 to 2, and R^{F3} represents a hydrogen atom or an alkyl group having 1 to 4 carbon atoms.

L^{F} in Formula (F1) is preferably a single bond, an alkylene group having 1 to 20 carbon atoms, or a divalent arylene group having 6 to 20 carbon atoms, more preferably a single bond or a divalent arylene group having 6 to 20 carbon atoms, and particularly preferably a single bond.

Cf in Formula (F1) is preferably an aromatic hydrocarbon group having 6 to 10 carbon atoms in which some or all of the hydrogen atoms of the aromatic hydrocarbon group are substituted with fluorine atoms, more preferably a phenyl group in which some or all of hydrogen atoms are substituted with fluorine atoms, and particularly preferably a perfluorophenyl group.

X^{F} in Formula (F2) and Formula (F3) preferably each independently represent an oxygen atom or -N(R^{F3})-, and more preferably each independently represent an oxygen atom.

R^{F2} in Formula (F2) is preferably a fluorine atom.

w1 in Formula (F2) is preferably an integer of 0 to 2, more preferably 1 or 2, and particularly preferably 2.

w2 in Formula (F2) is preferably an integer of 0 to 4, and more preferably 0.

w3 in Formula (F2) is preferably 0 or 1, and more preferably 0.

w4 in Formula (F2) is preferably an integer of 2 to 10, more preferably an integer of 4 to 8, and particularly preferably an integer of 4 to 6.

w5 in Formula (F3) is preferably 0 or 1, and more preferably 0.

R^{F3} in Formula (F3) is preferably a hydrogen atom, a methyl group, an ethyl group, a n-propyl group, or a n-butyl group, and more preferably a hydrogen atom or a methyl group.

Specific examples of the monomers having a fluorine atom used in the resin having a fluorine atom will be shown below. However, the present disclosure is not limited thereto.

From the viewpoint of on-press developability and on-press development residue suppressiveness, the aforementioned fluorohydrocarbon group-containing copolymer preferably contains a constitutional unit having a polyalkylene oxide structure, and more preferably contains a constitutional unit that is formed of a compound represented by any of Formula (F1) and Formula (F2) and a constitutional unit that has a polyalkylene oxide structure.

The fluorohydrocarbon group-containing copolymer preferably further has a constitutional unit formed of at least one kind of compound selected from the group consisting of poly(oxyalkylene) acrylate and a poly(oxyalkylene) methacrylate, in addition to the constitutional unit formed of a compound represented by any of Formula (F1) and Formula (F2).

The polyoxyalkylene group in the poly(oxyalkylene) acrylate and poly(oxyalkylene) methacrylate can be represented by -(OR^{F3})ₓ-. R^{F3} represents an alkyl group, and x represents an integer of 2 or more. R^{F3} is preferably a linear or branched alkylene group having 2 to 4 carbon atoms. As the linear or branched alkylene group having 2 to 4 carbon atoms, -CH₂CH₂-, -CH₂CH₂CH₂-, -CH(CH₃)CH₂-, or -CH(CH₃)CH(CH₃)- is preferable. x is preferably an integer of 2 to 100.

In the polyoxyalkylene groups, x pieces of "OR^{F3}" may be the same as or different from each other. That is, the polyoxyalkylene group may be composed of two or more kinds of "OR^{F3}" that are regularly or irregularly bonded to each other. For example, the polyoxyalkylene group may be composed of a linear or branched oxypropylene unit and an oxyethylene unit that are regularly or irregularly bonded to each other. More specifically, the polyoxyalkylene group may be composed of a block of a linear or branched oxypropylene unit and a block of an oxyethylene unit that are bonded to each other.

The polyoxyalkylene group may have one or more linking groups (for example, -CONH-Ph-NHCO-, -S-, and the like, where Ph represents a phenylene group).

The molecular weight of the polyoxyalkylene group is preferably 250 to 3,000.

As the poly(oxyalkylene) acrylate and the poly(oxyalkylene) methacrylate described above, commercially available products or synthetic products may be used.

The poly(oxyalkylene) acrylate and the poly(oxyalkylene) methacrylate can be synthesized, for example, by reacting a hydroxypoly(oxyalkylene) compound with acrylic acid, methacrylic acid, acryloyl chloride, methacryloyl chloride, acrylic acid anhydride, or the like by known methods.

As the aforementioned hydroxypoly(oxyalkylene) compound, commercially available products may be used. Examples thereof include ADEKA (registered trademark) PLURONIC (registered trademark) manufactured by ADEKA Corporation, ADEKA polyether manufactured by ADEKA Corporation, Carbowax (registered trademark) manufactured by Union Carbide Corporation, Triton manufactured by The Dow Chemical Company., PEG manufactured by DKS Co. Ltd., and the like.

As the poly(oxyalkylene) acrylate and the poly(oxyalkylene) methacrylate, poly(oxyalkylene) diacrylate or the like synthesized by known methods may also be used.

One kind of binder polymer may be used alone, or two or more kinds of binder polymers may be used in combination.

The content of the binder polymer to be incorporated into the image-recording layer can be randomly set. The content of the binder polymer with respect to the total mass of the image-recording layer is preferably 1% by mass to 90% by mass, and more preferably 5% by mass to 80% by mass.

### -Color developing agent-

The image-recording layer in the present disclosure preferably contains a color developing agent, and more preferably contains an acid color developing agent. Furthermore, the color developing agent preferably includes a leuco compound.

"Color developing agent" used in the present disclosure means a compound that develops or removes color by a stimulus such as light or acid and thus changes the color of the image-recording layer. Furthermore, "acid color developing agent" means a compound that develops or removes color by being heated in a state of accepting an electron accepting compound (for example, a proton of an acid or the like) and thus changes the color of the image-recording layer. The acid color developing agent is particularly preferably a colorless compound which has a partial skeleton such as lactone, lactam, sultone, spiropyran, an ester, or an amide and allows such a partial skeleton to rapidly open the ring or to be cleaved when coming into contact with an electron accepting compound.

Examples of such an acid color developing agent include the compounds described in paragraphs "0184" to "0191" of JP2019-18412A.

Particularly, from the viewpoint of visibility, the color developing agent used in the present disclosure is preferably at least one kind of compound selected from the group consisting of a spiropyran compound, a spirooxazine compound, a spirolactone compound, and a spirolactam compound.

From the viewpoint of visibility, the color of a colorant after color development preferably has maximum absorption in the range of 450 to 650 nm. The tint is preferably red, purple, blue, or dark green.

From the viewpoint of visibility and visibility of exposed portions, the acid color developing agent is preferably a leuco colorant.

The aforementioned leuco colorant is not particularly limited as long as it has a leuco structure. The leuco colorant preferably has a spiro structure, and more preferably has a spirolactone ring structure.

From the viewpoint of visibility and visibility of exposed portions, the leuco colorant is preferably a leuco colorant having a phthalide structure or a fluoran structure.

Furthermore, from the viewpoint of visibility and visibility of exposed portions, the leuco colorant having a phthalide structure or a fluoran structure is preferably a compound represented by any of Formula (Le-1) to Formula (Le-3), and more preferably a compound represented by Formula (Le-2).

In Formula (Le-1) to Formula (Le-3), ERG each independently represent an electron-donating group, X₁ to X₄ each independently represent a hydrogen atom, a halogen atom, or dialkylanilino group, X₅ to X₁₀ each independently represent a hydrogen atom, a halogen atom, or a monovalent organic group, Y₁ and Y₂ each independently represent C or N, X₁ does not exist in a case where Y₁ is N, X₄ does not exist in a case where Y₂ is N, Ra₁ represents a hydrogen atom, an alkyl group, or an alkoxy group, and Rbi to Rb₄ each independently represent a hydrogen atom, an alkyl group, or an aryl group.

As the electron-donating groups represented by ERG in Formula (Le-1) to Formula (Le-3), from the viewpoint of visibility and visibility of exposed portions, an amino group, an alkylamino group, an arylamino group, a dialkylamino group, a monoalkyl monoarylamino group, a diarylamino group, an alkoxy group, an aryloxy group or an alkyl group is preferable, an amino group, alkylamino group, arylamino group, dialkylamino group, monoalkyl monoarylamino group, diarylamino group, alkoxy group, or an aryloxy group is more preferable an arylamino group, a monoalkyl monoarylamino group, or a diarylamino group is even more preferable, and an arylamino group or a monoalkyl monoarylamino group is particularly preferable.

From the viewpoint of visibility and visibility of exposed portions, X₁ to X₄ in Formula (Le-1) to Formula (Le-3) preferably each independently represent a hydrogen atom or a chlorine atom, and more preferably each independently represent a hydrogen atom.

From the viewpoint of visibility and visibility of exposed portions, X₅ to X₁₀ in Formula (Le-2) or Formula (Le-3) preferably each independently represent a hydrogen atom, a halogen atom, an alkyl group, an aryl group, an amino group, an alkylamino group, an arylamino group, a dialkylamino group, a monoalkyl monoarylamino group, a diarylamino group, a hydroxy group, an alkoxy group, an aryloxy group, an acyl group, an alkoxycarbonyl group, an aryloxycarbonyl group, or a cyano group, more preferably each independently represent a hydrogen atom, a halogen atom, an alkyl group, an aryl group, an alkoxy group, or an aryloxy group, even more preferably each independently represent a hydrogen atom, a halogen atom, an alkyl group, or an aryl group, and particularly preferably each independently represent a hydrogen atom.

From the viewpoint of visibility and visibility of exposed portions, it is preferable that at least one of Y₁ or Y₂ in Formula (Le-1) to Formula (Le-3) be C, and it is more preferable that both of Y₁ and Y₂ be C.

From the viewpoint of visibility and visibility of exposed portions, Ra₁ in Formula (Le-3) is preferably an alkyl group or an alkoxy group, more preferably an alkoxy group, and particularly preferably a methoxy group.

From the viewpoint of visibility and visibility of exposed portions, Rbi to Rb₄ in Formula (Le-1) preferably each independently represent a hydrogen atom or an alkyl group, more preferably each independently represent an alkyl group, and particularly preferably each independently represent a methyl group.

From the viewpoint of visibility and visibility of exposed portions, the leuco colorant having a phthalide structure or a fluoran structure is more preferably a compound represented by any of Formula (Le-4) to Formula (Le-6), and even more preferably a compound represented by Formula (Le-5).

In Formula (Le-4) to Formula (Le-6), ERG each independently represent an electron-donating group, X₁ to X₄ each independently represent a hydrogen atom, a halogen atom, or a dialkylanilino group, Y₁ and Y₂ each independently represent C or N, X₁ does not exist in a case where Y₁ is N, X₄ does not exist in a case where Y₂ is N, Ra₁ represents a hydrogen atom, an alkyl group, or an alkoxy group, and Rbi to Rb₄ each independently represent a hydrogen atom, an alkyl group, or an aryl group.

ERG, X₁ to X₄, Yi, Y₂, Ra₁, and Rbi to Rb₄ in Formula (Le-4) to Formula (Le-6) have the same definitions as ERG, X₁ to X₄, Y₁, Y₂, Ra₁, and Rbi to Rb₄ in Formula (Le-1) to Formula (Le-3) respectively, and preferred aspects thereof are also the same.

From the viewpoint of visibility and visibility of exposed portions, the leuco colorant having a phthalide structure or a fluoran structure is more preferably a compound represented by any of Formula (Le-7) to Formula (Le-9), and particularly preferably a compound represented by Formula (Le-8).

In Formula (Le-7) to Formula (Le-9), X₁ to X₄ each independently represent a hydrogen atom, a halogen atom, or a dialkylanilino group, Y₁ and Y₂ each independently represent C or N, X₁ does not exist in a case where Y₁ is N, X₄ does not exist in a case where Y₂ is N, Ra₁ to Ra₄ each independently represent a hydrogen atom, an alkyl group, or an alkoxy group, Rbi to Rb₄ each independently represent a hydrogen atom, an alkyl group, or an aryl group, and Rci and Rc₂ each independently represent an aryl group.

X₁ to X₄, Yi, and Y₂ in Formula (Le-7) to Formula (Le-9) have the same definition as X₁ to X₄, Yi, and Y₂ in Formula (Le-1) to Formula (Le-3) respectively, and preferred aspects thereof are also the same.

From the viewpoint of visibility and visibility of exposed portions, Ra₁ to Ra₄ in Formula (Le-7) preferably each independently represent an alkyl group or an alkoxy group, more preferably each independently represent an alkoxy group, and particularly preferably each independently represent a methoxy group.

From the viewpoint of visibility and visibility of exposed portions, Rbi to Rb₄ in Formula (Le-7) to Formula (Le-9) preferably each independently represent a hydrogen atom, an alkyl group, or an aryl group substituted with an alkyl group or alkoxy group, more preferably each independently represent a hydrogen atom or an alkyl group, and particularly preferably each independently represent a hydrogen atom or a methyl group.

From the viewpoint of visibility and visibility of exposed portions, Rci and Rc₂ in Formula (Le-8) preferably each independently represent a phenyl group or an alkylphenyl group, and more preferably each independently represent a phenyl group.

In Formula (Le-8), from the viewpoint of visibility and visibility of exposed portions, X₁ to X₄ preferably each represent a hydrogen atom, and Y₁ and Y₂ preferably each represent C.

From the viewpoint of visibility and visibility of exposed portions, Rbi and Rb₂ in Formula (Le-8) preferably each independently represent a hydrogen atom, an alkyl group, or an aryl group substituted with an alkyl group or an alkoxy group, more preferably each independently represent a hydrogen atom or an alkyl group.

The alkyl group in Formula (Le-1) to Formula (Le-9) may be linear or branched or may have a ring structure.

The number of carbon atoms in the alkyl group in Formula (Le-1) to Formula (Le-9) is preferably 1 to 20, more preferably 1 to 8, even more preferably 1 to 4, and particularly preferably 1 or 2.

The number of carbon atoms in the aryl group in Formula (Le-1) to Formula (Le-9) is preferably 6 to 20, more preferably 6 to 10, and particularly preferably 6 to 8.

Each of the groups in Formula (Le-1) to Formula (Le-9), such as a monovalent organic group, an alkyl group, an aryl group, a dialkylanilino group, an alkylamino group, and an alkoxy group, may have a substituent. Examples of the substituent include an alkyl group, an aryl group, a halogen atom, an amino group, an alkylamino group, an arylamino group, a dialkylamino group, a monoalkyl monoarylamino group, a diarylamino group, a hydroxy group, an alkoxy group, an aryloxy group, an acyl group, an alkoxycarbonyl group, an aryloxycarbonyl group, a cyano group, and the like. These substituents may be further substituted with these substituents.

Examples of the leuco colorant having the phthalide structure or the fluoran structure that are suitably used include the following compounds.

As the acid color developing agent, commercially available products can be used. Examples thereof include ETAC, RED500, RED520, CVL, S-205, BLACK305, BLACK400, BLACK100, BLACK500, H-7001, GREEN300, NIRBLACK78, BLUE220, H-3035, BLUE203, ATP, H-1046, and H-2114 (all manufactured by Fukui Yamada Chemical Co., Ltd.), ORANGE-DCF, Vermilion-DCF, PINK-DCF, RED-DCF, BLMB, CVL, GREEN-DCF, and TH-107 (all manufactured by Hodogaya Chemical Co., Ltd.), ODB, ODB-2, ODB-4, ODB-250, ODB-BlackXV, Blue-63, Blue-502, GN-169, GN-2, Green-118, Red-40, and Red-8 (all manufactured by Yamamoto Chemicals, Inc.), crystal violet lactone (manufactured by Tokyo Chemical Industry Co., Ltd.), and the like. Among these commercially available products, ETAC, S-205, BLACK305, BLACK400, BLACK100, BLACK500, H-7001, GREEN300, NIRBLACK78, H-3035, ATP, H-1046, H-2114, GREEN-DCF, Blue-63, GN-169, and crystal violet lactone are preferable because these form a film having excellent visible light absorbance.

From the viewpoint of visibility and visibility of exposed portions, examples of suitably used a leuco colorant include the following compounds.

One kind of each of these color developing agents may be used alone. Alternatively, two or more kinds of components can be used in combination.

The content of the color developing agent with respect to the total mass of the image-recording layer is preferably 0.5% by mass to 10% by mass, and more preferably 1% by mass to 5% by mass.

### [Coloring compound and compound represented by Formula 1C or Formula 2C]

From the viewpoint of visibility of exposed portions, the image-recording layer preferably contains a coloring compound capable of having a coloring reaction with a decomposition product generated by the exposure of the image-recording layer, and more preferably contains a boron compound and a coloring compound.

Furthermore, from the viewpoint of visibility of exposed portions, the image-recording layer preferably contains a compound represented by Formula 1C or Formula 2C as the coloring compound, and more preferably contains a boron compound and a compound represented by Formula 1C or Formula 2C as the coloring compound.

In Formula 1C and Formula 2C, R^{1C} to R^{4C} each independently represent a monovalent organic group, L^{1C} and L^{2C} each independently represent a divalent organic group, A^{C} represents OH or NR^{5C}R^{6C}, R^{5C} and R^{6C} each independently represent a hydrogen atom or a monovalent organic group, and a dotted line portion represents a portion which may be a double bond.

"Coloring reaction" in the present disclosure is a chemical reaction accompanying a phenomenon of color development or discoloration.

The decomposition product generated by the exposure of the image-recording layer is not particularly limited. From the viewpoint of visibility of exposed portions, the decomposition product is preferably a decomposition product generated by the exposure of a polymerization initiator or a decomposition product generated by the exposure of an infrared absorber, more preferably a decomposition product generated by the exposure of a polymerization initiator, and particularly preferably a decomposition product generated by the exposure of an electron-donating polymerization initiator.

The decomposition product generated by the exposure of the image-recording layer includes not only a decomposition product decomposed by the exposure of the image-recording layer but also a compound generated by the further decomposition or modification of the decomposition product.

From the viewpoint of visibility of exposed portions, the coloring reaction is preferably a complex-forming reaction, and more preferably a boron complex-forming reaction.

An example of the coloring reaction will be shown below. The following reaction is a coloring reaction that occurs in a case where curcumin is used as a coloring compound, and sodium tetraphenylborate as a decomposition product generated by the exposure of the image-recording layer decomposes and generates boric acid. Due to keto-enol tautomerism, an enol tautomer of curcumin is generated as equilibrium. The reaction between the enol tautomer and the boric acid generates the following boron complex (Complex), and a coloring reaction from curcumin (yellow) to the following boron complex (red) occurs.

What is shown below is an example where hydrolysis proceeds to generate boric acid. For example, curcumin may form a complex together with diphenyl monohydroxyborate, monophenyl dihydroxyborate, or the like, or triphenyl borate may be coordinated as a zero-valent ligand to enol-type curcumin to form a complex.

From the viewpoint of visibility of exposed portions and tone reproducibility, the above coloring compound is preferably a compound having one or more ketone structures, more preferably a compound having one or more 1,3-diketone structures, β-hydroxyketone structures, or β-aminoketone structures, even more preferably a compound having one or more 1,3-diketone structures or β-hydroxyketone structures, and particularly preferably a compound having one or more 1,3-diketone structures.

Examples of the coloring compound also include a compound having one or more 1-hydroxy-3-amino structures or 1-hydroxy-3-imino structures.

From the viewpoint of visibility of exposed portions and tone reproducibility, the coloring compound is preferably a compound having an aromatic ring structure, more preferably a compound having two or more aromatic ring structures, even more preferably a compound having two to four aromatic ring structures, and particularly preferably a compound having two aromatic ring structures.

As the aromatic ring structure, from the viewpoint of visibility of exposed portions and tone reproducibility, for example, at least one kind of structure selected from the group consisting of a benzene ring structure and a naphthalene ring structure is preferable, and a benzene ring structure is more preferable.

The coloring compound may be a salt or a hydrate.

In a case where the coloring compound reacts with a decomposition product generated by the exposure of the image-recording layer and forms a complex, in the complex, the coloring compound may be a monodentate ligand or a polydentate ligand. From the viewpoint of complex forming properties, visibility of exposed portions, and tone reproducibility, the coloring compound is preferably a polydentate ligand, more preferably a ligand having a denticity of 2 to 6, even more preferably a ligand having a denticity of 2 to 4, particularly preferably a ligand having a denticity of 2 or 3, and most preferably a bidentate ligand.

From the viewpoint of visibility of exposed portions and tone reproducibility, the image-recording layer preferably contains a compound represented by Formula 1C or Formula 2C and more preferably contains a compound represented by Formula 1C, as the coloring compound.

Furthermore, in the image-recording layer, after exposure, the compound represented by Formula 1C or Formula 2C preferably reacts with the decomposition product generated by the exposure of the image-recording layer and forms a complex that has the compound represented by Formula 1C or Formula 2C as a zero-valent ligand or an anion formed by the removal of one hydrogen atom from the compound represented by Formula 1C or Formula 2C as a monovalent ligand, and more preferably reacts with the decomposition product generated by the exposure of the image-recording layer and forms a complex that has an anion formed by the removal of one hydrogen atom from the compound represented by Formula 1C or Formula 2C as a monovalent ligand.

In Formula 1C and Formula 2C, R^{1C} to R^{4C} each independently represent a monovalent organic group, L^{1C} and L^{2C} each independently represent a divalent organic group, A^{C} represents OH or NR^{5C}R^{6C}, R^{5C} and R^{6C} each independently represent a hydrogen atom or a monovalent organic group, and a dotted line portion represents a portion which may be a double bond.

In Formula 1C, two or more of R^{1C}, L^{1C}, and R^{2C} may be bonded to form a ring structure.

In Formula 2C, two or more of R^{3C}, L^{2C}, R^{4C}, R^{5C}, and R^{6C} may be bonded to form a ring structure.

From the viewpoint of visibility of exposed portions and tone reproducibility, R^{1C} and R^{2C} in Formula 1C preferably each independently represent a monovalent organic group having an aromatic ring, more preferably each independently represent an aryl group or an alkenyl group having an aryl group, and particularly preferably each independently represent a 2-arylvinyl group.

The aryl group may have a substituent. From the viewpoint of visibility of exposed portions and tone reproducibility, the aryl group is preferably an aryl group which has one or more groups selected from the group consisting of a hydroxy group and an alkoxy group as substituents, more preferably a phenyl group which has one or more groups selected from the group consisting of a hydroxy group and an alkoxy group as substituents, and particularly preferably a phenyl group which has a hydroxy group and an alkoxy group as substituents.

R^{1C} and R^{2C} in Formula 1C preferably each independently has a carbon number (number of carbon atoms) of 6 to 50, more preferably each independently has a carbon number of 6 to 20, and particularly preferably each independently has a carbon number of 8 to 20.

It is preferable that R^{1C} and R^{2C} in Formula 1C be the same group.

L^{1C} in Formula 1C is preferably an alkylene group and more preferably a methylene group.

From the viewpoint of visibility of exposed portions and tone reproducibility, R^{3C} in Formula 2C is preferably a monovalent organic group having an aromatic ring, and more preferably an aryl group or an alkenyl group having an aryl group.

In Formula 2C, from the viewpoint of visibility of exposed portions and tone reproducibility, L^{2C} and R^{4C} are preferably bonded to form an aromatic ring, and more preferably bonded to form a benzene ring.

R^{3C} and R^{4C} in Formula 2C preferably each independently have 6 to 50 carbon atoms, more preferably each independently have 6 to 30 carbon atoms, and particularly preferably each independently have 6 to 20 carbon atoms.

In a case where L^{2C} in Formula 2C is not bonded to R^{4C}, L^{2C} is preferably an alkylene group and more preferably a methylene group.

It is preferable that L^{2C} in Formula 2C be bonded to R^{4C} to form a ring member of an aromatic ring structure.

From the viewpoint of visibility of exposed portions and tone reproducibility, the compound represented by Formula 2C is preferably a compound having a 1-hydroxyanthraquinone structure or a 1-aminoanthraquinone structure, and more preferably a compound having a 1-hydroxyanthraquinone structure.

From the viewpoint of visibility of exposed portions and tone reproducibility, A^{C} in Formula 2C is preferably OH or NHR^{6C}, and more preferably OH.

R^{5C} in NR^{5C}R^{6C} in Formula 2C is preferably a hydrogen atom, an alkyl group, or an aryl group, more preferably a hydrogen atom or an alkyl group, and particularly preferably a hydrogen atom.

R^{6C} in NR^{5C}R^{6C} in Formula 2C is preferably a hydrogen atom, an alkyl group, or an anthraquinolyl group, more preferably an anthraquinolyl group, and particularly preferably a 1-anthraquinolyl group.

Specifically, suitable examples of the coloring compound include curcumin (CU-1 shown below), demethoxycurcumin (CU-2 shown below), alizarin (CU-3 shown below), iminodianthraquinone (CU-4 shown below), carminic acid (CU-5 shown below), azomethine H (CU-6 shown below), 1,3-bis(4-methoxyphenyl)-1,3-propanedione (CU-7 shown below), 4-methoxychalcone (CU-8 shown below), 1,3-bis(4-dimethylaminophenyl)-1,3-propanedione (CU-9 shown below), and the like.

One kind of coloring compound may be used alone, or two or more kinds of coloring compounds may be used in combination.

In addition, one kind of compound represented by Formula 1C or Formula 2C may be used alone, or two or more kinds of compounds represented by Formula 1C or Formula 2C may be used in combination.

Furthermore, one kind of complex described above may be formed, or two or more kinds of complexes described above may be formed.

From the viewpoint of visibility of exposed portions and tone reproducibility, the content of the coloring compound with respect to the total mass of the image-recording layer is preferably 0.001% by mass to 5% by mass, more preferably 0.01% by mass to 3% by mass, even more preferably 0.05% by mass to 2.5% by mass, and particularly preferably 0.05% by mass to 1.0% by mass.

From the viewpoint of visibility of exposed portions and tone reproducibility, the content of the compound represented by Formula 1C or Formula 2C with respect to the total mass of the image-recording layer is preferably 0.001% by mass to 5% by mass, more preferably 0.01% by mass to 3% by mass, even more preferably 0.05% by mass to 2.5% by mass, and particularly preferably 0.05% by mass to 1.0% by mass.

The molar ratio of a content M^{C} of the coloring compound (preferably the compound represented by Formula 1 or Formula 2) in the image-recording layer to a content M^{I} of the polymerization initiator in the image-recording layer is preferably M^{C}/M^{I} = 0.001 to 1, more preferably M^{C}/M^{I} = 0.01 to 0.8, and particularly preferably M^{C}/M^{I} = 0.05 to 0.5.

The molar ratio of a content M^{C} of the coloring compound (preferably the compound represented by Formula 1 or Formula 2) in the image-recording layer to a content M^{DI} of the Electron-donating polymerization initiator in the image-recording layer is preferably M^{C}/M^{DI} = 0.001 to 1.5, more preferably M^{C}/M^{DI} = 0.01 to 1, and particularly preferably M^{C}/M^{DI} = 0.05 to 0.8.

### [Chain transfer agent]

The image-recording layer used in the present disclosure may contain a chain transfer agent. The chain transfer agent contributes to the improvement of UV printing durability of the lithographic printing plate.

As the chain transfer agent, a thiol compound is preferable, a thiol compound having 7 or more carbon atoms is more preferable from the viewpoint of boiling point (low volatility), and a compound having a mercapto group on an aromatic ring (aromatic thiol compound) is even more preferable. The thiol compound is preferably a monofunctional thiol compound.

Specific examples of the chain transfer agent include the following compounds.

Only one kind of chain transfer agent may be added to the image-recording layer, or two or more kinds of chain transfer agents may be used in combination.

The content of the chain transfer agent with respect to the total mass of the image-recording layer is preferably 0.01% by mass to 50% by mass, more preferably 0.05% by mass to 40% by mass, and even more preferably 0.1% by mass to 30% by mass.

### [Oil sensitizing agent]

In order to improve ink receptivity, the image-recording layer preferably further contains an oil sensitizing agent.

The SP value of the oil sensitizing agent is preferably less than 18.0, more preferably 14 or more and less than 18, even more preferably 15 to 17, and particularly preferably 16 to 16.9.

Furthermore, the oil sensitizing agent may be a compound having a molecular weight (weight-average molecular weight in a case where the compound has molecular weight distribution) of 2,000 or more, or a compound having a molecular weight less than 2,000.

In the present disclosure, as the SP value (solubility parameters, unit: (MPa)^{1/2}), the Hansen solubility parameters are used.

The Hansen solubility parameters are obtained by dividing the solubility parameters introduced by Hildebrand into three components, a dispersion element δd, a polarity element δp, and a hydrogen bond element δh, and expressing the parameters in a three-dimensional space. In the present disclosure, the SP value is expressed as δ (unit: (MPa)^{1/2}), and a value calculated by the following equation is used. $δ {\left(MPa\right)}^{1 / 2} = {\left({δd}^{2}+{δp}^{2}+{δh}^{2}\right)}^{1 / 2}$

The dispersion element δd, the polarity element δp, and the hydrogen bond element δh of various substances have been found by Hansen and his successors, and are described in detail in the Polymer Handbook (fourth edition), VII-698 to 711.

Furthermore, in the present disclosure, the SP value of a polymer is calculated from the molecular structure of the polymer by the Hoy method described in Polymer Handbook fourth edition.

Examples of the aforementioned oil sensitizing agent include an onium salt compound, a nitrogen-containing low-molecular-weight compound, an ammonium compound such as an ammonium group-containing polymer, and the like.

Particularly, in a case where an inorganic lamellar compound is incorporated into an overcoat layer, these compounds function as a surface coating agent for the inorganic lamellar compound and can inhibit the receptivity deterioration caused in the middle of printing by the inorganic lamellar compound.

From the viewpoint of receptivity, the oil sensitizing agent is preferably an onium salt compound.

Examples of the onium salt compound include a phosphonium compound, an ammonium compound, a sulfonium compound, and the like. As the onium salt compound, from the viewpoint described above, at least one kind of compound selected from the group consisting of a phosphonium compound and an ammonium compound is preferable.

The onium salt compound, which will be described later, in a development accelerator or electron-accepting polymerization initiator is a compound having an SP value more than 18, and is not included in the oil sensitizing agent.

Examples of the phosphonium compound include the phosphonium compounds described in JP2006-297907A and JP2007-50660A. Specific examples thereof include 1,4-bis(triphenylphosphonio)butane=di(hexafluorophosphate), 1,7-bis(triphenylphosphonio)heptane=sulfate, and 1,9-bis(triphenylphosphonio)nonane=naphthalene-2,7-disulfonate, and the like.

Preferred examples of the ammonium compound include a nitrogen-containing low-molecular-weight compound, an ammonium group-containing polymer, and the like.

Examples of the nitrogen-containing low-molecular-weight compound include amine salts and quaternary ammonium salts. In addition, examples thereof also include imidazolinium salts, benzimidazolinium salts, pyridinium salts, and quinolinium salts.

Among these, quaternary ammonium salts and pyridinium salts are preferable.

Specific examples thereof include tetramethylammonium=hexafluorophosphate, tetrabutylammonium=hexafluorophosphate, dodecyltrimethylammonium=p-toluenesulfonate, benzyltriethylammonium=hexafluorophosphate, benzyldimethyloctylammonium=hexafluorophosphate, benzyldimethyldodecylammonium=hexafluorophosphate, the compounds described in paragraphs "0021" to "0037" of JP2008-284858A, the compounds described in paragraphs "0030" to "0057" of JP2009-90645A, and the like.

The ammonium group-containing polymer may have an ammonium group in the structure. As such a polymer, a polymer is preferable in which the content of (meth)acrylate having an ammonium group in a side chain as a copolymerization component is 5 mol% to 80 mol%. Specific examples thereof include the polymers described in paragraphs "0089" to "0105" of JP2009-208458A.

The reduced specific viscosity (unit: ml/g) of an ammonium salt-containing polymer determined according to the measurement method described in JP2009-208458A is preferably in a range of 5 to 120, more preferably in a range of 10 to 110, and particularly preferably in a range of 15 to 100. In a case where the reduced specific viscosity is converted into a weight-average molecular weight (Mw), the weight-average molecular weight is preferably 10,000 to 150,000, more preferably 17,000 to 140,000, and particularly preferably 20,000 to 130,000.

Specific examples of the ammonium group-containing polymer will be shown below.
(1) 2-(Trimethylammonio)ethylmethacrylate=p-toluenesulfonate/3,6-dioxaheptylmethacrylate copolymer (molar ratio: 10/90, Mw: 45,000)
(2) 2-(Trimethylammonio)ethylmethacrylate=hexafluorophosphate/3,6-dioxaheptylmethacrylate copolymer (molar ratio: 20/80, Mw: 60,000)
(3) 2-(Ethyldimethylammonio)ethylmethacrylate=p-toluenesulfonate/hexylmethacrylate copolymer (molar ratio: 30/70, Mw: 45,000)
(4) 2-(Trimethylammonio)ethylmethacrylate=hexafluorophosphate/2-ethylhexylmethacrylate copolymer (molar ratio: 20/80, Mw: 60,000)
(5) 2-(Trimethylammonio)ethylmethacrylate=methylsulfate/hexylmethacrylate copolymer (molar ratio: 40/60, Mw: 70,000)
(6) 2-(Butyldimethylammonio)ethylmethacrylate=hexafluorophosphate/3,6-dioxaheptylmethacryl ate copolymer (molar ratio: 25/75, Mw: 65,000)
(7) 2-(Butyldimethylammonio)ethylacrylate=hexafluorophosphate/3,6-dioxaheptylmethacrylate copolymer (molar ratio: 20/80, Mw: 65,000)
(8) 2-(Butyldimethylammonio)ethylmethacrylate=13-ethyl-5,8,11-trioxa-1-heptadecanesulfonate/ 3,6-dioxaheptylmethacrylate copolymer (molar ratio: 20/80, Mw: 75,000)

The content of the oil sensitizing agent with respect to the total mass of the image-recording layer is preferably 1% by mass to 40.0% by mass, more preferably 2% by mass to 25.0% by mass, and even more preferably 3% by mass to 20.0% by mass.

The image-recording layer may contain only one kind of oil sensitizing agent, or two or more kinds of oil sensitizing agents may be used in combination.

One of the preferred aspects of the image-recording layer used in the present disclosure is an aspect in which the image-recording layer contains two or more kinds of compounds as an oil sensitizing agent.

Specifically, from the viewpoint of satisfying both the on-press developability and receptivity, the image-recording layer used in the present disclosure preferably uses all the phosphonium compound, the nitrogen-containing low-molecular-weight compound, and the ammonium group-containing polymer as an oil sensitizing agent, and more preferably uses all the phosphonium compound, the quaternary ammonium salts, and the ammonium group-containing polymer as an oil sensitizing agent.

### [Development accelerator]

The image-recording layer used in the present disclosure preferably further contains a development accelerator.

The value of polarity element as an SP value of the development accelerator is preferably 6.0 to 26.0, more preferably 6.2 to 24.0, even more preferably 6.3 to 23.5, and particularly preferably 6.4 to 22.0.

In the present disclosure, as the value of polarity element as an SP value (solubility parameter, unit: (cal/cm³)^{1/2}), the value of polarity element δp in the Hansen solubility parameters is used. The Hansen solubility parameters are obtained by dividing the solubility parameters introduced by Hildebrand into three components, a dispersion element δd, a polarity element δp, and a hydrogen bond element δh, and expressing the parameters in a three-dimensional space. In the present disclosure, the polarity element δp is used.

δp [cal/cm³] is a dipole-dipole force element in the Hansen solubility parameters, V [cal/cm³] is a molar volume, and µ [D] is a dipole moment. As δp, the following equation simplified by Hansen and Beerbower is generally used.
${δ}_{p} = \frac{37.4 μ}{{V}^{1 / 2}}$

The development accelerator is preferably a hydrophilic polymer compound or a hydrophilic low-molecular-weight compound.

In the present disclosure, "hydrophilic" means that the value of polarity element as an SP value is 6.0 to 26.0, the hydrophilic polymer compound refers to a compound having a molecular weight (weight-average molecular weight in a case where the compound has molecular weight distribution) of 3,000 or more, and the hydrophilic low-molecular-weight compound refers to a compound having a molecular weight (weight-average molecular weight in a case where the compound has molecular weight distribution) of less than 3,000.

Examples of the hydrophilic polymer compound include a cellulose compound and the like. Among these, a cellulose compound is preferable.

Examples of the cellulose compound include cellulose or a compound obtained by modifying at least a part of cellulose (modified cellulose compound). Among these, a modified cellulose compound is preferable.

Preferred examples of the modified cellulose compound include a compound which is obtained by substituting at least some of hydroxy groups of cellulose with at least one kind of group selected from the group consisting of an alkyl group and a hydroxyalkyl group.

The degree of substitution of the compound, which is obtained by substituting at least some of hydroxy groups of cellulose with at least one kind of group selected from the group consisting of an alkyl group and a hydroxyalkyl group, is preferably 0.1 to 6.0, and more preferably 1 to 4.

As the modified cellulose compound, an alkyl cellulose compound or a hydroxyalkyl cellulose compound is preferable, and a hydroxyalkyl cellulose compound is more preferable.

Preferred examples of the alkyl cellulose compound include methyl cellulose.

Preferred examples of the hydroxyalkyl cellulose compound include hydroxypropyl cellulose.

The molecular weight of the hydrophilic polymer compound (weight-average molecular weight in a case where the compound has molecular weight distribution) is preferably 3,000 to 5,000,000, and more preferably 5,000 to 200,000.

Examples of the hydrophilic low-molecular-weight compound include a glycol compound, a polyol compound, an organic amine compound, an organic sulfonic acid compound, an organic sulfamine compound, an organic sulfuric acid compound, an organic phosphonic acid compound, an organic carboxylic acid compound, a betaine compound, and the like. Among these, a polyol compound, an organic sulfonic acid compound, or a betaine compound is preferable.

Examples of the glycol compound include glycols such as ethylene glycol, diethylene glycol, triethylene glycol, propylene glycol, dipropylene glycol, and tripropylene glycol, and ether or ester derivatives of these compounds.

Examples of the polyol compound include glycerin, pentaerythritol, tris(2-hydroxyethyl) isocyanurate, and the like.

Examples of the organic amine compound include triethanolamine, diethanolamine, monoethanolamine, salts of these, and the like.

Examples of the organic sulfonic acid compound include alkyl sulfonic acid, toluene sulfonic acid, benzene sulfonic acid, salts of these, and the like. Among these, for example, alkyl sulfonic acid having an alkyl group having 1 to 10 carbon atoms is preferable.

Examples of the organic sulfamine compound include alkylsulfamic acid, salts thereof, and the like.

Examples of the organic sulfuric acid compound include alkyl sulfate, alkyl ether sulfuric acid, salts of these, and the like.

Examples of the organic phosphonic acid compound include phenylphosphonic acid, salts thereof, and the like.

Examples of the organic carboxylic acid compound include tartaric acid, oxalic acid, citric acid, malic acid, lactic acid, gluconic acid, salts of these, and the like.

Examples of the betaine compound include a phosphobetaine compound, a sulfobetaine compound, a carboxybetaine compound, and the like. Among these, for example, trimethylglycine is preferable.

The molecular weight of the hydrophilic low-molecular-weight compound (weight-average molecular weight in a case where the compound has molecular weight distribution) is preferably 100 or more and less than 3,000, and more preferably 300 to 2,500.

The development accelerator is preferably a compound having a cyclic structure.

The cyclic structure is not particularly limited. Examples thereof include a glucose ring in which at least some of hydroxy groups may be substituted, an isocyanuric ring, an aromatic ring which may have a heteroatom, an aliphatic ring which may have a heteroatom, and the like. Among these, for example, a glucose ring or an isocyanuric ring is preferable.

Examples of the compound having a glucose ring include the aforementioned cellulose compound.

Examples of the compound having an isocyanuric ring include the aforementioned tris(2-hydroxyethyl) isocyanurate and the like.

Examples of the compound having an aromatic ring include the toluene sulfonic acid and benzene sulfonic acid described above, and the like.

Examples of the compound having an aliphatic ring include a compound which is the aforementioned alkyl sulfate and has an alkyl group having a ring structure, and the like.

The compound having a cyclic structure preferably has a hydroxy group.

Preferred examples of the compound having a hydroxy group and a cyclic structure include the aforementioned cellulose compound and the aforementioned tris(2-hydroxyethyl) isocyanurate.

The development accelerator is preferably an onium salt compound.

Examples of the onium salt compound include an ammonium compound, a sulfonium compound, and the like. Among these, an ammonium compound is preferable.

Examples of the development accelerator which is an onium salt compound include trimethylglycine and the like.

The value of polarity element as an SP value of the onium salt compound in the electron-accepting polymerization initiator is not in a range of 6.0 to 26.0. This onium salt compound is not included in the development accelerator.

The image-recording layer may contain only one kind of development accelerator, or two or more kinds of development accelerators may be used in combination.

One of the preferred aspects of the image-recording layer used in the present disclosure is an aspect in which the image-recording layer contains two or more kinds of compounds as a development accelerator.

Specifically, from the viewpoint of on-press developability and receptivity, the image-recording layer used in the present disclosure preferably contains, as a development accelerator, the polyol compound and the betaine compound described above, the betaine compound and the organic sulfonic acid compound described above, or the polyol compound and the organic sulfonic acid compound described above.

The content of the development accelerator with respect to the total mass of the image-recording layer is preferably 0.1% by mass or more and 20% by mass or less, more preferably 0.5% by mass or more and 15% by mass or less, and even more preferably 1% by mass or more and 10% by mass or less.

### [Other components]

As other components, a surfactant, a polymerization inhibitor, a higher fatty acid derivative, a plasticizer, inorganic particles, an inorganic lamellar compound, and the like can be incorporated into the image-recording layer. Specifically, the description in paragraphs "0114" to "0159" of JP2008-284817A can be referred to.

### [Formation of image-recording layer]

The image-recording layer in the lithographic printing plate precursor according to the present disclosure can be formed, for example, by preparing a coating liquid by dispersing or dissolving the necessary components described above in a known solvent, coating a support with the coating liquid by a known method such as bar coating, and drying the coating liquid, as described in paragraphs "0142" and "0143" of JP2008-195018A. The coating amount (solid content) of the image-recording layer after coating and drying varies with uses, but is preferably 0.3 g/m² to 3.0 g/m². In a case where the coating amount is in this range, excellent sensitivity and excellent film characteristics of the image-recording layer are obtained.

As the solvent, known solvents can be used. Specific examples thereof include water, acetone, methyl ethyl ketone (2-butanone), cyclohexane, ethyl acetate, ethylene dichloride, tetrahydrofuran, toluene, ethylene glycol monomethyl ether, ethylene glycol monoethyl ether, ethylene glycol dimethyl ether, propylene glycol monomethyl ether, propylene glycol monoethyl ether, acetylacetone, cyclohexanone, diacetone alcohol, ethylene glycol monomethyl ether acetate, ethylene glycol ethyl ether acetate, ethylene glycol monoisopropyl ether, ethylene glycol monobutyl ether acetate, 1-methoxy-2-propanol, 3-methoxy-1-propanol, methoxy methoxyethanol, diethylene glycol monomethyl ether, diethylene glycol monoethyl ether, diethylene glycol dimethyl ether, diethylene glycol diethyl ether, propylene glycol monomethyl ether acetate, propylene glycol monoethyl ether acetate, 3-methoxypropyl acetate, N,N-dimethylformamide, dimethyl sulfoxide, γ-butyrolactone, methyl lactate, ethyl lactate, and the like. One kind of solvent may be used alone, or two or more kinds of the solvents may be used in combination. The concentration of solid contents in the coating liquid is preferably 1% by mass to 50% by mass.

The coating amount (solid content) of the image-recording layer after coating and drying varies with uses. However, from the viewpoint of obtaining excellent sensitivity and excellent film characteristics of the image-recording layer, the coating amount is preferably 0.3 g/m² to 3.0 g/m².

The film thickness of the image-recording layer in the lithographic printing plate precursor according to the present disclosure is preferably 0.1 µm to 3.0 µm, and more preferably 0.3 µm to 2.0 µm.

In the present disclosure, the film thickness of each layer in the lithographic printing plate precursor is checked by preparing a slice by cutting the lithographic printing plate precursor in a direction perpendicular to the surface of the precursor and observing the cross section of the slice with a scanning electron microscope (SEM).

### <Support>

The lithographic printing plate precursor according to the present disclosure has a support.

The support to be used can be appropriately selected from known supports for a lithographic printing plate precursor.

As the support, a support having a hydrophilic surface (hereinafter, also called "hydrophilic support") is preferable.

As the support in the present disclosure, an aluminum plate is preferable which has been roughened using a known method and has undergone an anodization treatment. That is, the support in the present disclosure preferably has an aluminum plate and an anodic oxide film of aluminum disposed on the aluminum plate.

The aforementioned support preferably has an aluminum plate and an anodic oxide film of aluminum disposed on the aluminum plate, the anodic oxide film is preferably at a position closer to a side of the image-recording layer than the aluminum plate and preferably has micropores extending in a depth direction from the surface of the anodic oxide film on the side of the image-recording layer, and the average diameter of the micropores within the surface of the anodic oxide film is preferably more than 10 nm and 100 nm or less.

Furthermore, the micropores are preferably each composed of a large diameter portion that extends to a position at a depth of 10 nm to 1,000 nm from the surface of the anodic oxide film and a small diameter portion that is in communication with a bottom portion of the large diameter portion and extends to a position at a depth of 20 nm to 2,000 nm from a communicate position, an average diameter of the large diameter portion within the surface of the anodic oxide film is preferably 15 nm to 100 nm, and an average diameter of the small diameter portion at the communicate position is preferably 15 nm or less.

Fig. 1 is a schematic cross-sectional view of an embodiment of an aluminum support 12a.

The aluminum support 12a has a laminated structure in which an aluminum plate 18 and an anodic oxide film 20a of aluminum (hereinafter, also simply called "anodic oxide film 20a") are laminated in this order. The anodic oxide film 20a in the aluminum support 12a is positioned such that the anodic oxide film 20a is closer to the image-recording layer side than the aluminum plate 18. That is, it is preferable that the lithographic printing plate precursor according to the present disclosure have at least an anodic oxide film, an image-recording layer, and a water-soluble resin layer in this order on an aluminum plate.

### -Anodic oxide film-

Hereinafter, preferred aspects of the anodic oxide film 20a will be described.

The anodic oxide film 20a is a film prepared on a surface of the aluminum plate 18 by an anodization treatment. This film has uniformly distributed ultrafine micropores 22a approximately perpendicular to the surface of the film. The micropores 22a extend from a surface of the anodic oxide film 20a on the image-recording layer side (a surface of the anodic oxide film 20a opposite to the aluminum plate 18) along the thickness direction (toward the aluminum plate 18).

The average diameter (average opening diameter) of the micropores 22a within the surface of the anodic oxide film 20a is preferably more than 10 nm and 100 nm or less. Particularly, from the viewpoint of balance between printing durability, antifouling properties, and image visibility, the average diameter of the micropores 22a is more preferably 15 nm to 60 nm, even more preferably 20 nm to 50 nm, and particularly preferably 25 nm to 40 nm. The internal diameter of the pores may be larger or smaller than the pore diameter within the surface layer.

In a case where the average diameter is more than 10 nm, printing durability and image visibility are excellent. Furthermore, in a case where the average diameter is 100 nm or less, printing durability is excellent.

The average diameter of the micropores 22a is a value determined by observing the surface of the anodic oxide film 20a with a field emission scanning electron microscope (FE-SEM) at 150,000× magnification (N = 4), measuring the size (diameter) of 50 micropores existing in a range of 400 nm × 600 nm² in the obtained 4 images, and calculating the arithmetic mean thereof.

In a case where the shape of the micropores 22a is not circular, the equivalent circle diameter is used. "Equivalent circle diameter" is a diameter determined on an assumption that the opening portion is in the form of a circle having the same projected area as the projected area of the opening portion.

The shape of the micropores 22a is not particularly limited. In Fig. 1, the micropores 22a have a substantially straight tubular shape (substantially cylindrical shape). However, the micropores 22a may have a conical shape that tapers along the depth direction (thickness direction). The shape of the bottom portion of the micropores 22a is not particularly limited, and may be a curved (convex) or planar surface shape.

In the support (1), the micropores may be each composed of a large diameter portion that extends to a position at a certain depth from the surface of the anodic oxide film and a small diameter portion that is in communication with a bottom portion of the large diameter portion and extends to a position at a certain depth from the communicate position.

For example, as shown in Fig. 2, an aspect may be adopted in which an aluminum support 12b includes an aluminum plate 18 and an anodic oxide film 20b having micropores 22b each composed of a large diameter portion 24 and a small diameter portion 26.

For example, the micropores 22b in the anodic oxide film 20b are each composed of the large diameter portion 24 that extends to a position at a depth of 10 nm to 1,000 nm (depth D: see Fig. 2) from the surface of the anodic oxide film and the small diameter portion 26 that is in communication with the bottom portion of the large diameter portion 24 and further extends from the communicate position to a position at a depth of 20 nm to 2,000 nm. Specifically, for example, it is possible to use the aspect described in paragraphs "0107" to "0114" of JP2019-162855A.

### -Manufacturing method of support-

As a manufacturing method of the support used in the present disclosure, for example, a manufacturing method is preferable in which the following steps are sequentially performed.
·Roughening treatment step: step of performing roughening treatment on aluminum plate
·Anodization treatment step: step of subjecting aluminum plate having undergone roughening treatment to anodization
·Pore widening treatment step: step of bringing aluminum plate having anodic oxide film obtained by anodization treatment step into contact with aqueous acid solution or aqueous alkali solution such that diameter of micropores in anodic oxide film increases

Hereinafter, the procedure of each step will be specifically described.

### <<Roughening treatment step>>

The roughening treatment step is a step of performing a roughening treatment including an electrochemical roughening treatment on the surface of the aluminum plate. This step is preferably performed before the anodization treatment step which will be described later. However, in a case where the surface of the aluminum plate already has a preferable shape, the roughening treatment step may not be performed. This step can be carried out by the method described in paragraphs "0086" to "0101" of JP2019-162855A.

### <<Anodization treatment step>>

The procedure of the anodization treatment step is not particularly limited as long as the aforementioned micropores can be obtained. Examples thereof include known methods.

In the anodization treatment step, an aqueous solution of sulfuric acid, phosphoric acid, oxalic acid, or the like can be used as an electrolytic cell. For example, the concentration of sulfuric acid is 100 g/L to 300 g/L.

The conditions of the anodization treatment are appropriately set depending on the electrolytic solution used. For example, the liquid temperature is 5°C to 70°C (preferably 10°C to 60°C), the current density is 0.5 A/dm² to 60 A/dm² (preferably 1 A/dm² to 60 A/dm²), the voltage is 1 V to 100 V (preferably 5 V to 50 V), the electrolysis time is 1 second to 100 seconds (preferably 5 seconds to 60 seconds), and the film amount is 0.1 g/m² to 5 g/m² (preferably 0.2 g/m² to 3 g/m²).

### <<Pore widening treatment>>

The pore widening treatment is a treatment of enlarging the diameter of micropores (that is, the pore diameter) present in the anodic oxide film formed by the aforementioned anodization treatment step (that is, the pore diameter enlarging treatment).

The pore widening treatment can be carried out by bringing the aluminum plate obtained by the anodization treatment step into contact with an aqueous acid solution or an aqueous alkali solution. The contact method is not particularly limited, and examples thereof include a dipping method and a spraying method.

As necessary, the support may have a backcoat layer on the side opposite to the image-recording layer, the backcoat layer containing the organic polymer compound described in JP1993-45885A (JP-H5-45885A) or the alkoxy compound of silicon described in JP1994-35174A(JP-H6-35174A).

### <Undercoat layer>

The lithographic printing plate precursor according to the present disclosure preferably has an undercoat layer (also called interlayer in some cases) between the image-recording layer and the support. The undercoat layer enhances the adhesion between the support and the image-recording layer in an exposed portion, and enables the image-recording layer to be easily peeled from the support in a non-exposed portion. Therefore, the undercoat layer contributes to the improvement of developability without deteriorating printing durability. Furthermore, in the case of exposure to infrared laser, the undercoat layer functions as a heat insulating layer and thus brings about an effect of preventing sensitivity reduction resulting from the diffusion of heat generated by exposure to the support.

Examples of compounds that are used in the undercoat layer include polymers having adsorbent groups that can be adsorbed onto the surface of the support and hydrophilic groups. In order to improve adhesiveness to the image-recording layer, polymers having adsorbent groups and hydrophilic groups plus crosslinking groups are preferable. The compounds that are used in the undercoat layer may be low-molecular-weight compounds or polymers. As necessary, as the compounds that are used in the undercoat layer, two or more kinds of compounds may be used by being mixed together.

In a case where the compound used in the undercoat layer is a polymer, a copolymer of a monomer having an adsorbent group, a monomer having a hydrophilic group, and a monomer having a crosslinking group is preferable.

As the adsorbent group that can be adsorbed onto the surface of the support, a phenolic hydroxyl group, a carboxy group, -PO₃H₂, -OPO₃H₂, -CONHSO₂-, -SO₂NHSO₂-, and -COCH₂COCH₃ are preferable. As the hydrophilic groups, a sulfo group or salts thereof and salts of a carboxy group are preferable. As the crosslinking groups, an acryloyl group, a methacryloyl group, an acrylamide group, a methacrylamide group, an allyl group, and the like are preferable.

The polymer may have a crosslinking group introduced by the formation of a salt of a polar substituent of the polymer and a compound that has a substituent having charge opposite to that of the polar substituent and an ethylenically unsaturated bond, or may be further copolymerized with monomers other than the monomers described above and preferably with hydrophilic monomers.

Specifically, for example, silane coupling agents having addition polymerizable ethylenic double bond reactive groups described in JP1998-282679A (JP-H10-282679A) and phosphorus compounds having ethylenic double bond reactive groups described in JP1990-304441A (JP-H2-304441A) are suitable. The low-molecular-weight compounds or polymer compounds having crosslinking groups (preferably ethylenically unsaturated bonding groups), functional groups that interact with the surface of the support, and hydrophilic groups described in JP2005-238816A, JP2005-125749A, JP2006-239867A, and JP2006-215263A are also preferably used.

For example, the high-molecular-weight polymers having adsorbent groups that can be adsorbed onto the surface of the support, hydrophilic groups, and crosslinking groups described in JP2005-125749A and JP2006-188038A are more preferable.

The content of ethylenically unsaturated bonding group in the polymer used in the undercoat layer is preferably 0.1 mmol to 10.0 mmol per gram of the polymer, and more preferably 0.2 mmol to 5.5 mmol per gram of the polymer.

The weight-average molecular weight (Mw) of the polymer used in the undercoat layer is preferably 5,000 or more, and more preferably 10,000 to 300,000.

### -Hydrophilic compound-

From the viewpoint of developability, it is preferable that the undercoat layer contain a hydrophilic compound.

The hydrophilic compound is not particularly limited, and known hydrophilic compounds used for the undercoat layer can be used.

Preferred examples of the hydrophilic compound include phosphonic acids having an amino group such as carboxymethyl cellulose and dextrin, an organic phosphonic acid, an organic phosphoric acid, an organic phosphinic acid, amino acids, a hydrochloride of an amine having a hydroxy group, and the like.

In addition, examples of preferable hydrophilic compounds include a compound having an amino group or a functional group capable of inhibiting polymerization and a group that interacts with the surface of the support (for example, 1,4-diazabicyclo[2.2.2]octane (DABCO), 2,3,5,6-tetrahydroxy-p-quinone, chloranil, sulfophthalic acid, ethylenediaminetetraacetic acid (EDTA) or a salt thereof, hydroxyethyl ethylenediaminetriacetic acid or a salt thereof, dihydroxyethyl ethylenediaminediacetic acid or a salt thereof, hydroxyethyl iminodiacetic acid or a salt thereof, and the like).

From the viewpoint of scratch and contamination suppressiveness, it is preferable that the hydrophilic compound include hydroxycarboxylic acid or a salt thereof.

Furthermore, from the viewpoint of scratch and contamination suppressiveness, it is preferable that the hydrophilic compound, which is preferably hydroxycarboxylic acid or a salt thereof, be contained in a layer on the aluminum support. The layer on the aluminum support is preferably a layer on the side where the image-recording layer is formed or a layer in contact with the aluminum support.

Preferred examples of the layer on the aluminum support include a layer in contact with the aluminum support, such as the undercoat layer or the image-recording layer. Furthermore, a layer other than the layer in contact with the aluminum support, for example, the protective layer or the image-recording layer may contain a hydrophilic compound and preferably contains hydroxycarboxylic acid or a salt thereof.

In the lithographic printing plate precursor according to the present disclosure, from the viewpoint of scratch and contamination suppressiveness, it is preferable that the image-recording layer contain hydroxycarboxylic acid or a salt thereof.

Moreover, regarding the lithographic printing plate precursor according to the present disclosure, for example, an aspect is also preferable in which the surface of the aluminum support on the image-recording layer side is treated with a composition (for example, an aqueous solution or the like) containing at least hydroxycarboxylic acid or a salt thereof. In a case where the above aspect is adopted, at least some of the hydroxycarboxylic acid or a salt thereof used for treatment can be detected in a state of being contained in the layer on the image-recording layer side (for example, the image-recording layer or the undercoat layer) that is in contact with the aluminum support.

In a case where the layer on the side of the image-recording layer that is in contact with the aluminum support, such as the undercoat layer, contains hydroxycarboxylic acid or a salt thereof, the surface of the aluminum support on the image-recording layer side can be hydrophilized, and it is easy for the surface of the aluminum support on the image-recording layer side to have a water contact angle of 110° or less measured by an airborne water droplet method, which result in excellent scratch and contamination suppressiveness.

"Hydroxycarboxylic acid" is the generic term for organic compounds having one or more carboxy groups and one or more hydroxy groups in one molecule. These compounds are also called hydroxy acid, oxy acid, oxycarboxylic acid, or alcoholic acid (see Iwanami Dictionary of Physics and Chemistry, 5th Edition, published by Iwanami Shoten, Publishers.

(1998)). The hydroxycarboxylic acid or a salt thereof is preferably represented by Formula (HC).

R^{HC}(OH)_{mhc}(COOM^{HC})_{nhc} Formula (HC)

In Formula (HC), R^{HC} represents an (mhc + nhc)-valent organic group, M^{HC} each independently represent a hydrogen atom, an alkali metal, or an onium, and mhc and nhc each independently represent an integer of 1 or more. In a case where n is 2 or more, Ms may be the same as or different from each other.

Examples of the (mhc + nhc)-valent organic group represented by R^{HC} in Formula (HC) include an (mhc + nhc)-valent hydrocarbon group and the like. The hydrocarbon group may have a substituent and/or a linking group.

Examples of the hydrocarbon group include an (mhc + nhc)-valent group derived from aliphatic hydrocarbon, such as an alkylene group, an alkanetriyl group, an alkanetetrayl group, an alkanepentayl group, an alkenylene group, an alkenetriyl group, an alkenetetrayl group, and alkenepentayl group, an alkynylene group, an alkynetriyl group, alkynetetrayl group, or an alkynepentayl group, an (mhc + nhc)-valent group derived from aromatic hydrocarbon, such as an arylene group, an arenetriyl group, an arenetetrayl group, or an arenepentayl group, and the like. Examples of the substituent include an alkyl group, an alkenyl group, an alkynyl group, an aralkyl group, an aryl group, and the like. Specific examples of the substituent include a methyl group, an ethyl group, a propyl group, a butyl group, a pentyl group, a hexyl group, a heptyl group, an octyl group, a nonyl group, a decyl group, an undecyl group, a dodecyl group, a tridecyl group, a hexadecyl group, an octadecyl group, eicosyl group, isopropyl group, isobutyl group, s-butyl group, t-butyl group, isopentyl group, a neopentyl group, a 1-methylbutyl group, an isohexyl group, a 2-ethylhexyl group, a 2-methylhexyl group, a cyclohexyl group, a cyclopentyl group, a 2-norbornyl group, a methoxymethyl group, a methoxyethoxyethyl group, an allyloxymethyl group, a phenoxymethyl group, an acetyloxymethyl group, a benzoyloxymethyl group, a benzyl group, a phenethyl group, an α-methylbenzyl group, a 1-methyl-1-phenylethyl group, a p-methylbenzyl group, a cinnamyl group, an allyl group, a 1-propenylmethyl group, a 2-butenyl group, a 2-methylallyl group, a 2-methylpropenylmethyl group, a 2-propynyl group, a 2-butynyl group, a 3-butynyl group, a phenyl group, a biphenyl group, a naphthyl group, a tolyl group, a xylyl group, a mesityl group, a cumenyl group, a methoxyphenyl group, an ethoxyphenyl group, a phenoxyphenyl group, an acetoxyphenyl group, a benzoyloxyphenyl group, a methoxycarbonylphenyl group, an ethoxycarbonylphenyl group, a phenoxycarbonylphenyl group, and the like. Furthermore, the linking group is composed of at least one atom selected from the group consisting of a hydrogen atom, a carbon atom, an oxygen atom, a nitrogen atom, a sulfur atom, and a halogen atom, and the number of atoms is preferably 1 to 50. Specific examples thereof include an alkylene group, a substituted alkylene group, an arylene group, a substituted arylene group, and the like. The linking group may have a structure in which a plurality of these divalent groups are linked through any of an amide bond, an ether bond, a urethane bond, a urea bond, and an ester bond.

Examples of the alkali metal represented by M^{HC} include lithium, sodium, potassium, and the like. Among these, sodium is particularly preferable. Examples of the onium include ammonium, phosphonium, sulfonium, and the like. Among these, ammonium is particularly preferable.

From the viewpoint of scratch and contamination suppressiveness, M^{HC} is preferably an alkali metal or an onium, and more preferably an alkali metal.

The sum of mhc and nhc is preferably 3 or more, more preferably 3 to 8, and even more preferably 4 to 6.

The molecular weight of the hydroxycarboxylic acid or a salt thereof is preferably 600 or less, more preferably 500 or less, and particularly preferably 300 or less. The molecular weight is preferably 76 or more.

Specifically, examples of the hydroxycarboxylic acid constituting the hydroxycarboxylic acid or a salt of the hydroxycarboxylic acid include gluconic acid, glycolic acid, lactic acid, tartronic acid, hydroxybutyrate (such as 2-hydroxybutyrate, 3-hydroxybutyrate, or γ-hydroxybutyrate), malic acid, tartaric acid, citramalic acid, citric acid, isocitric acid, leucine acid, mevalonic acid, pantoic acid, ricinoleic acid, ricineraidic acid, cerebronic acid, quinic acid, shikimic acid, a monohydroxybenzoic acid derivative (such as salicylic acid, creosotic acid (homosalicylic acid, hydroxy(methyl) benzoate), vanillic acid, or syringic acid), a dihydroxybenzoic acid derivative (such as pyrocatechuic acid, resorcylic acid, protocatechuic acid, gentisic acid, or orsellinic acid), a trihydroxybenzoic acid derivative (such as gallic acid), a phenyl acetate derivative (such as mandelic acid, benzilic acid, or atrolactic acid), a hydrocinnamic acid derivative (such as melilotic acid, phloretic acid, coumaric acid, umbellic acid, caffeic acid, ferulic acid, sinapic acid, cerebronic acid, or carminic acid), and the like.

Among these, as the aforementioned hydroxycarboxylic acid or a hydroxycarboxylic acid constituting a salt of the hydroxycarboxylic acid, from the viewpoint of scratch and contamination suppressiveness, a compound having two or more hydroxy groups is preferable, a compound having 3 or more hydroxy groups is more preferable, a compound having 5 or more hydroxy groups is even more preferable, and a compound having 5 to 8 hydroxy groups is particularly preferable.

Furthermore, as a hydroxycarboxylic acid having one carboxy group and two or more hydroxy groups, gluconic acid or shikimic acid is preferable.

As hydroxycarboxylic acid having two or more carboxy groups and one hydroxy group, citric acid or malic acid is preferable.

As hydroxycarboxylic acid having two or more carboxy groups and two or more hydroxy groups, tartaric acid is preferable.

Among these, gluconic acid is particularly preferable as the aforementioned hydroxycarboxylic acid.

One kind of hydrophilic compound may be used alone, or two or more kinds of hydrophilic compounds may be used in combination.

In a case where the undercoat layer contains a hydrophilic compound, which is preferably hydroxycarboxylic acid or a salt thereof, the content of the hydrophilic compound, which is preferably hydroxycarboxylic acid or a salt thereof, with respect to the total mass of the undercoat layer is preferably 0.01% by mass to 50% by mass, more preferably 0.1% by mass to 40% by mass, and particularly preferably 1.0% by mass to 30% by mass.

In order to prevent contamination over time, the undercoat layer may contain a chelating agent, a secondary or tertiary amine, a polymerization inhibitor, and the like, in addition to the following compounds for an undercoat layer.

The undercoat layer is formed by known coating methods.

The coating amount (solid content) of the undercoat layer is preferably 0.1 mg/m² to 300 mg/m², and more preferably 5 mg/m² to 200 mg/m².

The lithographic printing plate precursor according to the present disclosure may have other layers in addition to those described above.

Known layers can be adopted as those other layers without particular limitations. For example, as necessary, a backcoat layer may be provided on a surface of the support that is opposite to the image-recording layer side.

### (Method of preparing lithographic printing plate and lithographic printing method)

The method of preparing a lithographic printing plate according to the present disclosure preferably includes a step of exposing the lithographic printing plate precursor according to the present disclosure in the shape of an image (exposure step) and a step of removing the image-recording layer in a non-image area by supplying at least one of a printing ink or dampening water on a printer (on-press development step).

The lithographic printing method according to the present disclosure preferably includes a step of exposing the lithographic printing plate precursor according to the present disclosure in the shape of an image (exposure step), a step of removing the image-recording layer in a non-image area by supplying one of a printing ink or dampening water on a printer such that a lithographic printing plate is prepared (on-press development step), and a step of performing printing by using the obtained lithographic printing plate (hereinafter, also called "printing step").

### <Exposure step>

The method of preparing a lithographic printing plate according to the present disclosure preferably includes an exposure step of exposing the lithographic printing plate precursor according to the present disclosure in the shape of an image such that an exposed portion and a non-exposed portion are formed. The lithographic printing plate precursor according to the present disclosure is preferably exposed to a laser through a transparent original picture having a linear image, a halftone dot image, or the like or exposed in the shape of an image by laser light scanning according to digital data or the like.

The wavelength of a light source to be used is preferably 750 nm to 1,400 nm. As the light source having a wavelength of 750 nm to 1,400 nm, a solid-state laser or a semiconductor laser that radiates infrared is suitable. In a case where an infrared laser is used, the output is preferably 100 mW or higher, the exposure time per pixel is preferably 20 microseconds or less, and the amount of irradiation energy is preferably 10 mJ/cm² to 300 mJ/cm². In addition, in order to shorten the exposure time, a multibeam laser device is preferably used. The exposure mechanism may be any one of an in-plane drum method, an external surface drum method, a flat head method, or the like.

The image exposure can be carried out by a common method using a platesetter or the like. In the case of on-press development, the image exposure may be carried out on a printer after the lithographic printing plate precursor is mounted on the printer.

### <On-press development step>

The method of preparing a lithographic printing plate according to the present disclosure preferably includes an on-press development step of removing the image-recording layer in a non-image area by supplying at least one selected from the group consisting of printing ink and dampening water on a printer.

Hereinafter, the on-press development method will be described.

### [On-press development method]

In the on-press development method, the lithographic printing plate precursor having undergone image exposure is preferably supplied with an oil-based ink and an aqueous component on a printer, such that the image-recording layer in a non-image area is removed and a lithographic printing plate is prepared.

That is, in a case where the lithographic printing plate precursor is subjected to image exposure and then directly mounted on a printer without being subjected to any development treatment, or in a case where the lithographic printing plate precursor is mounted on a printer, then subjected to image exposure on the printer, and then supplied with an oil-based ink and an aqueous component for printing, at the initial stage in the middle of printing, in a non-image area, a non-cured image-recording layer is removed by either or both of the supplied oil-based ink and the aqueous component by means of dissolution or dispersion, and the hydrophilic surface is exposed in the non-image area. On the other hand, in an exposed portion, the image-recording layer cured by exposure forms an oil-based ink-receiving portion having a lipophilic surface. What is supplied first to the precursor surface may be any of the oil-based ink or the aqueous component. However, in view of preventing the precursor from being contaminated by the components of the image-recording layer from which aqueous components are removed, it is preferable that the oil-based ink be supplied first. In the manner described above, the lithographic printing plate precursor is subjected to on-press development on a printer and used as it is for printing a number of sheets. As the oil-based ink and the aqueous component, ordinary printing ink and ordinary dampening water for lithographic printing are suitably used.

As the laser used for performing image exposure on the lithographic printing plate precursor according to the present disclosure, a light source having a wavelength of 750 nm to 1,400 nm is preferably used. As the light source having a wavelength of 750 nm to 1,400 nm, the light sources described above are preferably used.

### <Printing step>

The lithographic printing method according to the present disclosure includes a printing step of printing a recording medium by supplying a printing ink to a lithographic printing plate.

The printing ink is not particularly limited, and various known inks can be used as desired. In addition, preferred examples of the printing ink include oil-based ink or ultraviolet-curable ink (UV ink).

In the printing step, as necessary, dampening water may be supplied.

Furthermore, the printing step may be successively carried out after the on-press development step or the development step using a developer, without stopping the printer.

The recording medium is not particularly limited, and known recording media can be used as desired.

In the method of preparing a lithographic printing plate from the lithographic printing plate precursor according to the present disclosure and in the lithographic printing method according to the present disclosure, as necessary, the entire surface of the lithographic printing plate precursor may be heated as necessary before exposure, in the middle of exposure, or during a period of time from exposure to development. In a case where the lithographic printing plate precursor is heated as above, an image-forming reaction in the image-recording layer is accelerated, which can result in advantages such as improvement of sensitivity and printing durability, stabilization of sensitivity, and the like. Heating before development is preferably carried out under a mild condition of 150°C or lower. In a case where this aspect is adopted, it is possible to prevent problems such as curing of a non-image area. For heating after development, it is preferable to use an extremely severe condition which is preferably in a range of 100°C to 500°C. In a case where this aspect is adopted, a sufficient image-strengthening action is obtained, and it is possible to inhibit problems such as the deterioration of the support or the thermal decomposition of the image area.

### Examples

Hereinafter, the present disclosure will be specifically described based on examples, but the present disclosure is not limited thereto. In the present examples, unless otherwise specified, "%" and "part" mean "% by mass" and "part by mass" respectively. Unless otherwise described, the molecular weight of a polymer compound is a weight-average molecular weight (Mw), and the ratio of constitutional units of a polymer compound is expressed as molar percentage. The weight-average molecular weight (Mw) is a polystyrene-equivalent molecular weight measured by gel permeation chromatography (GPC).

### (Examples 1 to 29 and Comparative Examples 1 and 2)

### <Preparation of support X>

### <<Surface Treatment X»:

### [Support having large diameter portion and small diameter portion]

### (X-a) Alkaline etching treatment

An aqueous solution of caustic soda having a caustic soda (sodium hydroxide) concentration of 26% by mass and an aluminum ion concentration of 6.5% by mass was sprayed from a spray tube onto the aluminum plate at a temperature of 70°C, thereby performing an etching treatment. Then, rinsing was performed by means of spraying. The amount of dissolved aluminum within the surface to be subjected to the electrochemical roughening treatment later was 1.0 g/m².

### (X-b) Desmutting treatment in aqueous acidic solution (first desmutting treatment)

Next, a desmutting treatment was performed in an aqueous acidic solution. In the desmutting treatment, a 150 g/L aqueous sulfuric acid solution was used as the aqueous acidic solution. The liquid temperature was 30°C. The desmutting treatment was performed for 3 seconds by spraying the desmutting liquid. Then, a rinsing treatment was performed.

### (X-c) Electrochemical roughening treatment in aqueous hydrochloric acid solution

Next, an electrolytic roughening treatment was performed using alternating current and an electrolytic solution having a hydrochloric acid concentration of 14 g/L, an aluminum ion concentration of 13 g/L, and a sulfuric acid concentration of 3 g/L. The liquid temperature of the electrolytic solution was 30°C. The aluminum ion concentration was adjusted by adding aluminum chloride. The waveform of the alternating current was a sine wave in which positive and negative waveforms are symmetrical, the frequency was 50 Hz, the ratio of the anodic reaction time and the cathodic reaction time in one cycle of the alternating current was 1:1, and the current density was 75 A/dm² in terms of the peak current value of the alternating current waveform. In addition, the quantity of electricity was 450 C/dm² which was the total quantity of electricity used for the aluminum plate to have an anodic reaction, and the electrolysis treatment was performed 4 times by conducting electricity of 125 C/dm² for 4 seconds at each treatment session. A carbon electrode was used as the counter electrode of the aluminum plate. Then, a rinsing treatment was performed.

### (X-d) Alkaline etching treatment

An aqueous solution of caustic soda having a caustic soda concentration of 5% by mass and an aluminum ion concentration of 0.5% by mass was sprayed from a spray tube onto the aluminum plate having undergone the electrochemical roughening treatment at a temperature of 45°C, thereby performing an etching treatment. The amount of dissolved aluminum within the surface having undergone the electrochemical roughening treatment was 0.2 g/m². Then, a rinsing treatment was performed.

### (X-e) Desmutting treatment in aqueous acidic solution

Next, a desmutting treatment was performed in an aqueous acidic solution. In the desmutting treatment, as an aqueous acidic solution, a waste liquid was used which was generated in the anodization treatment step (170 g/L aqueous sulfuric acid solution containing dissolved aluminum ions at 5.0 g/L). The liquid temperature was 30°C. The desmutting treatment was performed for 3 seconds by spraying the desmutting liquid.

### (X-f) First-stage anodization treatment

By using the anodization device for direct current electrolysis having the structure shown in Fig. 3, a first-stage anodization treatment was performed. The anodization treatment was performed under the conditions shown in Table 1, thereby forming an anodic oxide film having a predetermined film thickness.

In the anodization treatment device 610, an aluminum plate 616 is transported as indicated by the arrow in Fig. 3. In a power supply tank 612 containing an electrolytic solution 618, the aluminum plate 616 is positively (+) charged by a power supply electrode 620. Then, the aluminum plate 616 is transported upwards by a roller 622 in the power supply tank 612, makes a turn downwards by a nip roller 624, then transported toward an electrolytic treatment tank 614 containing an electrolytic solution 626, and makes a turn by a roller 628 to move in the horizontal direction. Subsequently, the aluminum plate 616 is negatively (-) charged by an electrolysis electrode 630. As a result, an anodic oxide film is formed on the surface of the aluminum plate 616. The aluminum plate 616 exits from the electrolytic treatment tank 614 and is then transported for the next step. In the anodization treatment device 610, the roller 622, the nip roller 624, and the roller 628 constitute a direction change unit. Furthermore, in the inter-tank portion between the power supply tank 612 and the electrolytic treatment tank 614, the aluminum plate 616 is transported in a ridge shape and an inverted U shape by the rollers 622, 624, and 628. The power supply electrode 620 and the electrolysis electrode 630 are connected to a direct current power source 634.

### (X-g) Pore widening treatment

Under the conditions shown in Table 1, the aluminum plate having undergone the above anodization treatment was immersed in an aqueous solution of caustic soda at a temperature of 35°C and having a caustic soda concentration of 5% by mass and an aluminum ion concentration of 0.5% by mass, thereby performing a pore widening treatment. Then, rinsing was performed by means of spraying.

### (X-h) Second-stage anodization treatment

By using the anodization device for direct current electrolysis having the structure shown in Fig. 3, a second-stage anodization treatment was performed. The anodization treatment was performed under the conditions shown in Table 1, thereby forming an anodic oxide film having a predetermined film thickness.

### A support X was obtained by the surface treatment X.

Table 2 shows the average diameter (nm) of the large diameter portion in the anodic oxide film within the surface of the anodic oxide film having micropores obtained after the second-stage anodization treatment step, the average diameter (nm) of the small diameter portion at a communicate position, the depth (nm) of the large diameter portion and the small diameter portion, the pit density (micropore density, unit; number of micropores/µm²), and the thickness (nm) of the anodic oxide film from the bottom portion of the small diameter portion to the surface of the aluminum plate.

The average diameter of the micropores (average diameter of the large diameter portion and the small diameter portion) is a value obtained by observing the surface of the large diameter portion and the surface of the small diameter portion with FE-SEM at 150,000× magnification (N= 4), and measuring the diameters of micropores (large diameter portion and small diameter portion) in a range of 400 nm × 600 nm in the obtained 4 images, and calculating the average thereof. In a case where the large diameter portion was deep and it was difficult to measure the diameter of the small diameter portion, and in a case where an enlarged diameter portion in the small diameter portion was measured, the upper portion of the anodic oxide film was cut, and then various diameters were calculated.

The depth of the micropores (depth of the large diameter portion and the small diameter portion) is a value obtained by observing the cross section of the support (anodic oxide film) with FE-SEM (observation of the depth of the large diameter portion: 150,000× magnification, observation of the depth of the small diameter portion: 50,000× magnification), measuring the depths of 25 random micropores in the obtained image, and calculating the average thereof.

In Table 1, Film amount (AD) in the column of First-stage anodization treatment and Film amount (AD) in the column of Second-stage anodization treatment represent the amount of film obtained by each treatment. As electrolytic solutions, the aqueous solutions containing the components in Table 1 were used.

In Table 1, "170/5" in the column of component concentration means that the sulfuric acid concentration is 170 g/L and the aluminum ion concentration is 5 g/L. Furthermore, in Table 1, the unit of temperature is "°C", the unit of current density is "A/dm²", the unit of time is "s", and the unit of film amount is "G/m²".

### <Preparation of support Y>

### <<Treatment Y> >

### (Y-a) Alkaline etching treatment

An aqueous solution of caustic soda having a caustic soda concentration of 26% by mass and an aluminum ion concentration of 6.5% by mass was sprayed onto the aluminum plate at a temperature of 70°C, thereby performing an etching treatment. Then, rinsing was performed by means of spraying. The amount of dissolved aluminum within the surface to be subjected to the electrochemical roughening treatment later was 5 g/m².

### (Y-b) Desmutting treatment using aqueous acidic solution (first desmutting treatment)

Next, a desmutting treatment was performed using an aqueous acidic solution. In the desmutting treatment, a 150 g/L aqueous sulfuric acid solution was used as the aqueous acidic solution. The liquid temperature was 30°C. The desmutting treatment was performed for 3 seconds by spraying the aqueous acidic solution onto the aluminum plate. Then, a rinsing treatment was performed.

### (Y-c) Electrochemical roughening treatment

Next, an electrochemical roughening treatment was performed using alternating current and an electrolytic solution having a hydrochloric acid concentration of 14 g/L, an aluminum ion concentration of 13 g/L, and a sulfuric acid concentration of 3 g/L. The liquid temperature of the electrolytic solution was 30°C. The aluminum ion concentration was adjusted by adding aluminum chloride.

The waveform of the alternating current was a sine wave in which positive and negative waveforms are symmetrical, the frequency was 50 Hz, the ratio of the anodic reaction time and the cathodic reaction time in one cycle of the alternating current was 1:1, and the current density was 75 A/dm² in terms of the peak current value of the alternating current waveform. In addition, the quantity of electricity was 450 C/dm² which was the total quantity of electricity used for the aluminum plate to have an anodic reaction, and the electrolysis treatment was performed 4 times by conducting electricity of 112.5 C/dm² for 4 seconds at each treatment session. A carbon electrode was used as the counter electrode of the aluminum plate. Then, a rinsing treatment was performed.

### (Y-d) Alkaline etching treatment

An aqueous solution of caustic soda having a caustic soda concentration of 5% by mass and an aluminum ion concentration of 0.5% by mass was sprayed onto the aluminum plate having undergone the electrochemical roughening treatment at a temperature of 45°C, thereby performing an etching treatment. The amount of dissolved aluminum within the surface having undergone the electrochemical roughening treatment was 0.2 g/m². Then, a rinsing treatment was performed.

### (Y-e) Desmutting treatment using aqueous acidic solution

Next, a desmutting treatment was performed using an aqueous acidic solution. Specifically, the desmutting treatment was performed for 3 seconds by spraying the aqueous acidic solution onto the aluminum plate. In the desmutting treatment, an aqueous solution having a sulfuric acid concentration of 170 g/L and an aluminum ion concentration of 5 g/L was used as aqueous acidic solution. The liquid temperature was 30°C.

### (A-f) First-stage anodization treatment

By using the anodization device for direct current electrolysis having the structure shown in Fig. 3, a first-stage anodization treatment was performed. The anodization treatment was performed under the conditions described in the column of "First anodization treatment" shown in Table 3, thereby forming an anodic oxide film having a predetermined film amount.

### (Y-g) Pore widening treatment

The aluminum plate having undergone the above anodization treatment was immersed in an aqueous solution of caustic soda at a temperature of 40°C and having a caustic soda concentration of 5% by mass and an aluminum ion concentration of 0.5% by mass under the time conditions shown in Table 3, thereby performing a pore widening treatment. Then, rinsing was performed by means of spraying.

### (Y-h) Second-stage anodization treatment

By using the anodization device for direct current electrolysis having the structure shown in Fig. 3, a second-stage anodization treatment was performed. The anodization treatment was performed under the conditions described in the column of "Second anodization treatment" shown in Table 3, thereby forming an anodic oxide film having a predetermined film amount.

A support Y was obtained by the surface treatment Y

### <Method of forming undercoat layer>

The supports described in Tables 4 to 6 were coated with the coating liquid C or B for an undercoat layer described in Tables 4 to 6 having the following compositions such that the dry coating amount of 20 mg/m² was obtained, and the supports were dried in an oven at 100°C for 30 seconds, thereby forming an undercoat layer.

### -Composition of coating liquid C for undercoat layer-

·Polymer (U-1) [the following structure]: 0.14 parts
·Chelest 400: 0.035 parts
·Chelest 3EAF: 0.035 parts
·Surfactant (EMALEX 710, manufactured by NIHON EMULSION Co., Ltd.): 0.0016 parts
·Preservative (BIOHOPE L, manufactured by K·I Chemical Industry Co., LTD.): 0.0015 parts
·Water: 3.29 parts

### -Composition of coating liquid B for undercoat layer-

·Polymer (U-1) [the following structure]: 0.18 parts
·Hydroxyethyl iminodiacetic acid: 0.10 parts
·Water: 61.4 parts

### -Synthesis of polymer (U-1)-

### «Purification of monomer M-1»

LIGHT ESTER P-1M (2-methacryloyloxyethyl acid phosphate, manufactured by KYOEISHA CHEMICAL Co., LTD.) (420 parts), 1,050 parts of diethylene glycol dibutyl ether, and 1,050 parts of distilled water were added to a separating funnel, vigorously stirred, and then left to stand. The upper layer was discarded, 1,050 parts of diethylene glycol dibutyl ether was then added thereto, the solution was vigorously stirred, and then left to stand. The upper layer was discarded, thereby obtaining 1,300 parts of an aqueous solution of a monomer M-1 (10.5% by mass in terms of solid content).

### <<Synthesis of polymer (U-1)>>

Distilled water (53.73 parts) and 3.66 parts of Monomer M-2 were added to a three-neck flask, and heated to 55°C in a nitrogen atmosphere. Then, the following dripping liquid 1 was added dropwise thereto for 2 hours, the obtained solution was stirred for 30 minutes, and 0.386 parts of VA-046B (manufactured by FUJIFELM Wako Pure Chemical Corporation) was added thereto. The solution was heated to 80°C and stirred for 1.5 hours. The reaction solution was returned to room temperature (25°C), a 30% by mass aqueous sodium hydroxide solution was added thereto such that the pH was adjusted to 8.0, and then 0.005 parts of 4-hydroxy-2,2,6,6-tetramethylpiperidin-1-oxyl (4-OH-TEMPO) was added thereto. By the above operation, 180 parts of an aqueous solution of a polymer (U-1) was obtained. The polyethylene glycol-equivalent weight-average molecular weight (Mw) thereof that was measured by gel permeation chromatography (GPC) was 200,000.

### <<Composition of dripping liquid 1»

·Aqueous solution of the monomer M-1: 87.59 parts
·The above monomer M-2: 14.63 parts
·VA-046B (2,2'-azobis[2-(2-imidazolin-2-yl)propane]disulfate dihydrate, manufactured by FUJIFILM Wako Pure Chemical Corporation): 0.386 parts
·Distilled water: 20.95 parts

### <Formation of image-recording layer>

By bar coating, the support or the undercoat layer was coated with a coating liquid for an image-recording layer having the composition described in Tables 4 to 6 (here, the coating liquid for an image-recording layer contained the components described in Tables 4 and 6, and the solid contents thereof were adjusted to 6% by mass by using a mixed solvent of 1-methoxy-2-propanol (MFG):methyl ethyl ketone (MEK):methanol = 4: 4:1 (mass ratio)). The support or the undercoat layer was dried in an oven at 120°C for 40 seconds, thereby forming an image-recording layer having a dry coating amount described in Tables 4 to 6.

Each component used in the image-recording layer will be shown below.

### [Infrared absorber]

D-1 to D-3: compounds having the following structures

Bu represents a n-butyl group, and TsO⁻ represents a tosylate anion.

### [Electron-accepting polymerization initiator]

I-1: compound having the following structure, TsO⁻ represents a tosylate anion.
I-2: compound having the following structure

### [Acid color developing agent]

SA-1: the following compound
SA-2: the following compound

### [Electron-donating polymerization initiator]

### B-1: compound having the following structure

### [Polymerizable compound]

M-1: urethane acrylate synthesized according to the following synthesis method
M-2: Ethoxylated isocyanuric acid triacrylate, A-9300 manufactured by SHIN-NAKAMURA CHEMICAL CO, LTD.
M-3: the following compound
M-4: the following compound

### <Synthesis of M-1>

A mixed solution was heated to 65°C which was composed of TAKENATE (registered trademark) D-160N (ethyl acetate solution of a trimethylolpropane adduct of hexamethylene diisocyanate (concentration of solid contents: 75% by mass), manufactured by Mitsui Chemicals, Inc.), 4.7 parts by mass,

ARONIX (registered trademark) M-405 (dipentaerythritol penta- and hexa-acrylate, manufactured by TOAGOSEI CO., LTD.) in an amount in which the ratio of NCO value of polyisocyanate and the hydroxyl number of hydroxyl group-containing polyfunctional acrylate is 1:1, 0.02 parts by mass of t-butylbenzoquinone, and 11.5 parts by mass of methyl ethyl ketone.

NEOSTANN (registered trademark) U-600 (bismuth-based polycondensation catalyst, manufactured by NITTO KASEI CO., LTD., 0.11 parts by mass) was added to the reaction solution, and the reaction solution was heated at the same temperature for 4 hours.

The reaction solution was cooled to room temperature (25°C), and methyl ethyl ketone was added thereto, thereby synthesizing a urethane acrylate solution having a solid content of 50% by mass.

The representative structure of urethane acrylate contained in M-1 is shown below as an example.

### [Polymer particles]

R-1: polymer particles prepared as below
R-2: polymer particles prepared as below

### <Preparation of polymer particles R-1>

·Microgel (polymer particles R-1): 2.640 parts
·Distilled water: 2.425 parts

The microgel was prepared by the following method.

### -Preparation of polyvalent isocyanate compound-

Bismuth tris(2-ethylhexanoate) (NEOSTAN U-600, manufactured by NITTO KASEI CO., LTD., 0.043 parts) was added to an ethyl acetate (25.31 g) suspension solution of 17.78 parts (80 molar equivalents) of isophorone diisocyanate and 7.35 parts (20 molar equivalents) of Polyhydric phenol compound (1), and the obtained solution was stirred. The reaction temperature was set to 50°C at a point in time when heat release subsided, and the solution was stirred for 3 hours, thereby obtaining an ethyl acetate solution of the polyvalent isocyanate compound (1) (50% by mass).

### -Preparation of microgel-

The following oil-phase components and water-phase components were mixed together and emulsified at 12,000 rpm for 10 minutes by using a homogenizer. The obtained emulsion was stirred at 45°C for 4 hours, a 10% by mass aqueous solution of 5.20 g of 1,8-diazabicyclo[5.4.0]undec-7-ene-octylate (U-CAT SA102, manufactured by San-Apro Ltd.) was added thereto, and the solution was stirred at room temperature for 30 minutes and left to stand at 45°C for 24 hours. Distilled water was added thereto such that the concentration of solid contents was adjusted to 20% by mass, thereby obtaining an aqueous dispersion liquid of a microgel. The average particle diameter thereof measured by a light scattering method was 0.20 µm.

### -Oil-phase component-

(Component 1) ethyl acetate: 12.0 parts
(Component 2) an adduct obtained by addition of trimethylolpropane (6 molar equivalents), xylene diisocyanate (18 molar equivalents), and polyoxyethylene having one methylated terminal (1 molar equivalent, the number of repeating oxyethylene units: 90) (50% by mass ethyl acetate solution, manufactured by Mitsui Chemicals, Inc.): 3.76 parts
(Component 3) polyvalent isocyanate compound (1) (as 50% by mass ethyl acetate solution): 15.0 parts
(Component 4) 65% by mass ethyl acetate solution of dipentaerythritol pentaacrylate (SR-399, manufactured by Sartomer Company Inc.): 11.54 parts
(Component 5) 10% by mass ethyl acetate solution of sulfonate type surfactant (PIONIN A-41-C, manufactured by TAKEMOTO OIL & FAT Co., Ltd.): 4.42 parts

### -Water-phase component-

Distilled water: 46.87 parts

### <Preparation of polymer particles R-2>

### -Preparation of oil-phase component-

WANNATE (registered trademark) PM-200 (polyfunctional isocyanate compound: manufactured by Wanhua Chemical Group Co., Ltd.): 6.66 g,
TAKENATE (registered trademark) D-116N (50% by mass ethyl acetate solution of an adduct (the following structure) of trimethylolpropane (TMP), m-xylylene diisocyanate (XDI), and polyethylene glycol monomethyl ether (EO90): manufactured by Mitsui Chemicals, Inc.): 5.46 g,
65% by mass ethyl acetate solution of SR399 (dipentaerythritol pentaacrylate: manufactured by Sartomer Company Inc.): 11.24 g, ethyl acetate: 14.47 g, and
PIONIN (registered trademark) A-41-C (manufactured by TAKEMOTO OIL & FAT CO., LTD.): 0.45 g
were mixed together and stirred at room temperature (25°C) for 15 minutes, thereby obtaining an oil-phase component.

### -Preparation of water-phase component-

As a water-phase component, 47.2 g of distilled water was prepared.

### -Particle forming step-

The oil-phase component and the water-phase component were mixed together, and the obtained mixture was emulsified at 12,000 rpm for 16 minutes by using a homogenizer, thereby obtaining an emulsion.

Distilled water (16.8 g) was added to the obtained emulsion, and the obtained liquid was stirred at room temperature for 180 minutes.

After stirring, the liquid was heated at 45°C, and stirred for 5 hours in a state of being kept at 45°C such that ethyl acetate was distilled away from the liquid. BIOHOPE (registered trademark) (antifungal preservative: manufactured by K·I Chemical Industry Co., LTD.): 13 mg was added thereto, and then the concentration of solid contents was adjusted to 20% by mass by using distilled water, thereby obtaining an aqueous dispersion liquid of polymer particles R-2. R-2 had a volume average particle diameter of 165 nm that was measured using a laser diffraction/scattering-type particle diameter distribution analyzer LA-920 (manufactured by HORIBA, Ltd.).

### [Binder polymer]

P-1: partially acetylated polyvinyl acetal, S-LEC BL10 manufactured by SEKISUI CHEMICAL CO., LTD.

### [Hydrophilic compound]

### T-1: compound having the following structure

### [Additive]

O-1: compound having the following structure
O-2: compound having the following structure

### [Surfactant]

### U-1 and U-2: the following compounds

### <Formation of outermost layer>

The image-recording layer was bar-coated with the coating liquid for an outermost layer composed as described in Tables 4 to 6 (here, the coating liquid for an outermost layer contained the components described in Tables 4 to 6, the solid content thereof was adjusted to 6% by mass by using deionized water), followed by drying in an oven at 120°C for 60 seconds, thereby forming an outermost layer having a dry coating amount described in Tables 4 to 6.

Through the above steps, lithographic printing plate precursors of examples and comparative examples were obtained.

Each component used in the outermost layer will be shown below.

### [Water-soluble polymer]

WP-1: Polyvinyl alcohol, GOHSENOL L-3266 manufactured by Mitsubishi Chemical Corporation., saponification degree of 86% to 89% or higher
WP-2: Mowiol 4-88 (polyvinyl alcohol (PVA), manufactured by Sigma-Aldrich Co. LLC.)
WP-3: Mowiol 8-88 (polyvinyl alcohol (PVA), manufactured by Sigma-Aldrich Co. LLC.)

### [Hydrophobic polymer particles]

WR-1: styrene-acrylic resin particles, FS-102 manufactured by Nippon paint Industrial Coatings Co., LTD., Tg = 103°C
WR-2: Aqueous polyvinylidene chloride dispersion, Diofan (registered trademark) A50 manufactured by Solvin S.A.
WR-3: same particles as polymer particles R-2
WR-4: same particles as polymer particles R-1
WR-5: PARTICLES prepared as below
WR-6: MP-1451 (anion-dispersible non-crosslinked acrylic particles having glass transition temperature of 128°C: manufactured by Soken Chemical & Engineering Co., Ltd.)
WR-7: particles prepared as below, anion-dispersible

### <Preparation of hydrophobic polymer particles WR-5>

A polyfunctional isocyanate compound (polymeric MDI WANNATE (registered trademark) PM-200: manufactured by Wanhua Chemical Group Co., Ltd.): 6.66 parts, a 50% by mass ethyl acetate solution of "TAKENATE (registered trademark) D-116N (adduct of trimethylolpropane (TMP), m-xylylene diisocyanate (XDI), and polyethylene glycol monomethyl ether (EO90) (the above structure)" manufactured by Mitsui Chemicals, Inc.: 5.46 parts, a 65% by mass ethyl acetate solution of a polymerizable compound M-1 having the following structure": 11.53 parts, ethyl acetate: 18.66 parts, and PIONIN (registered trademark) A-41-C manufactured by TAKEMOTO OIL & FAT CO., LTD.: 0.45 parts were mixed together and stirred at room temperature (25°C) for 15 minutes, thereby obtaining an oil-phase component.

As a water-phase component, pure water: 46.89 parts was added to the obtained oil-phase component and mixed together, and the obtained mixture was emulsified at 12,000 revolutions per minute (rpm) for 12 minutes by using a homogenizer, thereby obtaining an emulsion.

The obtained emulsion was added to 16.66 parts of distilled water, and stirred. Then, the obtained liquid was heated to 45°C, and stirred for 4 hours in a state of being kept at 45°C such that ethyl acetate was distilled off from the liquid. Then, the liquid from which ethyl acetate was distilled off was heated to 45°C and stirred for 48 hours in a state of being kept at 45°C, thereby obtaining microcapsule-type hydrophobic polymer particles WR-5 made of a polyaddition-type resin in a liquid. Thereafter, the liquid containing the hydrophobic polymer particles WR-5 was diluted with distilled water such that the concentration of solid contents was 20% by mass, thereby obtaining an aqueous dispersion of the hydrophobic polymer particles WR-5.

The hydrophobic polymer particles WR-5 had a volume average particle diameter of 220 nm that was measured using a laser diffraction/scattering-type particle diameter distribution analyzer LA-920 (manufactured by HORIBA, Ltd.).

The content of the polymerizable compound M-1 with respect to the total mass of the hydrophobic polymer particles WR-5 was 42% by mass.

### <Preparation of hydrophobic polymer particles WR-7>

A stirrer, a thermometer, a dropping funnel, a nitrogen introduction pipe, and a reflux condenser were installed in a four-necked flask, and nitrogen gas was introduced into the flask to perform deoxygenation. In this state, 425 ml of distilled water and 1.5 g of sodium dodecyl sulfate as a dispersant were added thereto, and the mixture was heated until the internal temperature reached 70°C. Furthermore, 1.35 g of potassium persulfate was added thereto as a polymerization initiator, and then 25 g of methyl methacrylate was added dropwise thereto from the dropping funnel for about 2 hours. After the dropwise addition, the reaction was continued as it was for 3 hours. Then, the unreacted monomer was removed by steam distillation. Thereafter, the mixture was cooled, and the pH thereof was adjusted to 6 with aqueous ammonia. Finally, pure water was added thereto such that the content of a non-volatile component was 5% by mass, thereby obtaining hydrophobic polymer particles WR-7. The average particle diameter of the polymer particles was 0.12 µm.

### [Surfactant]

V-1: polyoxyethylene lauryl ether, EMALEX 710, manufactured by Nihon Emulsion Co., Ltd.

### [Discoloring compound]

### wIR-1: the following compound

### <Evaluation of lithographic printing plate precursor>

### [Measurement of contact angle of water as a droplet of water-in-oil on surface of outermost layer]

The contact angle of water as a droplet of water-in-oil on the surface of the outermost layer was measured by the following method.

By using a contact angle meter (Model: DMC-MC3) manufactured by Kyowa Interface Science Co., Ltd., the lithographic printing plate precursor was mounted on a fixing tool and put in a glass cell filled with linseed oil to prepare a sample. At 25°C, 1 µL of pure water was added dropwise to the precursor in the linseed oil. Then, 30 seconds or 60 seconds after the pure water was added dropwise, the angle between the precursor surface and a tangent of the water droplet interface at an intersection between the landed pure water droplet and the precursor surface was measured as a contact angle. It is preferable to promptly measure the contact angle after the precursor is put in the linseed oil. The precursor left in the oil for 2 minutes or more is not suitable for the measurement. The contact angle was measured at 3 or more sites on the same precursor, and the average thereof was adopted.

### [Method of confirming sea-island structure]

The printing plate precursor was bent such that the fracture surface was exposed, and then a protective film was formed thereon by C (carbon) vapor deposition, and the printing plate precursor was observed using SU8010 type SEM manufactured by Hitachi High-Tech Corporation. (acceleration voltage: 5 kV, reflected electron mode).

### [Evaluation of on-press development residue suppressiveness]

By using Magnus 800 Quantum manufactured by Kodak Japan Ltd. that was equipped with an infrared semiconductor laser, the lithographic printing plate precursor prepared as above was exposed under the conditions of output of 27 W, an outer drum rotation speed of 450 rpm, and a resolution of 2,400 dots per inch (dpi), 1 inch is equal to 2.54 cm) (irradiation energy equivalent to 110 mJ/cm²). The exposure was performed such that the proportion of a non-image area was 70% in the image.

The obtained exposed precursor was mounted on a Kikuban-sized (636 mm × 939 mm) cylinder of a printer SX-74 manufactured by Heidelberger Druckmaschinen AG without being developed. This printer was connected to a 100 L-capacity dampening water circulation tank having a non-woven fabric filter and a temperature control device. A circulation device was filled with 80 L of dampening water containing 2.0% by mass dampening water S-Z1 (manufactured by FUJIFILM Corporation), and T&K UV OFS K-HS black GE-M (manufactured by T&K TOKA CO., LTD.) was used as printing ink. The dampening water and ink were supplied by a standard automatic printing start method, and then printing was performed on TOKUBISHI art paper (manufactured by MITSUBISHI PAPER MILLS LIMITED., ream weight: 76.5 kg) at a printing rate of 10,000 sheets/hour to perform on-press development. On-press development was performed until no ink was transferred to the non-image area. The on-press development was repeated on the same 15 precursors having undergone exposure.

After the on-press development for 15 precursors was finished, the surface of the dampening roller in the printer was observed to evaluate the deposition of development residues.

By using DYCLEAN (ink roller washing solution, manufactured by DIC Graphics Corporation) as a washing solution, a dampening roller and the like were washed according to the standard setting of the aforementioned printer.

The evaluation indices are as follows.
A: No dirt adheres to the dampening roller.
B: Although dirt adheres to a part of the dampening roller, the dirt can be washed off by rinsing the roller once.
C: Although dirt adheres to a part of the dampening roller, the dirt can be washed off by rinsing the roller 2 or 3 times.
D: Dirt adheres to the entire surface of the dampening roller, and remains on the roller even after the roller is rinsed 3 times.

### [Evaluation of on-press developability]

By using Magnus 800 Quantum manufactured by Kodak Japan Ltd. that was equipped with an infrared semiconductor laser, the lithographic printing plate precursor prepared as above was exposed under the conditions of output of 27 W, an outer drum rotation speed of 450 rpm, and a resolution of 2,400 dots per inch (dpi), 1 inch is equal to 2.54 cm) (irradiation energy equivalent to 110 mJ/cm²). The exposure images included a solid image and an amplitude modulated screening (AM screening) as a 3% halftone dot chart.

The obtained exposed precursor was mounted on a Kikuban-sized (636 mm × 939 mm) cylinder of a printer SX-74 manufactured by Heidelberger Druckmaschinen AG without being developed. This printer was connected to a 100 L-capacity dampening water circulation tank having a non-woven fabric filter and a temperature control device. A circulation device was filled with dampening water (80 L) containing 2.0% by mass dampening water S-Z1 (manufactured by FUJIFILM Corporation), and T&K UV OFS K-HS black GE-M (manufactured by T&K TOKA CO., LTD.) was used as printing ink. The dampening water and ink were supplied by a standard automatic printing start method, and then printing was performed on 500 sheets of TOKUBISHI art paper (manufactured by MITSUBISHI PAPER MILLS LIMITED., ream weight: 76.5 kg) at a printing rate of 10,000 sheets/hour.

During the on-press development described above, the number of printing papers used until no ink was transferred to a non-image area was measured as the on-press developability.

### [Evaluation of printing durability]

After the on-press developability was evaluated as above, printing was continued. As the number of printing sheets increased, the image area gradually wore out, and thus the ink density on the printed matter decreased. The area ratio of the AM screen 3% halftone dots in the printed matter was measured using a Gretag density meter (manufactured by GretagMacbeth). The number of printing sheets at a point in time when the measured area ratio was 1% lower than the area ratio measured after 500 sheets were printed was adopted as the number of sheets of completed printing and used for evaluation of printing durability. The evaluation was based on relative printing durability to 100 which represents the printing durability of a lithographic printing plate precursor capable of printing 50,000 sheets. The higher the numerical value, the better the printing durability. $Relative printing durability = \left(\begin{matrix}number of printing sheets obtained from subject \\ lithographic printing plate precursor\end{matrix}\right) / 50,000 \times 100$

### [Evaluation of receptivity]

The lithographic printing plate precursor exposed by the same method as the exposure method performed in the evaluation of on-press developability described above was mounted on a plate cylinder of a printer LITHRONE26 manufactured by KOMORI Corporation.

Dampening water composed of Ecolity-2 (manufactured by FUJIFILM Corporation)/tap water = 2/98 (volume ratio) and Values-G(N) black ink (manufactured by DIC Corporation) were supplied by the standard automatic printing start method of LITHRONE26 to perform on-press development, and then printing was performed on 100 sheets of TOKUBISHI art paper (manufactured by MITSUBISHI PAPER MILLS LIMITED., ream weight: 76.5 kg) at a printing rate of 10,000 sheets/hour.

The number of sheets of printing paper used until the density of ink transferred to the printing paper from the image area of the lithographic printing plate reached the prescribed standard density was counted.

The smaller the number of sheets of printing paper, the better the receptivity.

The evaluation results are shown in Tables 4 to 6.

The outermost layer of the lithographic printing plate precursors of Examples 1 to 29 had a sea-island structure consisting of a discontinuous phase that contains a hydrophobic polymer and a continuous phase that contains a water-soluble polymer.

On the other hand, the outermost layer of the lithographic printing plate precursor of Comparative Example 1 or 2 was a layer in which the hydrophobic polymer and the water-soluble polymer were compatible with each other, and no sea-island structure was observed.

As is evident from the results shown in Tables 4 to 6, compared to the lithographic printing plate precursors according to comparative examples, the obtained lithographic printing plate precursors according to examples have higher receptivity and higher on-press development residue suppressiveness.

Furthermore, it has been revealed that the lithographic printing plate precursor according to the present disclosure makes it possible to obtain a lithographic printing plate excellent in printing durability and on-press developability.

### Explanation of References

12a, 12b: aluminum support
14: undercoat layer
16: image-recording layer
18: aluminum plate
20a, 20b: anodic oxide film
22a, 22b: micropore
24: large diameter portion
26: small diameter portion
D: depth of large diameter portion
610: anodization treatment device
612: power supply tank
614: electrolytic treatment tank
616: aluminum plate
618, 626: electrolytic solution
620: power supply electrode
62, 628: roller
624: nip roller
630: electrolysis electrode
632: cell wall
634: direct current power source

The entire disclosure of Japanese Patent Application No. 2020-130529, filed July 31, 2020, is incorporated into the present specification by reference.

All of documents, patent applications, and technical standards described in the present specification are incorporated into the present specification by reference to approximately the same extent as a case where it is specifically and respectively described that the respective documents, patent applications, and technical standards are incorporated by reference.

## Claims

1. An on-press development type lithographic printing plate precursor comprising, in the following order:
a support;
an image-recording layer; and
an outermost layer,
wherein the outermost layer has a sea-island structure consisting of a discontinuous phase that contains a hydrophobic polymer and a continuous phase that contains a water-soluble polymer.

2. The on-press development type lithographic printing plate precursor according to claim 1,
wherein a contact angle of water on a surface of the outermost layer that is measured 30 seconds after the water is landed as a droplet of water-in-oil is 60° to 160°.

3. The on-press development type lithographic printing plate precursor according to claim 1 or 2,
wherein a contact angle of water on a surface of the outermost layer that is measured 60 seconds after the water is landed as a droplet of water-in-oil is 60° to 160°.

4. The on-press development type lithographic printing plate precursor according to any one of claims 1 to 3,
wherein the hydrophobic polymer is particles.

5. The on-press development type lithographic printing plate precursor according to claim 4,
wherein the particles are crosslinked particles.

6. The on-press development type lithographic printing plate precursor according to claim 4 or 5,
wherein the particles have a dispersible group.

7. The on-press development type lithographic printing plate precursor according to claim 6,
wherein the dispersible group includes a group represented by Formula Z,
*-Q-W-Y Formula Z
in Formula Z, Q represents a divalent linking group, W represents a divalent group having a hydrophilic structure or a divalent group having a hydrophobic structure, Y represents a monovalent group having a hydrophilic structure, either W or Y has a hydrophilic structure, and * represents a bonding site with another structure.

8. The on-press development type lithographic printing plate precursor according to claim 6 or 7,
wherein the dispersible group has a polyalkylene oxide structure.

9. The on-press development type lithographic printing plate precursor according to any one of claims 1 to 8,
wherein the water-soluble polymer includes polyvinyl alcohol.

10. The on-press development type lithographic printing plate precursor according to claim 9,
wherein a saponification degree of the polyvinyl alcohol is 65% to 100%.

11. The on-press development type lithographic printing plate precursor according to any one of claims 1 to 10,
wherein the image-recording layer or the outermost layer contains a fluorohydrocarbon group-containing copolymer.

12. The on-press development type lithographic printing plate precursor according to claim 11,
wherein the fluorohydrocarbon group-containing copolymer includes constitutional units derived from monomers represented by Formula (F1) to Formula (F3),
in Formula (F1) to Formula (F3), R^{F1} each independently represent a hydrogen atom or a methyl group, L^{F} represents a single bond or a divalent linking group, Cf represents a linear or branched hydrocarbon group having 1 to 10 carbon atoms in which some or all of hydrogen atoms of the hydrocarbon group are substituted with fluorine atoms, X^{F} each independently represent an oxygen atom, a sulfur atom, or -N(R^{F3})-, R^{F2} represents a hydrogen atom or a fluorine atom, w1 to w3 each independently represent an integer of 0 to 9, w4 represents an integer of 1 to 10, w5 represents an integer of 0 to 2, and R^{F3} represents a hydrogen atom or an alkyl group having 1 to 4 carbon atoms.

13. The on-press development type lithographic printing plate precursor according to claim 12,
wherein the fluorohydrocarbon group-containing copolymer includes a constitutional unit derived from a monomer represented by Formula (F2) or Formula (F3).

14. The on-press development type lithographic printing plate precursor according to any one of claims 11 to 13,
wherein the fluorohydrocarbon group-containing copolymer includes a constitutional unit having a polyalkylene oxide structure.

15. The on-press development type lithographic printing plate precursor according to any one of claims 1 to 14,
wherein the outermost layer contains a preservative.

16. The on-press development type lithographic printing plate precursor according to any one of claims 1 to 15,
wherein the outermost layer contains a discoloring compound.

17. The on-press development type lithographic printing plate precursor according to claim 16,
wherein the discoloring compound includes a decomposable compound that decomposes due to exposure to infrared.

18. The on-press development type lithographic printing plate precursor according to any one of claims 1 to 17,
wherein the image-recording layer contains an infrared absorber, an electron-accepting polymerization initiator, an electron-donating polymerization initiator, and a polymerizable compound.

19. The on-press development type lithographic printing plate precursor according to claim 18,
wherein an energy level of HOMO of the infrared absorber - an energy level of HOMO of the electron-donating polymerization initiator is 0.70 eV or less.

20. The on-press development type lithographic printing plate precursor according to claim 18 or 19,
wherein an energy level of LUMO of the electron-accepting polymerization initiator - an energy level of LUMO of the infrared absorber is 1.00 eV or less.

21. The on-press development type lithographic printing plate precursor according to any one of claims 18 to 20,
wherein the electron-accepting polymerization initiator is an onium salt compound.

22. The on-press development type lithographic printing plate precursor according to any one of claims 18 to 20,
wherein the electron-accepting polymerization initiator includes a compound represented by Formula (II),
in Formula (II), X^{A} represents a halogen atom, and R^{A} represents an aryl group.

23. The on-press development type lithographic printing plate precursor according to any one of claims 18 to 22,
wherein the polymerizable compound includes a polymerizable compound having functionalities of 2 or less.

24. The on-press development type lithographic printing plate precursor according to any one of claims 18 to 23,
wherein the polymerizable compound includes a polymerizable compound having functionalities of 7 or more.

25. The on-press development type lithographic printing plate precursor according to any one of claims 1 to 24,
wherein the image-recording layer contains polyvinyl acetal.

26. The on-press development type lithographic printing plate precursor according to any one of claims 1 to 25,
wherein the support has an aluminum plate and an anodic oxide film of aluminum disposed on the aluminum plate,
the anodic oxide film is at a position closer to a side of the image-recording layer than the aluminum plate and has micropores extending in a depth direction from a surface of the anodic oxide film on the side of the image-recording layer, and
an average diameter of the micropores within the surface of the anodic oxide film is more than 10 nm and 100 nm or less.

27. The on-press development type lithographic printing plate precursor according to claim 26,
wherein the micropores are each composed of a large diameter portion that extends to a position at a depth of 10 nm to 1,000 nm from the surface of the anodic oxide film and a small diameter portion that is in communication with a bottom portion of the large diameter portion and extends to a position at a depth of 20 nm to 2,000 nm from a communicate position,
an average diameter of the large diameter portion within the surface of the anodic oxide film is 15 nm to 100 nm, and
an average diameter of the small diameter portion at the communicate position is 15 nm or less.

28. A method of preparing a lithographic printing plate, comprising:
a step of exposing the on-press development type lithographic printing plate precursor according to any one of claims 1 to 27 in a shape of an image; and
a step of supplying at least one of a printing ink or dampening water on a printer to remove the image-recording layer in a non-image area.

29. A lithographic printing method, comprising:
a step of exposing the on-press development type lithographic printing plate precursor according to any one of claims 1 to 27 in a shape of an image;
a step of supplying at least one of a printing ink or dampening water to remove the image-recording layer in a non-image area on a printer and to prepare a lithographic printing plate, and
a step of performing printing by using the obtained lithographic printing plate.
